



US005580690A

**United States Patent** [19]**Kato et al.**[11] **Patent Number:** **5,580,690**[45] **Date of Patent:** **Dec. 3, 1996**[54] **ELECTROPHOTOGRAPHIC  
LIGHT-SENSITIVE MATERIAL**[75] Inventors: **Eiichi Kato; Kazuo Ishii**, both of Shizuoka, Japan[73] Assignee: **Fuji Photo Film Co., Ltd.**, Kanagawa, Japan[21] Appl. No.: **357,150**[22] Filed: **Dec. 15, 1994****Related U.S. Application Data**

[63] Continuation of Ser. No. 70,540, Jun. 2, 1993, abandoned, which is a continuation-in-part of Ser. No. 39,138, Apr. 7, 1993, abandoned.

[30] **Foreign Application Priority Data**

|               |      |       |       |          |
|---------------|------|-------|-------|----------|
| Aug. 7, 1991  | [JP] | Japan | ..... | 3-221294 |
| Sep. 12, 1991 | [JP] | Japan | ..... | 3-260531 |
| Oct. 14, 1991 | [JP] | Japan | ..... | 3-291865 |
| Nov. 25, 1991 | [JP] | Japan | ..... | 3-334539 |
| Jul. 29, 1992 | [JP] | Japan | ..... | 4-220928 |
| Aug. 3, 1992  | [JP] | Japan | ..... | 4-224563 |

[51] **Int. Cl.<sup>6</sup>** ..... **G03G 5/05**[52] **U.S. Cl.** ..... **430/96**[58] **Field of Search** ..... **430/96, 95**[56] **References Cited**

## U.S. PATENT DOCUMENTS

|           |        |             |       |        |
|-----------|--------|-------------|-------|--------|
| 5,021,311 | 6/1991 | Kato et al. | ..... | 430/96 |
| 5,089,368 | 2/1992 | Kato et al. | ..... | 430/96 |

*Primary Examiner*—Christopher D. Rodee  
*Attorney, Agent, or Firm*—Sughrue, Mion, Zinn, Macpeak & Seas

[57]

**ABSTRACT**

An electrophotographic light-sensitive material which has improved electrostatic characteristics and image forming performance and is excellent particularly in reproducibility of highly accurate image using a liquid developer and image forming performance upon a scanning exposure system using a laser beam of a low power.

The electrophotographic light-sensitive material contains, as a binder resin, at least one resin selected from a low molecular weight resin (A<sub>1</sub>) formed from a macromonomer containing a polymer component of formula (I) and a monomer of the formula (I) and having a polar group bonded at one terminal of the main chain thereof, a low molecular weight resin (A<sub>2</sub>) formed from a macromonomer containing at random polar groups and a low molecular weight resin (A<sub>3</sub>) formed from a macromonomer containing polar groups as a block, and a resin (B) which is a medium to high molecular weight starlike polymer comprising an organic molecule having bonded thereto at least three polymer chains each containing a polymer component containing a specified polar group and a polymer component of formula (I).



wherein a<sup>1</sup> and a<sup>2</sup>: hydrogen, halogen, a cyano group, a hydrocarbon group, —COOR<sup>4</sup> or —COOR<sup>4</sup> bonded via a hydrocarbon group (R<sup>4</sup>: hydrocarbon group), and R<sup>3</sup>: a hydrocarbon group.

**7 Claims, No Drawings**

## ELECTROPHOTOGRAPHIC LIGHT-SENSITIVE MATERIAL

This is a continuation of application No. 08/070,540 filed Jun. 2, 1993, abandoned, which is a continuation-in-part of Application No. 08/039,138 filed Apr. 7, 1993, now abandoned.

### TECHNICAL FIELD

The present invention relates to an electrophotographic light-sensitive material, and more particularly to an electrophotographic light-sensitive material which is excellent in electrostatic characteristics and moisture resistance.

### TECHNICAL BACKGROUND

An electrophotographic light-sensitive material may have various structures depending upon the characteristics required or an electrophotographic process to be employed.

Typical electrophotographic light-sensitive materials widely employed comprise a support having provided thereon at least one photoconductive layer and, if necessary, an insulating layer on the surface thereof. The electrophotographic light-sensitive material comprising a support and at least one photoconductive layer formed thereon is used for the image formation by an ordinary electrophotographic process including electrostatic charging, imagewise exposure, development, and, if desired, transfer.

Furthermore, a process using an electrophotographic light-sensitive material as an offset master plate precursor for direct plate making is widely practiced. In particular, a direct electrophotographic lithographic plate has recently become important as a system for printing in the order of from several hundreds to several thousands prints having a high image quality.

Under these circumstances, binder resins which are used for forming the photoconductive layer of an electrophotographic light-sensitive material are required to be excellent in the film-forming properties by themselves and the capability of dispersing photoconductive powder therein. Also, the photoconductive layer formed using the binder resin is required to have satisfactory adhesion to a base material or support. Further, the photoconductive layer formed by using the binder resin is required to have various excellent electrostatic characteristics such as high charging capacity, small dark decay, large light decay, and less fatigue due to prior light-exposure and also have an excellent image forming properties, and the photoconductive layer stably maintains these electrostatic properties in spite of the fluctuation in humidity at the time of image formation.

Further, extensive studies have been made for lithographic printing plate precursors using an electrophotographic light-sensitive material, and for such a purpose, binder resins for a photoconductive layer which satisfy both the electrostatic characteristics as an electrophotographic light-sensitive material and printing properties as a printing plate precursor are required.

It has been found that the chemical structure of binder resin used in a photoconductive layer which contains at least an inorganic photoconductive substance, a spectral sensitizing dye and a binder resin has a great influence upon the electrostatic characteristics as well as smoothness of the photoconductive layer. Among the electrostatic characteristics, dark charge retention rate (D.R.R.) and photosensitivity are particularly affected.

Techniques for improvements in smoothness and electrostatic characteristics of a photoconductive layer by using a resin of a graft type copolymer having a low molecular weight and containing an acidic group at one terminal of the copolymer main chain or the graft portion thereof are described, for example, in U.S. Pat. No. 5,021,311, JP-A-2-247656 (the term "JP-A" as used herein means an "unexamined published Japanese Patent Application") and U.S. Pat. No. 5,089,368.

Further, techniques for improving a mechanical strength of a photoconductive layer by using the above described low molecular weight resin containing an acidic group together with a medium to high molecular weight resin are described, for example, in JP-A-2-96174, JP-A-2-127651, JP-A-2-135454, JP-A-2-134641, JP-A-2-272560, JP-A-2-304451, JP-A-2-308168, JP-A-3-42666, JP-A-3-77953, JP-A-3-77955, U.S. Patent 5,116,710 JP-A-3-223762, JP-A-3-238463, JP-A-3-238464, JP-A-3-261957, JP-A-3-259152, JP-A-4-15655, JP-A-4-20968, JP-A-4-25850, JP-A-4-29244, JP-A-4-30170, JP-A-4-37857, JP-A-4-39666, and JP-A-4-44047.

### PROBLEMS TO BE SOLVED BY THE INVENTION

However, it has been found that, even in a case of using these various low molecular weight resins having an acidic group or in a case of using these low molecular weight resins together with medium to high molecular weight resins, it is yet insufficient to keep the stable performance in the case of greatly fluctuating the ambient conditions from high-temperature and high-humidity to low-temperature and low-humidity. In particular, in a scanning exposure system using a semiconductor laser beam, the exposure time becomes longer and also there is a restriction on the exposure intensity as compared to a conventional overall simultaneous exposure system using a visible light, and hence a higher performance has been required for the electrostatic characteristics, in particular, the dark charge retention characteristics and photosensitivity.

Further, when the scanning exposure system using a semiconductor laser beam is applied to hitherto known light-sensitive materials for electrophotographic lithographic printing plate precursors, various problems may occur in that the difference between  $E_{1/2}$  and  $E_{1/10}$  is particularly large and the contrast of the duplicated image is decreased. Moreover, it is difficult to reduce the remaining potential after exposure, which results in severe fog formation in duplicated image, and when employed as lithographic printing plate precursors, edge marks of originals pasted up appear on the prints, in addition to the insufficient electrostatic characteristics described above.

Moreover, it has been desired to develop a technique which can faithfully reproduce highly accurate images of continuous gradation as well as images composed of lines and dots using a liquid developer. However, the above-described known techniques are still insufficient to fulfill such a requirement. Specifically, in the known technique, the improved electrostatic characteristics which are achieved by means of the low molecular weight resin may be sometimes deteriorated by using it together with the medium to high molecular weight resin. In fact, it has been found that an electrophotographic light-sensitive material having a photoconductive layer wherein the above described known resins are used in combination may cause a problem on reproducibility of the above described highly accurate image

(particularly, an image of continuous gradation) or on image forming performance in case of using a scanning exposure system with a laser beam of low power.

The present invention has been made for solving the problems of conventional electrophotographic light-sensitive materials as described above.

An object of the present invention is to provide an electrophotographic light-sensitive material having stable and excellent electrostatic characteristics and giving clear good images even when the ambient conditions during the formation of duplicated images are fluctuated to low-temperature and low-humidity or to high-temperature and high-humidity.

Another object of the present invention is to provide a CPC electrophotographic light-sensitive material having excellent electrostatic characteristics and showing less environmental dependency.

A further object of the present invention is to provide an electrophotographic light-sensitive material effective for a scanning exposure system using a semiconductor laser beam.

A still further object of the present invention is to provide an electrophotographic lithographic printing plate precursor having excellent electrostatic characteristics (in particular, dark charge retention characteristics and photosensitivity), capable of reproducing a faithfully duplicated image to the original (in particular, a highly accurate image of continuous gradation), forming neither overall background stains nor dotted background stains of prints, and showing excellent printing durability.

Other objects of the present invention will become apparent from the following description.

#### DISCLOSURE OF THE INVENTION

It has been found that the above described objects of the present invention are accomplished by an electrophotographic light-sensitive material having a photoconductive layer containing at least an inorganic photoconductive substance, a spectral sensitizing dye and a binder resin, wherein the binder resin comprises at least one resin selected from resin (A<sub>1</sub>), resin (A<sub>2</sub>) and resin (A<sub>3</sub>) shown below and at least one resin (B) shown below.

Resin (A<sub>1</sub>):

A copolymer having a weight average molecular weight of from  $1\times 10^3$  to  $2\times 10^4$  and being formed at least from a monofunctional macromonomer (M<sub>1</sub>) described below and a monomer corresponding to a repeating unit represented by the general formula (I) described below, wherein the copolymer has a polymer component containing at least one polar group selected from  $-\text{PO}_3\text{H}_2$ ,  $-\text{SO}_3\text{H}$ ,



(wherein R<sup>1</sup> represents a hydrocarbon group or  $-\text{OR}^2$  (wherein R<sup>2</sup> represents a hydrocarbon group)) and a cyclic acid anhydride group bonded at one terminal of the main chain thereof.

Monofunctional Macromonomer (M<sub>1</sub>):

A monofunctional macromonomer having a weight average molecular weight of not more than  $2\times 10^4$  and having a polymerizable double bond group bonded at only one terminal of the main chain of a polymer containing not less than 30% by weight of a polymer component corresponding to a repeating unit represented by the general formula (I) described below.



(wherein a<sup>1</sup> and a<sup>2</sup> each represents a hydrogen atom, a halogen atom, a cyano group, a hydrocarbon group,  $-\text{COOR}^4$  or  $-\text{COOR}^4$  bonded via a hydrocarbon group (wherein R<sup>4</sup> represents a hydrocarbon group); and R<sup>3</sup> represents a hydrocarbon group).

Resin (A<sub>2</sub>):

A copolymer having a weight average molecular weight of from  $1\times 10^3$  to  $2\times 10^4$  and being formed at least from a monofunctional macromonomer (M<sub>2</sub>) described below and a monomer corresponding to a repeating unit represented by the general formula (I) described above.

Monofunctional Macromonomer (M<sub>2</sub>):

A monofunctional macromonomer having a weight average molecular weight of not more than  $2\times 10^4$  and having a polymerizable double bond group at only one terminal of the main chain of a polymer containing at random not less than 30% by weight of a polymer component corresponding to a repeating unit represented by the general formula (I) described above and from 1 to 50% by weight of a polymer component containing at least one polar group selected from the specified polar groups as described in the resin (A<sub>1</sub>) above.

Resin (A<sub>3</sub>):

A copolymer having a weight average molecular weight of from  $1\times 10^3$  to  $2\times 10^4$  and being formed at least from a monofunctional macromonomer (M<sub>3</sub>) described below and a monomer corresponding to a repeating unit represented by the general formula (I) described above.

Monofunctional Macromonomer (M<sub>3</sub>):

A monofunctional macromonomer having a weight average molecular weight of not more than  $2\times 10^4$ , comprising an AB block copolymer composed of an A block containing a polymer component containing at least one polar group selected from the specified polar groups as described in the resin (A<sub>1</sub>) above and a B block containing a polymer component corresponding to a repeating unit represented by the general formula (II) described below and having a polymerizable double bond group bonded at the terminal of the main chain of the B block polymer.



wherein b<sup>1</sup> and b<sup>2</sup> each represents a hydrogen atom, a halogen atom, a cyano group, a hydrocarbon group,  $-\text{COOR}^4$  or  $-\text{COOR}^4$  bonded via a hydrocarbon group (wherein R<sup>4</sup> represents a hydrocarbon group); V<sup>1</sup> represents  $-\text{COO}-$ ,  $-\text{OCO}-$ ,  $-(\text{CH}_2)_a\text{OCO}-$ ,  $-(\text{CH}_2)_a\text{COO}-$  (wherein a represents an integer of from 1 to 3),  $-\text{O}-$ ,  $-\text{SO}_2-$ ,  $-\text{CO}-$ ,



(wherein  $Z^1$  represents a hydrogen atom or a hydrocarbon group),  $-CONHCOO-$ ,  $-CONHCONH-$  or



and  $R^5$  represents a hydrocarbon group, provided that when  $V^1$  represents



$R^5$  represents a hydrogen atom or a hydrocarbon group. Resin (B):

A starlike polymer having a weight average molecular weight of from  $3 \times 10^4$  to  $1 \times 10^6$  and comprising an organic molecule having bonded thereto at least three polymer chains each containing a polymer component containing at least one polar group selected from the specified polar groups as described in the resin ( $A_1$ ) above and a polymer component corresponding to a repeating unit represented by the general formula (I) as described in the resin ( $A_1$ ) above, wherein the polymer contains the polymer component containing a polar group in an amount of from 0.01 to 10% by weight and the polymer component corresponding to the general formula (I) in an amount not less than 30% by weight.

In short, the binder resin according to the present invention comprises at least one of the resin ( $A_1$ ) which is a copolymer formed at least from the macromonomer ( $M_1$ ) described above and the monomer corresponding to the general formula (I) described above and having the specified polar group bonded at one terminal of the main chain thereof, the resin ( $A_2$ ) which is a copolymer formed at least from the macromonomer ( $M_2$ ) described above containing at random the specified polar group-containing component and the monomer corresponding to the general formula (I) described above and the resin ( $A_3$ ) which is a copolymer formed at least from the macromonomer ( $M_3$ ) described above comprising an AB block copolymer being composed of an A block containing the specified polar group-containing component and a B block containing a polymer component corresponding to the general formula (II) described above and having a polymerizable double bond group bonded at one terminal of the B block polymer chain and the monomer corresponding to the general formula (I) described above (hereinafter, the macromonomers ( $M_1$ ), ( $M_2$ ) and ( $M_3$ ) are generically referred to as a macromonomer ( $M$ ), and the resins ( $A_1$ ), ( $A_2$ ) and ( $A_3$ ) are generically referred to as a resin (A), sometimes) and the resin (B) which is a starlike polymer comprising an organic molecule having bonded thereto at least three polymer chains each containing the specified polar group-containing polymer component described above and the polymer component corresponding to the general formula (I) described above.

As a result of various investigations, it has been found that, in the known technique wherein the low molecular weight resin containing a polar group is used together with the medium to high molecular weight resin, the improved electrostatic characteristics achieved by the low molecular weight resin are sometimes deteriorated by the medium to

high molecular weight resin used together as described above. Further, it has become apparent that an appropriate action of medium to high molecular weight resin on the interaction between the photoconductive substance, spectral sensitizing dye and low molecular weight resin in the photoconductive layer is an unexpectedly important factor.

It has been found that the above described objects can be effectively achieved by using the starlike polymer comprising an organic molecule having bonded thereto at least three polymer chains each containing the polar group-containing component and the component corresponding to the general formula (I) according to the present invention as a medium to high molecular weight resin to be used together with the low molecular weight resin (A) containing the polar group.

It is presumed that the electrostatic characteristics are stably maintained at a high level as a result of synergistic effect of the resin (A) and resin (B) according to the present invention wherein particles of photoconductive substance are sufficiently dispersed without the occurrence of aggregation, a spectral sensitizing dye and a chemical sensitizer are sufficiently adsorbed on the surface of particles of photoconductive substance, and the binder resin is sufficiently adsorbed to excessive active sites on the surface of the photoconductive substance to compensate the traps.

More specifically, the low molecular weight graft type copolymer resin (A) containing the specific polar group has an important function in that the resin is sufficiently adsorbed on the surface of particles of the photoconductive substance to disperse uniformly and to restrain the occurrence of aggregation due to its short polymer chain and in that adsorption of the spectral sensitizing dye on the photoconductive substance is not disturbed.

Further, by using the medium to high molecular weight starlike polymer comprising an organic molecule having at least three polymer chains each containing the specific components mechanical strength of the photoconductive layer is remarkably increased. This is believed to be based on that the polar group-containing component of the resin (B) has a weak interaction with the particles of photoconductive substance compared with the resin (A) and that the polymer chains of the resin (B) intertwine each other due to their starlike formation.

Moreover, according to the present invention the electrostatic characteristics are more improved in comparison with a case wherein a known medium to high molecular weight resin is employed. This is believed to be based on that the resin (B) acts to control the disturbance of adsorption of spectral sensitizing dye on the surface of particles of photoconductive substance due to the polar group present in the polar group-containing portion which interacts with the particles of photoconductive substance.

As a result, it is presumed that the resin (B) appropriately effects on controlling the disturbance of adsorption of spectral sensitizing dye on the surface of particles of photoconductive substance and the electrophotographic interactions and increasing the strength of the photoconductive layer in a system wherein the particles of photoconductive substance, spectral sensitizing dye and resin (A) are coexistent with the resin (B), while details thereof are not clear.

This effect is especially remarkable in a case wherein polymethine dyes or phthalocyanine series pigments which are particularly effective as spectral sensitizing dyes for the region of near infrared to infrared light are used.

When the electrophotographic light-sensitive material according to the present invention containing photoconductive zinc oxide as the photoconductive substance is applied to a conventional direct printing plate precursor, extremely good water retentivity as well as the excellent image forming performance can be obtained. More specifically, when

the light-sensitive material according to the present invention is subjected to an electrophotographic process to form an duplicated image, oil-desensitization of non-image portions by chemical treatment with a conventional oil-desensitizing solution to prepare a printing plate, and printing by an offset printing system, it exhibits excellent characteristics as a printing plate.

When the electrophotographic light-sensitive material according to the present invention is subjected to the oil-desensitizing treatment, the non-image portions are rendered sufficiently hydrophilic to increase water retention which results in remarkable increase in the number of prints obtained. It is believed that these results are obtained by the fact that the condition is formed under which a chemical reaction for rendering the surface of zinc oxide hydrophilic upon the oil-desensitizing treatment is able to proceed easily and effectively. Specifically, zinc oxide particles are uniformly and sufficiently dispersed in the resin (A) and resin (B) used as a binder resin and the state of binder resin present on or adjacent to the surface of zinc oxide particles is proper to conduct an oil-desensitizing reaction with the oil-desensitizing solution rapidly and effectively.

Now, the resin (A) which can be used as the binder resin for the photoconductive layer of the electrophotographic light-sensitive material according to the present invention will be described in more detail below.

The resin (A) according to the present invention is a graft type copolymer having a weight average molecular weight of from  $1\times 10^3$  to  $2\times 10^4$  and containing the polymer component represented by the general formula (I), and it includes three embodiments of the resins (A<sub>1</sub>), (A<sub>2</sub>) and (A<sub>3</sub>) mainly depending on a kind of macromonomer used for forming a copolymer component.

The resin (A<sub>1</sub>) is a graft type copolymer containing the polymer component represented by the general formula (I) in the graft portion and main chain portion thereof and having a polymer component containing the specified polar group bonded at one terminal of the main chain thereof.

The resin (A<sub>2</sub>) is a graft type copolymer containing the polymer component represented by the general formula (I) in the graft portion and main chain portion thereof and containing the specified polar group-containing component at random in the graft portion thereof.

The resin (A<sub>3</sub>) is a graft type copolymer containing the polymer component represented by the general formula (I) in the main chain thereof and containing the specified polar group-containing component as a block in the graft portion thereof.

The weight average molecular weight of the resin (A) is from  $1\times 10^3$  to  $2\times 10^4$ , and preferably from  $3\times 10^3$  to  $1\times 10^4$ . The glass transition point of the resin (A) is preferably from  $-30^\circ\text{C}$ . to  $110^\circ\text{C}$ . and more preferably from  $-20^\circ\text{C}$ . to  $90^\circ\text{C}$ .

If the weight average molecular weight of the resin (A) is less than  $1\times 10^3$  the film-forming property of the resin is lowered, thereby a sufficient film strength cannot be maintained, and on the other hand, if the weight average molecular weight of the resin (A) is higher than  $2\times 10^4$ , the effect of the present invention for obtaining stable duplicated images is reduced since fluctuations of electrophotographic characteristics (particularly, initial potential, dark charge retention rate and photosensitivity) of the photoconductive layer, in particular, that containing a spectral sensitizing dye for sensitization in the range of from near-infrared to infrared become somewhat large under severe conditions of high temperature and high humidity or low temperature and low humidity.

In the resin (A) according to the present invention, the total amount of polymer component containing the specified polar group present at the terminal of the main chain and the graft portion of the graft type copolymer is preferably from 0.5 to 20 parts by weight and more preferably from 1 to 15 parts by weight per 100 parts by weight of the resin (A).

If the content of the polar group-containing component in the resin (A) is less than 0.5% by weight, the initial potential is low and thus satisfactory image density is hardly obtained. On the other hand, if the content of the polar group-containing component is larger than 20% by weight, various undesirable problems may occur, for example, the dispersibility of photoconductive substance is reduced, and further when the light-sensitive material is used as an offset master plate, the occurrence of background stains may increase even a low molecular weight resin.

The weight average molecular weight of the macromonomer (M) used in the resin (A) is not more than  $2\times 10^4$ . If the weight average molecular weight of the macromonomer (M) exceeds  $2\times 10^4$ , copolymerizability with other monomers, for example, those corresponding to the general formula (I) described in detail hereinafter is undesirably reduced. If, on the other hand, it is too small, the effect of improving electrophotographic characteristics of the light-sensitive layer would be small. Accordingly, the macromonomer (M) preferably has a weight average molecular weight of at least  $1\times 10^3$ .

The content of the macromonomer (M) in the resin (A) is suitably from 1 to 70% by weight, and preferably from 5 to 50% by weight.

If the content of the macromonomer is less than 1% by weight in the resin (A), electrophotographic characteristics (particularly, dark charge retention rate and photosensitivity) may be reduced and the fluctuations of electrophotographic characteristics of the photoconductive layer, particularly that containing a spectral sensitizing dye for the sensitization in the range of from near-infrared to infrared become large depending on changes in ambient conditions. The reason therefor is considered that the construction of the polymer becomes similar to that of a conventional homopolymer or random polymer due to the presence of only a small amount of macromonomer which constitutes the graft portion. On the other hand, if the content of the macromonomer in the resin (A) exceeds 70% by weight, the copolymerizability of the macromonomer with other monomers corresponding to other copolymer components according to the present invention may become insufficient, and there is a tendency that the sufficient electrophotographic characteristics can not be obtained as the binder resin.

The content of the polymer component corresponding to the repeating unit represented by the general formula (I) copolymerizable with the macromonomer present in the resin (A) is suitably not less than 30% by weight, and preferably not less than 50% by weight.

The repeating unit represented by the general formula (I) above which is contained in the resin (A) will be described in greater detail below.

In the general formula (I), a<sup>1</sup> and a<sup>2</sup> each preferably represents a hydrogen atom, a halogen atom (e.g., chlorine and bromine), a cyano group, an alkyl group having from 1 to 4 carbon atoms (e.g., methyl, ethyl, propyl and butyl), —COOR<sup>4</sup> or —COOR<sup>4</sup> bonded via a hydrocarbon group (wherein R<sup>4</sup> represents a hydrogen atom or an alkyl, alkenyl, aralkyl, alicyclic or aryl group which may be substituted, and specifically includes those as described for R<sup>3</sup> hereinafter). Particularly preferably a<sup>1</sup> represents a hydrogen atom and a<sup>2</sup> represents a methyl group.

The hydrocarbon group in the above described  $-\text{COOR}^4$  group bonded via a hydrocarbon group includes, for example, a methylene group, an ethylene group and a propylene group.

$R^3$  preferably represents a hydrocarbon group having not more than 18 carbon atoms, which may be substituted. The substituent for the hydrocarbon group may be any substituent other than the polar groups contained in the polar group-containing polymer component described above present in the resin (A). Suitable examples of the substituent include a halogen atom (e.g., fluorine, chlorine and bromine),  $-\text{OR}^6$ ,  $-\text{COOR}^6$ , and  $-\text{OCOR}^6$  (wherein  $R^6$  represents an alkyl group having from 1 to 22 carbon atoms, e.g., methyl, ethyl, propyl, butyl, hexyl, octyl, decyl, dodecyl, hexadecyl and octadecyl). Preferred examples of the hydrocarbon group include an alkyl group having from 1 to 18 carbon atoms which may be substituted (e.g., methyl, ethyl, propyl, butyl, pentyl, hexyl, heptyl, octyl, decyl, dodecyl, hexadecyl, octadecyl, 2-chloroethyl, 2-bromoethyl, 2-cyanoethyl, 2-hydroxyethyl, 2-methoxycarbonyethyl, 2-methoxyethyl, 2-ethoxyethyl, 3-hydroxypropyl and 3-bromopropyl), an alkenyl group having from 2 to 18 carbon atoms which may be substituted (e.g., vinyl, allyl, 2-methyl-1-propenyl, 2-butenyl, 2-pentenyl, 3-methyl-2-pentenyl, 1-pentenyl, 1-hexenyl, 2-hexenyl and 4-methyl-2-hexenyl), an aralkyl group having from 7 to 12 carbon atoms which may be substituted (e.g., benzyl, phenethyl, 3-phenylpropyl, naphthylmethyl, 2-naphthylethyl, chlorobenzyl, bromobenzyl, methylbenzyl, ethylbenzyl, methoxybenzyl, dimethylbenzyl and dimethoxybenzyl), an alicyclic group having from 5 to 8 carbon atoms which may be substituted (e.g., cyclopentyl, cyclohexyl, 2-cyclohexylethyl and 2-cyclopentylethyl), and an aromatic group having from 6 to 12 carbon atoms which may be substituted (e.g., phenyl, naphthyl, tolyl, xylyl, propylphenyl, butylphenyl, octylphenyl, dodecylphenyl, methoxyphenyl, ethoxyphenyl, butoxyphenyl, decyloxyphenyl, chlorophenyl, dichlorophenyl, bromophenyl, cyanophenyl, acetylphenyl, methoxycarbonylphenyl, ethoxycarbonylphenyl, butoxycarbonylphenyl, acetamidophenyl, propioamidophenyl and dodecyloylamidophenyl).

More preferably, the polymer component corresponding to the repeating unit represented by the general formula (I) is a methacrylate component having the specific aryl group represented by the general formula (Ia) and/or (Ib) described below. The low molecular weight resin containing the specific aryl group-containing methacrylate polymer component described above is sometimes referred to as a resin (A') hereinafter.



Formula (Ia) 50



Formula (Ib)

wherein  $T_1$  and  $T_2$  each represents a hydrogen atom, a halogen atom, a hydrocarbon group having from 1 to 10 carbon atoms,  $-\text{COR}_a$  or  $-\text{COOR}_a$ , wherein  $R_a$  represents a hydrocarbon group having from 1 to 10 carbon atoms; and  $L_1$  and  $L_2$  each represents a mere bond or a linking group

containing from 1 to 4 linking atoms, which connects  $-\text{COO--}$  and the benzene ring.

In the resin (A'), the content of the methacrylate polymer component corresponding to the repeating unit represented by the general formula (Ia) and/or (Ib) is suitably not less than 30% by weight, preferably from 50 to 97% by weight, and the content of polymer component containing the specified polar group is suitably from 0.5 to 20% by weight, preferably from 1 to 15% by weight.

In case of using the resin (A'), the electrophotographic characteristics (particularly,  $V_{10}$ , D.R.R. and  $E_{1/10}$ ) of the electrophotographic material can be furthermore improved.

In the general formula (Ia),  $T_1$  and  $T_2$  each preferably represents a hydrogen atom, a chlorine atom, a bromine atom, an alkyl group having from 1 to 4 carbon atoms (e.g., methyl, ethyl, propyl and butyl), an aralkyl group having from 7 to 9 carbon atoms (e.g., benzyl, phenethyl, 3-phenylpropyl, chlorobenzyl, dichlorobenzyl, bromobenzyl, methylbenzyl, methoxybenzyl and chloromethylbenzyl), an aryl group (e.g., phenyl, tolyl, xylyl, bromophenyl, methoxyphenyl, chlorophenyl and dichlorophenyl),  $-\text{COR}_a$  or  $-\text{COOR}_a$  (wherein  $R_a$  preferably represents any of the above-recited preferred hydrocarbon groups having from 1 to 10 carbon atoms).

In the general formulae (Ia) and (Ib),  $L_1$  and  $L_2$  each represents a mere bond or a linking group containing from 1 to 4 linking atoms which connects between  $-\text{COO--}$  and the benzene ring, e.g.,  $-\text{CH}_2\text{--O--}_n$  (wherein  $n$  represents an integer of 1 to 3),  $-\text{CH}_2\text{O--CO--}$ ,  $-\text{CH}_2\text{CH}_2\text{O--CO--}$ ,  $-\text{CH}_2\text{O--}_m$  (wherein  $m$  represents an integer of 1 or 2) and  $-\text{CH}_2\text{CH}_2\text{O--}$ , and preferably represents a mere bond or a linking group containing from 1 to 2 linking atoms.

Specific examples of the polymer component corresponding to the repeating unit represented by the general formula (Ia) or (Ib) which can be used in the resin (A) according to the present invention are set forth below, but the present invention should not be construed as being limited thereto. In the following formulae (a-1) to (a-17),  $n$  represents an integer of from 1 to 4;  $m$  represents an integer of from 0 to 3;  $p$  represents an integer of from 1 to 3;  $R_{10}$  to  $R_{13}$  each represents  $-\text{C}_n\text{H}_{2n+1}$  or  $-(\text{CH}_2)_m\text{C}_6\text{H}_5$  (wherein  $n$  and  $m$  each has the same meaning as defined above); and  $X_1$  and  $X_2$ , which may be the same or different, each represents a hydrogen atom,  $-\text{Cl}$ ,  $-\text{Br}$  or  $-\text{I}$ .



**11**  
-continued

(a-4)

5

(a-5) 10

15

(a-6)

20

(a-7)

30

(a-8)

35

(a-9)

45

(a-10)

(a-11)

55

60

**12**  
-continued

(a-12)

(a-13)

(a-14)

(a-15)

(a-16)

(a-17)

In the graft type copolymer according to the present invention, one or more other monomers may be employed as a component copolymerizable with the macromonomer (M) in addition to a monomer corresponding to the repeating unit of the general formula (I), (Ia) or (Ib). Examples of such monomers include, in addition to methacrylic acid esters, acrylic acid esters and crotonic acid esters containing substituents other than those described for the general formula (I),  $\alpha$ -olefins, vinyl or allyl esters of carboxylic acids (including, e.g., acetic acid, propionic acid, butyric acid, valeric acid, benzoic acid and naphthalenecarboxylic acid, as examples of the carboxylic acids), acrylonitrile, methacrylonitrile, vinyl ethers, itaconate acid esters (e.g., dimethyl itaconate and diethyl itaconate), acrylamides, methacrylamides, styrenes (e.g., styrene, vinyltoluene,

chlorostyrene, hydroxystyrene, N,N-dimethylaminomethylstyrene, methoxycarbonylstyrene, methanesulfonyloxystyrene and vinylnaphthalene), vinylsulfone-containing compounds, vinylketone-containing compounds and heterocyclic vinyl compounds (e.g., vinylpyrrolidone, vinylpyridine, vinylimidazole, vinylthiophene, vinylimidazole, vinylpyrazoles, vinyldioxane, vinylquinoline, vinyltetrazole and vinyloxazine). Preferred examples thereof include vinyl or allyl esters of alcanoic acids containing from 1 to 3 carbon atoms, acrylonitrile, methacrylonitrile, styrene and styrene derivatives (e.g., vinyltoluene, butylstyrene, methoxystyrene, chlorostyrene, dichlorostyrene, bromostyrene and ethoxystyrene). It is preferred that the content of the polymer components corresponding to such other monomers does not exceed 20% by weight of the resin (A).

Now, the polymer component having the specified polar group present in the resin (A) will be described in detail below.

The polymer component having the specified polar group includes that is present in the graft portion of the resin (A) and that is present at one terminal of the copolymer main chain.

The polar group included in the polar group-containing polymer component is selected from  $-\text{PO}_3\text{H}_2$ ,  $-\text{SO}_3\text{H}$ ,  $-\text{COOH}$ ,



and a cyclic acid anhydride group, as described above.

In the group



above,  $\text{R}^1$  represents a hydrocarbon group or  $-\text{OR}^2$  (wherein  $\text{R}^2$  represents a hydrocarbon group). The hydrocarbon group represented by  $\text{R}^1$  or  $\text{R}^2$  preferably includes an aliphatic group having from 1 to 22 carbon atoms which may be substituted (e.g., methyl, ethyl, propyl, butyl, hexyl, octyl, decyl, dodecyl, octadecyl, 2-chloroethyl, 2-methoxyethyl, 3-ethoxypropyl, allyl, crotonyl, butenyl, cyclohexyl, benzyl, phenethyl, 3-phenylpropyl, methylbenzyl, chlorobenzyl, fluorobenzyl and methoxybenzyl) and an aryl group which may be substituted (e.g., phenyl, tolyl, ethylphenyl, propylphenyl, chlorophenyl, fluorophenyl, bromophenyl, chloromethylphenyl, dichlorophenyl, methoxyphenyl, cyanophenyl, acetamidophenyl, acetylphenyl and butoxyphenyl).

The cyclic acid anhydride group is a group containing at least one cyclic acid anhydride. The cyclic acid anhydride to be contained includes an aliphatic dicarboxylic acid anhydride and an aromatic dicarboxylic acid anhydride.

Specific examples of the aliphatic dicarboxylic acid anhydrides include succinic anhydride ring, glutaconic anhydride ring, maleic anhydride ring, cyclopentane-1,2-dicarboxylic acid anhydride ring, cyclohexane-1,2-dicarboxylic acid anhydride ring, cyclohexene-1,2-dicarboxylic acid anhydride ring, and 2,3-bicyclo[2.2.2]octanedicarboxylic acid anhydride. These rings may be substituted with, for example, a halogen atom such as a chlorine atom and a bromine atom and an alkyl group such as a methyl group, an ethyl group, a butyl group and a hexyl group.

Specific examples of the aromatic dicarboxylic acid anhydrides include phthalic anhydride ring, naphthalenedicarboxylic acid anhydride ring, pyridinedicarboxylic acid anhydride ring and thiophenedicarboxylic acid anhydride ring. These rings may be substituted with, for example, a halogen atom (e.g., chlorine and bromine), an alkyl group (e.g., methyl, ethyl, propyl and butyl), a hydroxyl group, a cyano group, a nitro group and an alkoxy carbonyl group (e.g., a methoxy group and an ethoxy group as an alkoxy group).

In a case wherein the polar group is present in the polymer chain of the macromonomer as in the resins (A<sub>2</sub>) and (A<sub>3</sub>), the polar group may be bonded to the polymer chain either directly or via an appropriate linking group.

The linking group can be any group for connecting the polar group to the polymer chain. Specific examples of suitable linking group include



(wherein  $\text{d}_1$  and  $\text{d}_2$ , which may be the same or different, each represents a hydrogen atom, a halogen atom (e.g., chlorine and bromine), a hydroxyl group, a cyano group, an alkyl group (e.g., methyl, ethyl, 2-chloroethyl, 2-hydroxyethyl, propyl, butyl and hexyl), an aralkyl group (e.g., benzyl and phenethyl) or a phenyl group),



(wherein  $\text{d}_3$  and  $\text{d}_4$  each has the same meaning as defined for  $\text{d}_1$  or  $\text{d}_2$  above),  $-\text{C}_6\text{H}_{10}$ ,  $-\text{C}_6\text{H}_4-$ ,  $-\text{O}-$ ,  $-\text{S}-$ ,



(wherein  $\text{d}_5$  represents a hydrogen atom or a hydrocarbon group (preferably having from 1 to 12 carbon atoms (e.g., methyl, ethyl, propyl, butyl hexyl, octyl, decyl, dodecyl, 2-methoxyethyl, 2-chloroethyl, 2-cyanoethyl, benzyl, methylbenzyl, phenethyl, phenyl, tolyl, chlorophenyl, methoxyphenyl and butylphenyl)),  $-\text{CO}-$ ,  $-\text{COO}-$ ,  $-\text{OCO}-$ ,  $\text{CON}(\text{d}_5)-$ ,  $-\text{SO}_2\text{N}(\text{d}_5)-$ ,  $-\text{SO}_2-$ ,  $-\text{NHCONH}-$ ,  $-\text{NHCOO}-$ ,  $-\text{NHSO}_2-$ ,  $-\text{CONHCOO}-$ ,  $-\text{CONHCONH}-$ , a heterocyclic ring (preferably a 5-membered or 6-membered ring containing at least one of O, S and N as a hereto atom or a condensed ring thereof (e.g., thiophene, pyridine, furan, imidazole, piperidine and morpholine rings)),



(wherein  $\text{d}_6$  and  $\text{d}_7$ , which may be the same or different, each represents a hydrocarbon group or  $-\text{Od}_8$  (wherein  $\text{d}_8$  represents a hydrocarbon group)), and a combination thereof. Suitable examples of these hydrocarbon groups include those described for  $\text{d}_5$ .

The polymer component containing the polar group according to the present invention may be any of specified polar group-containing vinyl compounds copolymerizable with, for example, a monomer corresponding to the repeating unit represented by the general formula (I) (including

that represented by the general formula (Ia) or (Ib)). Examples of such vinyl compounds are described, e.g., in Kobunshi Gakkai (ed.), *Kobunshi Data Handbook Kisohen (Polymer Data Handbook Basis)*, Baifukan (1986). Specific examples of these vinyl monomers include acrylic acid,  $\alpha$ - and/or  $\beta$ -substituted acrylic acids (e.g.,  $\alpha$ -acetoxy,  $\alpha$ -acetoxyethyl,  $\alpha$ -(2-amino)ethyl,  $\alpha$ -chloro,  $\alpha$ -bromo,  $\alpha$ -fluoro,  $\alpha$ -tributylsilyl,  $\alpha$ -cyano,  $\beta$ -chloro,  $\beta$ -bromo,  $\alpha$ -chloro- $\beta$ -methoxy and  $\alpha$ , $\beta$ -dichloro compounds), methacrylic acid, itaconic acid, itaconic half esters, itaconic half amides, crotonic acid, 2-alkenylcarboxylic acids (e.g., 2-pentenoic acid, 2-methyl-2-hexenoic acid, 2-octenoic acid, 4-methyl-2-hexenoic acid and 4-ethyl-2-octenoic acid), maleic acid, maleic half esters, maleic half amides, vinylbenzenecarboxylic acid, vinylbenzenesulfonic acid, vinylsulfonic acid, vinylphosphonic acid, dicarboxylic acid vinyl or allyl half esters, and ester or amide derivatives of these carboxylic acids or sulfonic acids containing the specified polar group in the substituent thereof.

Specific examples of the polar group-containing polymer components are set forth below. In the following formulae,  $e_1$  represents  $-\text{H}$  or  $-\text{CH}_3$ ;  $e_2$  represents  $-\text{H}$ ,  $-\text{CH}_3$  or  $-\text{CH}_2\text{COOCH}_3$ ;  $R_{14}$  represents an alkyl group having from 1 to 4 carbon atoms;  $R_{15}$  represents an alkyl group having from 1 to 6 carbon atoms, a benzyl group or a phenyl group;  $c$  represents an integer of from 1 to 3;  $d$  represents an integer of from 2 to 11;  $e$  represents an integer of from 1 to 11;  $f$  represents an integer of from 2 to 4; and  $g$  represents an integer of from 2 to 10.



**17**  
-continued**18**  
-continued



In the resin ( $A_2$ ) according to the present invention, the polymer components containing the polar group described above are present irregularly in the macromonomer ( $M_2$ ), and the content thereof is preferably from 1 to 50% by weight and more preferably from 3 to 30% by weight based on the macromonomer ( $M_2$ ).

(b-44) 20 Of the resins ( $A_2$ ), those additionally having at least one polar group selected from the above described polar groups bonded at one terminal of the copolymer main chain thereof (hereinafter, these resins are particularly referred to as resin ( $A_{12}$ ) sometimes) are preferred.

(b-45) 25 In the resin (A<sub>12</sub>), the polar group contained in the polymer component of the macromonomer and the polar group bonded at one terminal of the copolymer main chain may be the same or different, and the ratio of the polar group present in the polymer chain of the macromonomer to the polar group bonded to the terminal of the polymer main chain may be varied depending on the kinds and amounts of other binder resins, a spectral sensitizing dye, a chemical sensitizer and other additives which constitute the photo-conductive layer according to the present invention, and can be appropriately controlled. What is important is that the total amount of the polar group-containing component present in the resin (A<sub>12</sub>) is from 0.5 to 20% by weight.

(b-46) 30

In a case wherein the polar group is present at one terminal of the copolymer main chain as in the resins (A<sub>1</sub>) and (A<sub>12</sub>), the polar group may be bonded to the terminal of the copolymer main chain either directly or via an appropriate linking group. Suitable examples of the linking groups include those illustrated for the cases wherein the polar groups are present in the polymer chain hereinbefore described.

In the resins (A<sub>1</sub>) and (A<sub>2</sub>) (including the resin (A<sub>12</sub>)), the polymer component which constitutes a repeating unit of the monofunctional macromonomer (M<sub>1</sub>) or (M<sub>2</sub>) having a polymerizable double bond group bonded at one terminal of the polymer chain thereof includes the component represented by the general formula (I), (Ia) and/or (Ib), and the content thereof is not less than 30% by weight, preferably not less than 50% by weight in the macromonomer.

(b-49) The component of the general formula (I) used as the copolymer component and the component of the general formula (I) included as the polymer component in the macromonomer ( $M_1$ ) or ( $M_2$ ) may be the same or different in the resin ( $A_1$ ) or ( $A_2$ ). The macromonomers ( $M_1$ ) and ( $M_2$ ) may further contain a polymer component other than the polymer components represented by the general formula (I), (Ia) and (Ib) and the polymer component containing the specified polar group which may be used if desired. Such other polymer components include those described as the other components which are copolymerizable with the macromonomer (M) and the component of the general formula (I) for forming the copolymer main chain of the resin (A) described above.

55

60

(b-50)

65

In the resin ( $A_3$ ) containing an AB block copolymer in the graft portion, the polar group-containing component

described above is present in the A block. Two or more kinds of the polar group-containing components may be present in the A block, and in such a case, two or more kinds of these polar group-containing components may be contained in the form of a random copolymer or a block copolymer in the block A. The A block may further contain a component which does not contain the polar group (for example, a component represented by the general formula (II) described in detail below) in addition to the polar group-containing component. The content of the polar group-containing component in the A block is preferably from 30 to 100% by weight.

Now, the repeating unit represented by the general formula (II) which is a component constituting the B block in the resin (A<sub>3</sub>) will be described in detail below.

In the general formula (II), V<sup>1</sup> represents —COO—, —OCO—, —(CH<sub>2</sub>)<sub>a</sub>OCO—, —(CH<sub>2</sub>)<sub>a</sub>COO— (wherein a represents an integer of from 1 to 3), —O—, —SO<sub>2</sub>—, —CO—,



—CONHCOO—, —CONHCONH— or



(wherein Z<sup>1</sup> represents a hydrogen atom or a hydrocarbon group).

Preferred examples of the hydrocarbon group represented by Z<sup>1</sup> include an alkyl group having from 1 to 22 carbon atoms which may be substituted (e.g., methyl, ethyl, propyl, butyl, hexyl, heptyl octyl, decyl, dodecyl, hexadecyl, octadecyl, 2-chloroethyl, 2-bromoethyl, 2-cyanoethyl, 2-methoxycarbonylethyl, 2-methoxyethyl and 3-bromopropyl), an alkenyl group having from 4 to 18 carbon atoms which may be substituted (e.g., 2-methyl-1-propenyl, 2-butenyl, 2-pentenyl, 3-methyl-2-pentenyl, 1-pentenyl, 1-hexenyl, 2-hexenyl and 4-methyl-2-hexenyl), an aralkyl group having from 7 to 12 carbon atoms which may be substituted (e.g., benzyl, phenethyl, 3-phenylpropyl, naphthylmethyl, 2-naphthylethyl, chlorobenzyl, bromobenzyl, methylbenzyl, ethylbenzyl, methoxybenzyl, dimethylbenzyl and dimethoxybenzyl), an alicyclic group having from 5 to 8 carbon atoms which may be substituted (e.g., cyclohexyl, 2-cyclohexylethyl and 2-cyclopentylethyl) and an aromatic group having from 6 to 12 carbon atoms which may be substituted (e.g., phenyl, naphthyl, tolyl, xylyl, propylphenyl, butylphenyl, octylphenyl, dodecylphenyl, methoxyphenyl, ethoxyphenyl, butoxyphenyl, decyloxyphenyl, chlorophenyl, dichlorophenyl, bromophenyl, cyanophenyl, acetylphenyl, methoxycarbonylphenyl, ethoxycarbonylphenyl, butoxycarbonylphenyl, acetamidophenyl, propioamidophenyl and dodecyloylaminophenyl).

In the general formula (II), R<sup>5</sup> represents a hydrocarbon group, and preferred examples thereof include those described for Z<sup>1</sup> above.

When V<sup>1</sup> represents



R<sup>5</sup> represents a hydrogen atom or a hydrocarbon group, and the benzene ring thereof may further be substituted. Suitable

examples of the substituents include a halogen atom (e.g., chlorine and bromine), an alkyl group (e.g., methyl, ethyl, propyl, butyl, chloromethyl and methoxymethyl) and an alkoxy group (e.g., methoxy, ethoxy, propoxy and butoxy).

In the general formula (II), b<sup>1</sup> and b<sup>2</sup>, which may be the same or different, each has the same meaning as defined for a<sup>1</sup> or a<sup>2</sup> in the general formula (I) described above.

More preferably, in the general formula (II), V<sup>1</sup> represents —COO—, —OCO—, —CH<sub>2</sub>OCO—, —CH<sub>2</sub>COO—, —O—, —CONH—, —SO<sub>2</sub>NH— or



and b<sup>1</sup> and b<sup>2</sup>, which may be the same or different, each represents a hydrogen atom, a methyl group, —COOZ<sup>3</sup>, or —CH<sub>2</sub>COOZ<sup>3</sup>, wherein Z<sup>3</sup> represents an alkyl group having from 1 to 6 carbon atoms (e.g., methyl, ethyl, propyl, butyl and hexyl). Most preferably, either one of b<sup>1</sup> and b<sup>2</sup> represents a hydrogen atom.

The content of the polymer component corresponding to the general formula (II) above present in the B block of the macromonomer (M<sub>3</sub>) in the resin (A<sub>3</sub>) is preferably not less than 30% by weight, more preferably not less than 50% by weight of the B block.

The B block may further contain a polymer component other than the polymer component represented by the general formula (II). Such other polymer components include those described as the other components which are copolymerizable with the macromonomer and the component of the general formula (I) for forming the copolymer main chain of the resin (A). Such other components, however, are employed in a range of not more than 20 parts by weight per 100 parts by weight of the total polymer components constituting the B block. Further, the B block preferably does not contain any specified polar group-containing polymer component which is a component constituting the A block. When two or more kinds of polymer components are present in the B block, two or more kinds of these polymer components may be contained in the B block in the form of a random copolymer or a block copolymer. However, it is preferred that they are present at random in view of simplicity in synthesis.

The copolymer component constituting the macromonomer (M<sub>3</sub>) used in the resin (A<sub>3</sub>) comprises the A block and the B block as described above, and a ratio of A block/B block is preferably 1 to 70/99 to 30 by weight and more preferably 3 to 50/97 to 50 by weight.

Now, the polymerizable double bond group bonded at one terminal of the macromonomer (M) constituting the resin (A) which is the graft type copolymer according to the present invention will be described in detail below.

In a case of the macromonomer (M<sub>3</sub>) constituting the resin (A<sub>3</sub>), the polymerizable double bond group is bonded at one terminal of the B block the other terminal of which is bonded to the A block as described above.

Suitable examples of the polymerizable double bond group include those represented by the following general formula (III):



Formula (III)

wherein V<sup>2</sup> has the same meaning as V<sup>1</sup> defined in the general formula (II), and c<sup>1</sup> and c<sup>2</sup>, which may be the same

or different, each has the same meaning as a<sup>1</sup> or a<sup>2</sup> defined in the general formula (I).

Specific examples of the polymerizable double bond group represented by the general formula (III) include



The polymerizable double bond group may be bonded to one terminal of the polymer chain which constitutes a graft portion either directly or via an appropriate linking group. Suitable examples of the linking groups include those illustrated for the cases wherein the polar groups are present in the polymer chain hereinbefore described.

The macromonomer (M) constituting the resin (A) used in the present invention can be produced by conventionally known synthesis methods.

- 10 Specifically, the macromonomers (M<sub>1</sub>) and (M<sub>2</sub>) contained in the resins (A<sub>1</sub>) and (A<sub>2</sub>) can be synthesized by a radical polymerization method of forming the macromonomer by reacting an oligomer having a reactive group bonded at the terminal thereof and various reagents. The oligomer used above can be obtained by a radical polymerization using a polymerization initiator and/or a chain transfer agent each having the reactive group such as a carboxy group, a carboxyhalide group, a hydroxy group, an amino group, a halogen atom, an epoxy group, etc., in the molecule thereof.
- 15 More specifically, they can be synthesized according to the methods as described, for example, in P. Dreyfuss & R. P. Quirk, *Encycl. Polym. Sci. Eng.*, 7, 551 (1987), P. F. Rempp & E. Franta, *Adv. Polym. Sci.*, 58, 1 (1984), Yusuke Kawakami, *Kagaku Kogyo (Chemical Industry)*, 38, 56 (1987), Yuuya Yamashita, *Kobunshi (Polymer)*, 31, 988 (1982), Shiro Kobayashi, *Kobunshi (Polymer)*, 30, Koichi Ito, *Kobunshi Kako (Polymer Processing)*, 35, 262 (1986), Kishiro Higashi & Takashi Tsuda, *Kino Zairyo (Functional Materials)*, 1987, No. 10, 5, and the literature references and patents cited therein.

20 However, since the macromonomer (M<sub>2</sub>) used in the present invention has the above-described polar group as the component of the repeating unit, the following matters should be considered in the synthesis thereof.

- 25 In one method, the radical polymerization and the introduction of a terminal reactive group are carried out by the above-described method using a monomer having the polar group as the form of a protected functional group as shown, for example, in the following reaction formula (A).



-continued  
Reaction Formula (A)

\* [Pre] : protective group for  $-\text{COOH}$ , e.g.,  $-\text{C}(\text{C}_6\text{H}_5)_3$ ,



The reaction for introducing the protective group and the reaction for removal of the protective group (e.g., hydrolysis reaction, hydrogenolysis reaction and oxidative decomposition reaction) for the polar group being randomly contained in the macromonomer ( $M_2$ ) used in the present invention can be carried out by any of conventional known methods.

These methods are specifically described, for example, in J. F. W. McOmie, *Protective Groups in Organic Chemistry*, Plenum Press (1973), T. W. Greene, *Protective Groups in Organic Synthesis*, John Wiley & Sons (1981), Ryohei Oda, *Kobunshi Fine Chemical (Polymer Fine Chemical)*, Kodansha K. K., (1976), Yoshio Iwakura and Keisuke Kurita, *Hannosei Kobunshi (Reactive Polymers)*, Kodansha K. K. (1977), G. Berner, et al, *J. Radiation Curing*, No. 10, 10(1986), JP-A-62-212669, JP-A-62-286064, JP-A-62-210475, JP-A-62-195684, JP-A-62-258476, JP-A-63-260439, Japanese Patent Application Nos. 62-220520 and 62-226692.

Another method for producing the macromonomer ( $M_2$ ) comprises synthesizing the oligomer in the same manner as described above and then reacting the oligomer with a reagent having a polymerizable double bond group which reacts with only the specific reactive group bonded at one terminal by utilizing the difference between the reactivity of the specific reactive group and the reactivity of the polar group contained in the oligomer as shown in the following reaction formula (B).

10      the present invention should not be construed as being limited thereto. It is important to utilize the selectivity of reaction in an ordinary organic chemical reaction and the macromonomer may be formed without protecting the polar group present in the oligomer. In Table 1, Moiety A is a functional group in the reagent for introducing a polymerizable group, Moiety B is a specific functional group bonded at the terminal of oligomer, and Moiety C is a polar group present in the repeating unit in the oligomer.

15

20

25

30

Reaction Formula (B)



60  
 Specific examples of combination of the specific functional groups (moieties A, B, and C) as described in the reaction formula (B) are shown in Table 1 below, although

TABLE 1

| Moiety A                                                                                  | Moiety B                   | Moiety C                                                         |
|-------------------------------------------------------------------------------------------|----------------------------|------------------------------------------------------------------|
|                                                                                           | -COOH, -NH <sub>2</sub>    | -OH                                                              |
|                                                                                           |                            |                                                                  |
| -COCl, Acid Anhydride                                                                     | -OH, -NH <sub>2</sub>      | -COOH, -SO <sub>3</sub> H, -PO <sub>3</sub> H <sub>2</sub> ,<br> |
| -SO <sub>2</sub> Cl,                                                                      |                            |                                                                  |
| -COOH, -NHR <sup>9</sup><br>(wherein R <sup>9</sup> is a hydrogen atom or an alkyl group) | -Halogen                   | -COOH, -SO <sub>3</sub> H, -PO <sub>3</sub> H <sub>2</sub> ,<br> |
| -COOH, -NHR <sup>9</sup>                                                                  |                            | -OH                                                              |
|                                                                                           |                            |                                                                  |
| -OH, -NHR <sup>9</sup>                                                                    | -COCl, -SO <sub>2</sub> Cl | -COOH, -SO <sub>3</sub> H, -PO <sub>3</sub> H <sub>2</sub>       |

The chain transfer agent which can be used includes, for example, mercapto compounds having the polar group or a substituent capable of being converted into the polar group later (e.g., thioglycolic acid, thiomalic acid, thisalicylic acid, 2-mercaptopropionic acid, 3-mercaptopropionic acid, 3-mercaptopbutyric acid, N-(2-mercaptopropionyl)glycine, 2-mercaptopicotinic acid, 3-[N-(2-mercaptopethyl)carbamoyl]propionic acid, 3-[N-(2-mercaptopethyl)amino]propionic acid, N-(3-mercaptopropionyl)alanine, 2-mercaptopethane-sulfonic acid, 3-mercaptopropanesulfonic acid, 4-mercaptopbutanesulfonic acid, 2-mercaptopethanol, 3-mercaptop-1,2-propanediol, 1-mercaptop-2-propanol, 3-mercaptop-2-butanol, mercaptophenol, 2-mercaptopethylamine, 2-mercaptopimidazole and 2-mercaptop-3-pyridinol), disulfide compounds which are the oxidation products of these mercapto compounds, and iodized alkyl compounds having the above described polar group or substituent (e.g., iodoacetic acid, iodopropionic acid, 2-iodoethanol, 2-iodoethanol-sulfonic acid and 3-iodopropanesulfonic acid). Of these compounds, the mercapto compounds are preferred.

Also, the polymerization initiator having a specific reactive group which can be used includes, for example, 2,2'-azobis(2-cyanopropanol), 2,2'-azobis(2-cyanopentanol), 4,4'-azobis(4-cyanovaleric acid), 4,4'-azobis(4-cyanovaleric acid chloride), 2,2'-azobis[2-(5-methyl-2-imidazolin-2-yl)propane], 2,2'-azobis[2-(3,4,5,6-tetrahydropyrimidin-2-yl)propane], 2,2'-azobis2-[1-(2-hydroxyethyl)-2-imidazolin-2-yl]propane, 2,2'-azobis[2-methyl-N-(2-hydroxyethyl)propionamide] and the derivatives thereof.

The chain transfer agent or the polymerization initiator is usually used in an amount of from 0.1 to 15% by weight, and preferably from 0.5 to 10% by weight based on the total monomers used.

Specific examples of the macromonomers (M<sub>1</sub>) and (M<sub>2</sub>) used in the present invention are illustrated below. It should also be noted that specific examples of the macromonomer (M<sub>1</sub>) are those shown below but having no specified polar group-containing component. However, the present invention is not to be construed as being limited thereto.

In the following formulae, R<sup>26</sup> represents -H or -CH<sub>3</sub>, R<sup>27</sup>, and R<sup>28</sup> and R<sup>29</sup> each represents -H, -CH<sub>3</sub> or -CH<sub>2</sub>COOCH<sub>3</sub>, R<sup>30</sup> represents -C<sub>k</sub>H<sub>2k+1</sub> (wherein k represents an integer of from 1 to 18), -CH<sub>2</sub>C<sub>6</sub>H<sub>5</sub>,



wherein R<sup>31</sup> and R<sup>32</sup> each represents -H, -Cl, -Br, -CH<sub>3</sub> or -COOCH<sub>3</sub>)



R<sup>33</sup> represents -CN, -OCOCH<sub>3</sub>, -CONH<sub>2</sub> or -C<sub>6</sub>H<sub>5</sub>, R<sup>34</sup> represents -Cl, -Br, -CN or -OCH<sub>3</sub>, m<sub>2</sub> represents an integer of from 2 to 18, n<sub>2</sub> represents an integer of from 2 to 12, and p<sub>2</sub> represents an integer of from 2 to 4.



(M-1)



(M-2)



(M-3)



(M-4)



(M-5)



(M-6)



(M-7)



(M-8)



(M-9)

(M-10)



(M-11)



(M-12)



(M-13)



(M-14)



(M-15)



(M-16)



(M-17)



(M-18)



The macromonomer (M<sub>3</sub>) used in the resin (A<sub>3</sub>) can be synthesized in the following manner. Specifically, it is synthesized according to a method comprising previously protecting the specified polar group in a monomer corresponding to the polymer component having the specified polar group to form a functional group, synthesizing an AB block copolymer by a so-called known living polymerization reaction, for example, an ion polymerization reaction with an organic metal compound (e.g., alkyl lithiums, lithium diisopropylamide and alkylmagnesium halides) or a hydrogen iodide/iodine system, a photopolymerization reaction

50 tion using a porphyrin metal complex as a catalyst, or a group transfer polymerization reaction, then a polymerizable double bond group is introduced into the terminal of the resulting living polymer by a reaction with a various kind of reagents, and thereafter a protection-removing reaction of the functional group which has been formed by protecting the polar group is conducted by a hydrolysis reaction, a hydrogenolysis reaction, an oxidative decomposition reaction, or a photodecomposition reaction to form the polar group. One example thereof is shown by the following reaction scheme (C):



(in case of (a))



(in case of (b))

**Prep**: Protective group for  $-\text{COOH}$ ,

$-\text{b}-$ : A bond connecting two blocks present on both sides.  
n, m: Repeating unit

The living polymer can be easily synthesized according to synthesis methods as described, for example, in P. Lutz, P. Masson et al, *Polym. Bull.*, 12, 79 (1984), B. C. Anderson, G. D. Andrews et al, *Macromolecules*, 14, 1601 (1981), K. Hatada, K. Ute et al, *Polym. J.*, 17, 977 (1985), ibid., 18, 1037 (1986), Koichi Ute and Koichi Hatada, *Kobunshi Kako*

(*Polymer Processing*), 36, 366 (1987), Toshinobu Higashimura and Mitsuo Sawamoto, *Kobunshi Ronbun Shu (Polymer Treatises*, 46, 189 (1989), M. Kuroki and T. Aida, *J. Am. Chem. Soc.*, 109, 4737 (1989), Teizo Aida and Shohei Inoue, *Yuki Gosei Kagaku (Organic Synthesis Chemistry)*, 43, 300

(1985), and D. Y. Sogah, W. R. Hertler et al, *Macromolecules*, 20, 1473 (1987).

Further, in order to introduce a polymerizable double bond group into the terminal of the living polymer, a conventionally known synthesis method for macromonomer can be employed. Specifically, it can be performed by methods as described, for example, in P. Dreyfuss and R. P. Quirk, *Encycl. Polym. Sci. Eng.*, 7, 551 (1987), P. F. Rempp and E. Franta, *Adv. Polym. Sci.*, 58, 1 (1984), V. Percec, *Appl. Polym. Sci.*, 285, 95 (1984), R. Asami and M. Takari, *Makromol. Chem. Suppl.*, 12, 163 (1985), P. Rempp et al., *Makromol. Chem. Suppl.*, 8, 3 (1984), Yushi Kawakami, *Kogaku Kogyo*, 38, 56 (1987), Yuya Yamashita, *Kobunshi*, 31, 988 (1982), Shiro Kobayashi, *Kobunshi*, 30, 625 (1981), Toshinobu Higashimura, *Nippon Seccaku Kyokaishi*, 18, 536 (1982), Koichi Itoh, *Kobunshi Kako*, 35, 262 (1986), Kishiro Higashi and Takashi Tsuda, *Kino Zairyo*, 1987, No. 10, 5, and references and patents cited therein.

Also, the protection of the specified polar group of the present invention by a protective group and the release of the protective group (a reaction for removing the protective group) can be easily conducted by utilizing conventionally known knowledges. More specifically, they can be performed by appropriately selecting methods as described, for example, in Yoshio Iwakura and Keisuke Kurita, *Hannosei Kobunshi (Reactive Polymer)*, Kodansha (1977), T. W. Greene, *Protective Groups in Organic Synthesis*, John Wiley & Sons (1981), and J. F. W. McOmie, *Protective Groups in Organic Chemistry*, Plenum Press, (1973), as well as the methods as described in the above references.

Furthermore, the AB block copolymer can be also synthesized by a photoiniferter polymerization method using a dithiocarbamate compound as an initiator. For example, the block copolymer can be synthesized according to synthesis methods as described, for example, in Takayuki Otsu, *Kobunshi (Polymer)*, 37, 248 (1988), Shunichi Himori and Ryuichi Otsu, *Polym. Rep., Jap.* 37, 3508 (1988), JP-A-64-111 and JP-A-64-26619.

The macromonomer (M) according to the present invention can be obtained by applying the above described synthesis method for macromonomer.

Specific examples of the macromonomer (M3) which can be used in the present invention are set forth below, but the present invention should not be construed as being limited thereto. In the following formulae,  $p^3$ ,  $p^4$  and  $p^5$  each represents  $-H$ ,  $-CH_3$  or  $-CH_2COOCH_3$ ,  $p^6$  represents

$-H$  or  $-CH_3$ ,  $R^{20}$  represents  $-C_pH_{2p+1}$  (wherein  $p$  represents an integer of from 1 to 18),



(wherein  $q$  represents an integer of from 1 to 3),



(wherein  $Y^1$  represents  $-H$ ,  $-Cl$ ,  $-Br$ ,  $-CH_3$ ,  $-OCH_3$  or  $-COCH_3$ )



(wherein  $r$  represents an integer of from 0 to 3),  $R^{12}$  represents  $-C_sH_{2s+1}$  (wherein  $s$  represents an integer of from 1 to 8) or



$Y^2$  represents  $-COOH$ ,  $-SO_3H$ ,



$Y^3$  represents  $-COOH$ ,  $-SO_3H$ ,



$t$  represents an integer of from 2 to 12, and  $u$  represents an integer of from 2 to 6.



(M-101)



(M-102)

-continued



(M-103)



(M-104)



(M-105)



(M-106)



(M-107)



(M-108)



(M-109)

-continued



(M-110)



(M-111)



(M-112)



(M-113)



(M-114)



(M-115)



(M-116)

The resin (A) according to the present invention can be produced by copolymerization of at least one compound each selected from the macromonomers (M) and other monomers (for example, those represented by the general formula (I)) in the desired ratio. The copolymerization can be performed using a known polymerization method, for example, solution polymerization, suspension polymerization, precipitation polymerization, and emulsion polymerization. More specifically, according to the solution polymerization monomers are added to a solvent such as benzene

or toluene in the desired ratio and polymerized with an azobis compound, a peroxide compound or a radical polymerization initiator to prepare a copolymer solution. The solution is dried or added to a poor solvent whereby the desired copolymer can be obtained. In case of suspension polymerization, monomers are suspended in the presence of a dispersing agent such as polyvinyl alcohol or polyvinyl pyrrolidone and copolymerized with a radical polymerization initiator to obtain the desired copolymer.

Now, the resin (B) which can be used as the binder resin for the photoconductive layer of the electrophotographic light-sensitive material according to the present invention will be described in more detail below.

The resin (B) is a starlike polymer comprising an organic molecule having bonded thereto at least three polymer chains each containing a polymer component containing the specified polar group and a polymer component corresponding to a repeating unit represented by the general formula (I). For instance, the starlike polymer according to the present invention can be schematically illustrated below.



(B-1)



(B-2)

wherein X represents an organic molecule, and [Polymer] represents a polymer chain.

Three or more polymer chains which are bonded to the organic molecule may be the same as or different from each other in their structures, and the length of each polymer chain may be the same or different.

As described above, the polymer chain comprises at least one polymer component containing the specified polar group and at least one polymer component represented by the general formula (I), and the composition of the polymer chain may include various embodiments. Specifically, the specified polar group-containing components and the components represented by the general formula (I) each constituting the polymer chain may be present at random or as a block.

In the latter case, the resin (B) is a starlike polymer comprising an organic molecule having bonded thereto at least three AB block polymer chains each containing an A block comprising a polymer component containing the specified polar group and a B block comprising a polymer component represented by the general formula (I). The B block does not contain any specified polar group included in the A block. The A block and the B block in the polymer chain can be arranged in any order. Such a type of the resin (B) can, for example, be schematically illustrated below.



(B-3)



(B-4)

wherein X represents an organic molecule, (A) represents an A block, (B) represents a B block, and (A)-(B) represents a polymer chain.

In another embodiment, the polymer chain in the resin (B) may have one of the above described specified polar group bonded at the terminal thereof opposite to the terminal at which the polymer chain is bonded to the organic molecule. In such a case, the resin (B) is a starlike polymer comprising an organic molecule having bonded thereto at least three polymer chains each containing at least a polymer component represented by the general formula (I) and having the specified polar group bonded at the terminal thereof opposite to the terminal at which the polymer chain is bonded to the organic molecule. Such a type of the resin (B) can, for example, be schematically illustrated below.



(B-5)



(B-6)

wherein X represents an organic molecule, [Polymer] represents a polymer chain, (A) represents an A block, (B) represents a B block, (A)-(B) represents a polymer chain; and W represents a specified polar group.

Particularly, the resin (B) wherein the polymer chain comprises the B block and the A block and the specified polar group is bonded at the terminal of the A block as described in (B-6) above is preferred in view of providing more improved electrostatic characteristics.

In the starlike polymer of the resin (B), a number of the polymer chains bonded to an organic molecule is at most 15, and usually about 10 or less.

The resin (B) is characterized by containing from 0.01 to 10% by weight of polymer component containing the specified polar group and not less than 30% by weight of polymer component represented by the general formula (I) bases on the resin (B) as described above.

If the content of the polar group-containing component in the resin (B) is less than 0.01% by weight, the initial potential is low and thus satisfactory image density can not be obtained. On the other hand, if the content of the polar group-containing component is larger than 10% by weight, various undesirable problems may occur, for example, the dispersibility of particles of photoconductive substance is reduced, the film smoothness and the electrophotographic characteristics under high temperature and high humidity condition deteriorate, and further when the light-sensitive material is used as an offset master plate, the occurrence of background stains increases. The amount of the polar group-

containing component in the resin (B) is preferably from 0.05 to 8% by weight.

It is also preferred that the total amount of the specified polar group-containing polymer component contained in the resin (B) is from 10 to 50% by weight based on the total amount of the specified polar group-containing polymer component present in the resin (A).

If the total amount of the specified polar group-containing component in the resin (B) is less than 10% by weight of that in the resin (A), the electrophotographic characteristics (particularly, dark charge retention rate and photosensitivity) and film strength tend to decrease. On the other hand, if it is larger than 50% by weight, a sufficiently uniform dispersion of particles of photoconductive substance may not be obtained, whereby the electrophotographic characteristics decrease and water retentivity decline when used as an offset master plate.

The content of the polymer component represented by the general formula (I) in the resin (B) is preferably not less than 50% by weight.

The weight average molecular weight of the resin (B) is from  $3 \times 10^4$  to  $1 \times 10^6$ , and preferably from  $5 \times 10^4$  to  $5 \times 10^5$ . If the weight average molecular weight of the resin (B) is less than  $3 \times 10^4$ , the film-forming property of the resin is lowered, whereby a sufficient film strength cannot be maintained, while if the weight average molecular weight of the resin (B) is higher than  $1 \times 10^6$ , the effect of the resin (B) of the present invention is reduced, whereby the electrophotographic characteristics thereof become almost the same as those of conventionally known resins.

The glass transition point of the resin (B) is preferably from  $-10^\circ$  C. to  $100^\circ$  C., and more preferably from  $0^\circ$  C. to  $90^\circ$  C.

The polymer component having the specified polar group (including that is present in the polymer chain and/or at the terminal of the polymer chain) and the polymer component represented by the general formula (I) are the same as those described in detail for the resin (A) hereinbefore.

The resin (B) may contain other polymer components than the polymer components described above. Preferred examples of such other polymer components include those corresponding to the repeating unit represented by the general formula (II) as described in detail with respect to the resin (A) above.

Moreover, the resin (B) may further contain other polymer components corresponding to monomers copolymerizable with monomers corresponding to the polymer components represented by the general formula (II). Examples of such monomers include acrylonitrile, methacrylonitrile and heterocyclic vinyl compounds (e.g., vinylpyridine, vinylimidazole, vinylpyrrolidone, vinylthiophene, vinylpyrazoles, vinyldioxane and vinyloxazine). However, such other monomers are preferably employed in an amount of not more than 20 parts by weight per 100 parts by weight of the resin (B).

The organic molecule to which at least three polymer chains are bonded and which is used in the resin (B) according to the present invention is any organic molecule having a molecular weight of 1000 or less. Suitable examples of the organic molecules include those containing a trivalent or more hydrocarbon moiety shown below.



5

-continued



wherein ( ) represents a repeating unit;  $r^1$ ,  $r^2$ ,  $r^3$  and  $r^4$  each represents a hydrogen atom or a hydrocarbon group, provided that at least one of  $r^1$  and  $r^2$  or  $r^3$  and  $r^4$  is bonded to a polymer chain.

These organic moieties may be employed individually or as a combination thereof. In the latter case, the combination may further contain an appropriate linking unit, for example,  $-\text{O}-$ ,  $-\text{S}-$ ,

15



(wherein  $r^7$  represents a hydrogen atom or a hydrocarbon group),  $-\text{CO}-$ ,  $-\text{CS}-$ ,  $-\text{COO}-$ ,

25



$-\text{NHCOO}-$ ,  $-\text{NHCONH}-$  and a heterocyclic group containing at least one hetero atom such as oxygen, sulfur or nitrogen (e.g., thiophene, pyridine, pyran, imidazole, benzimidazole, furan, piperidine, pyrazine, pyrrole and piperazine, as the hetero ring).

Other examples of the organic molecules to which the polymer chains are bonded include those comprising a combination of

30



with a linking unit described above. However, the organic molecules which can be used in the present invention should not be construed as being limited to those described above.

The starlike polymer according to the present invention can be prepared by utilizing conventionally known synthesis methods of starlike polymers using monomers containing a polar group and a polymerizable double bond group. For instance, a method of polymerization reaction using a carboanion as an initiator can be employed. Such a method is specifically described in M. Morton, T. E. Helminiak et al, *J. Polym. Sci.*, 57, 471 (1962), B. Gordon III, M. Blumenthal, J. E. Loftus, et al *Polym. Bull.*, 11, 349 (1984), and R. B. Bates, W. A. Beavers, et al, *J. Org. Chem.*, 44, 3800 (1979). In case of using the reaction, it is required that the specified polar group be protected to form a functional group and the protective group be removed after polymerization.

The protection of the specified polar group of the present invention by a protective group and the release of the protective group (a reaction for removing a protective group) can be easily conducted by utilizing conventionally known knowledges. More specifically, they can be performed by appropriately selecting methods described, e.g., in Yoshio Iwakura and Keisuke Kurita, *Hannsei Kobunshi (Reactive Polymer)*, Kodansha (1977), T. W. Greene, *Protective Groups in Organic Synthesis*, John Wiley & Sons (1981), and J. F. W. McOmie, *Protective Groups in Organic Chemistry*, Plenum Press, (1973), as well as methods as described in the above references.

Further, in another method, the polymer can be synthesized by conducting a polymerization reaction under light

35

40

45

50

55

60

65

irradiation using a monomer having the unprotected polar group and also using a dithiocarbamate group-containing compound and/or a xanthate group-containing compound as an initiator. For example, copolymer can be synthesized according to the synthesis methods described, e.g., in Takyu Otsu, *Kobunshi (Polymer)*, 37, 248 (1988), Shunichi Himori and Ryichi Otsu, *Polym. Rep. Jap.* 37, 3508 (1988), JP-A-64-111, JP-A-64-26619, Nobuyuki Higashi et al, *Polymer Preprints Japan*, 36 (6) 1511 (1987), and M. Niwa, N. Higashi et al, *J. Macromol. Sci. Chem.*, A24(5), 567 (1987).

The ratio of resin (A) to resin (B) used in the present invention is preferably 0.05 to 0.60/0.95 to 0.40, more preferably 0.10 to 0.40/0.90 to 0.60 in terms of a weight ratio of resin (A)/resin (B).

When the weight ratio of resin (A)/resin (B) is less than 0.05, the effect for improving the electrostatic characteristics may be reduced. On the other hand, when it is more than 0.60, the film strength of the photoconductive layer may not be sufficiently maintained in some cases (particularly, in case of using as an electrophotographic printing plate precursor).

The resin (A) used in the photoconductive layer according to the present invention includes three embodiments of the resins (A<sub>1</sub>), (A<sub>2</sub>) and (A<sub>3</sub>) as described above. Two or more kinds of each of the resins (A) and the resins (B) may be employed in the photoconductive layer. What is important is that the resin (A) and the resin (B) are employed in the ratio described above.

Furthermore, in the present invention, the binder resin used in the photoconductive layer may contain other resin(s) known for inorganic photoconductive substance in addition to the resin (A) and the resin (B) according to the present invention. However, the amount of other resins described above should not exceed 30 parts by weight per 100 parts by weight of the total binder resins since, if the amount is more than 30 parts by weight, the effects of the present invention are remarkably reduced.

Representative other resins which can be employed together with the resins (A) and (B) according to the present invention include vinyl chloride-vinyl acetate copolymers, styrene-butadiene copolymers, styrene-methacrylate copolymers, methacrylate copolymers, acrylate copolymers, vinyl acetate copolymers, polyvinyl butyral resins, alkyd resins, silicone resins, epoxy resins, epoxyester resins, and polyester resins.

Specific examples of other resins used are described, for example, in Takaharu Shibata and Jiro Ishiwatari, *Kobunshi (High Molecular Materials)*, 17, 278 (1968), Harumi Miyamoto and Hidehiko Takei, *Imaging* No. 8, 9 (1973), Koichi Nakamura, *Kiroku Zairyoyo Binder no Jissai Gijutsu (Practical Technique of Binders for Recording Materials)*, Cp. 10, published by C. M. C. Shuppan (1985), D. Tatt, S. C. Heidecker *Tappi*, 49, No. 10, 439 (1966), E. S. Baltazzi, R. G. Blanquette, et al., *Photo. Sci. Eng.*, 16, No. 5, 354 (1972), Nguyen Chank Keh, Isamu Shimizu and Eiichi Inoue, *Densi Shashin Gakkaishi (Journal of Electrophotographic Association)*, 18, No. 2, 22 (1980), JP-B-50-31011, JP-A-53-54027, JP-A-54-20735, JP-A-57-202544 and JP-A-58-68046.

The total amount of binder resin used in the photoconductive layer according to the present invention is preferably from 10 to 100 parts by weight, more preferably from 15 to 50 parts by weight, per 100 parts by weight of the inorganic photoconductive substance.

When the total amount of binder resin used is less than 10 parts by weight per 100 parts by weight of the inorganic photoconductive substance, it may be difficult to maintain

the film strength of the photoconductive layer. On the other hand, when it is more than 100 parts by weight, the electrostatic characteristics may decrease and the image forming performance may degrade to result in the formation of poor duplicated image.

The inorganic photoconductive substance which can be used in the present invention includes zinc oxide, titanium oxide, zinc sulfide, cadmium sulfide, cadmium carbonate, zinc selenide, cadmium selenide, tellurium selenide, and lead sulfide.

As the spectral sensitizing dye which can be used in the present invention, various dyes can be employed individually or as a combination of two or more thereof. Examples of the spectral sensitizing dyes include, for example, carbonium dyes, diphenylmethane dyes, triphenylmethane dyes, xanthene dyes, phthalein dyes, polymethine dyes (e.g., oxonol dyes, merocyanine dyes, cyanine dyes, rhodacyanine dyes, and styryl dyes), and phthalocyanine dyes (including metallized dyes) as described for example, in Harumi Miyamoto and Hidehiko Takei, *Imaging*, 1973, No. 8, 12, C. J. Young et al., *RCA Review*, 15, 469 (1954), Kohei Kiyota et al., *Denkisushin Gakkai Ronbunshi*, J 63-C, No. 2, 97 (1980), Yuj i Harasaki et al., *Kogyo Kagaku Zasshi*, 66, 78 and 188 (1963), Tadaaki Tani, *Nihon Shashin Gakkaishi*, 35, 208 (1972).

Specific examples of the carbonium dyes, triphenylmethane dyes, xanthene dyes, and phthalein dyes are described, for example, in JP-B-51-452, JP-A-50-90334, JP-A-50-114227, JP-A-53-39130, JP-A-53-82353, U.S. Pat. Nos. 3,052,540 and 4,054,450, and JP-A-57-16456.

The polymethine dyes, such as oxonol dyes, merocyanine dyes, cyanine dyes, and rhodacyanine dyes, include those described, for example, in F. M. Hamer, *The Cyanine Dyes and Related Compounds*. Specific examples include those described, for example, in U.S. Pat. Nos. 3,047,384, 3,110, 591, 3,121,008, 3,125,447, 3,128,179, 3,132,942, and 3,622, 317, British Patents 1,226,892, 1,309,274 and 1,405,898, JP-B-48-7814 and JP-B-55-18892.

In addition, polymethine dyes capable of spectrally sensitizing in the longer wavelength region of 700 nm or more, i.e., from the near infrared region to the infrared region, include those described, for example, in JP-A-47-840, JP-A-47-44180, JP-B-51-41061, JP-A-49-5034, JP-A-49-45122, JP-A-57-46245, JP-A-56-35141, JP-A-57-157254, JP-A-61-26044, JP-A-61-27551, U.S. Pat. Nos. 3,619,154 and 4,175,956, and *Research disclosure*, 216, 117 to 118 (1982).

The electrophotographic light-sensitive material of the present invention is excellent in that the performance properties thereof are not liable to variation even when various kinds of sensitizing dyes are employed together.

If desired, the photoconductive layer may further contain various additives commonly employed in conventional electrophotographic light-sensitive layer, such as chemical sensitizers. Examples of such additives include electron-accepting compounds (e.g., halogen, benzoquinone, chloranil, acid anhydrides, and organic carboxylic acids) as described in the above-mentioned *Imaging*, 1973, No. 8, 12; and polyarylkane compounds, hindered phenol compounds, and p-phenylenediamine compounds as described in Hiroshi Kokado et al., *Saikin-no Kododen Zairyō to Kankotai no Kaihatsu Jitsuyōka*, Chaps. 4 to 6, Nippon Kagaku Joho K.K. (1986).

The amount of these additives is not particularly restricted and usually ranges from 0.0001 to 2.0 parts by weight per 100 parts by weight of the photoconductive substance.

The photoconductive layer suitably has a thickness of from 1 to 100  $\mu$ m, preferably from 10 to 50  $\mu$ m.

In cases where the photoconductive layer functions as a charge generating layer in a laminated light-sensitive mate-

rial composed of a charge generating layer and a charge transporting layer, the thickness of the charge generating layer suitably ranges from 0.01 to 1  $\mu\text{m}$ , preferably from 0.05 to 0.5  $\mu\text{m}$ .

If desired, an insulating layer can be provided on the light-sensitive layer of the present invention. When the insulating layer is made to serve for the main purposes for protection and improvement of durability and dark charge characteristics of the light-sensitive material, its thickness is relatively small. When the insulating layer is formed to provide the light-sensitive material suitable for application to special electrophotographic processes, its thickness is relatively large, usually ranging from 5 to 70  $\mu\text{m}$ , preferably from 10 to 50  $\mu\text{m}$ .

Charge transporting materials in the above-described laminated light-sensitive material include polyvinylcarbazole, oxazole dyes, pyrazoline dyes, and triphenylmethane dyes. The thickness of the charge transporting layer ranges usually from 5 to 40  $\mu\text{m}$ , preferably from 10 to 30  $\mu\text{m}$ .

Resins to be used in the insulating layer or charge transporting layer typically include thermoplastic and thermosetting resins, e.g., polystyrene resins, polyester resins, cellulose resins, polyether resins, vinyl chloride resins, vinyl acetate resins, vinyl chloride-vinyl acetate copolymer resins, polyacrylate resins, polyolefin resins, urethane resins, epoxy resins, melamine resins, and silicone resins.

The photoconductive layer according to the present invention can be provided on any known support. In general, a support for an electrophotographic light-sensitive layer is preferably electrically conductive. Any of conventionally employed conductive supports may be utilized in the present invention. Examples of usable conductive supports include a substrate (e.g., a metal sheet, paper, and a plastic sheet) having been rendered electrically conductive by, for example, impregnating with a low resistant substance; the above-described substrate with the back side thereof (opposite to the light-sensitive layer side) being rendered conductive and having further coated thereon at least one layer for the purpose of prevention of curling; the above-described substrate having provided thereon a water-resistant adhesive layer; the above-described substrate having provided thereon at least one precoat layer; and paper laminated with a conductive plastic film on which aluminum is vapor deposited.

Specific examples of conductive supports and materials for imparting conductivity are described, for example, in Yukio Sakamoto, *Denshishashin*, 14, No. 1, pp. 2 to 11 (1975), Hiroyuki Moriga, *Nyumon Tokushushi no Kagaku*,

Kobunshi Kankokai (1975), and M. F. Hoover, *J. Macromol. Sci. Chem.* A-4(6), pp. 1327 to 1417 (1970).

The electrophotographic light-sensitive material according to the present invention can be utilized in any known electrophotographic process. Specifically, the light-sensitive material of the present invention is employed in any recording system including a PPC system and a CPC system in combination with any developer including a dry type developer and a liquid developer. In particular, the light-sensitive material is preferably employed in combination with a liquid developer in order to obtain the excellent effect of the

present invention since the light-sensitive material is capable of providing faithfully duplicated image of highly accurate original.

Further, a color duplicated image can be produced by using it in combination with a color developer in addition to the formation of black and white image. Reference can be made to methods described, for example, in Kuro Takizawa, *Shashin Kogyo*, 33, 34 (1975) and Masayasu Anzai, *Den-shitsushin Gakkai Giutsu Kenkyu Hokoku*, 77, 17 (1977).

Moreover, the light-sensitive material of the present invention is effective for recent other uses utilizing an electrophotographic process. For instance, the light-sensitive material containing photoconductive zinc oxide as a

photoconductive substance is employed as an offset printing plate precursor, and the light-sensitive material containing photoconductive zinc oxide or titanium oxide which does not cause environmental pollution and has good whiteness is employed as a recording material for forming a block copy usable in an offset printing process or a color proof.

## BEST MODE FOR CONDUCTING THE INVENTION

The present invention is illustrated in greater detail with reference to the following examples wherein the molecular weights of macromonomers M-1, M-2, M-4 and M-101, and of resins A-1, A-11, A-29 and A-101 where measured by GPC, but the present invention is not to be construed as being limited thereto.

Synthesis examples of the resin (A) are specifically illustrated below.

## SYNTHESIS EXAMPLE 1 OF MACROMONOMER: (M-1)

A mixed solution of 75 g of methyl methacrylate, 25 g of methyl acrylate, 5 g of thioglycolic acid, and 200 g of toluene was heated to a temperature of 75°C. with stirring under nitrogen gas stream and, after adding thereto 1.0 g of 2,2-azobisisobutyronitrile (A.I.B.N.), the reaction was carried out for 8 hours. Then, to the reaction mixture were added 8 g of glycidyl methacrylate, 1.0 g of N,N-dimethyldodecylamine, and 0.5 g of *t*-butylhydroquinone, and the resulting mixture was stirred for 12 hours at a temperature of 100°C. After cooling, the reaction mixture was reprecipitated from 2 liters of *n*-hexane to obtain 82 g of white powder. A weight average molecular weight (M<sub>w</sub>) of the resulting polymer was  $3.8 \times 10^3$ .



## SYNTHESIS EXAMPLE 2 OF MACROMONOMER: (M-2)

A mixed solution of 90 g of butyl methacrylate, 10 g of methacrylic acid, 4 g of 2-mercaptoethanol, and 200 g of tetrahydrofuran was heated to a temperature of 70° C. with stirring under nitrogen gas stream and, after adding thereto 1.2 g of A.I.B.N., the reaction was carried out for 8 hours.

Then, the reaction mixture was cooled to a temperature of 20° C. in a water bath and, after adding thereto 10.2 g of triethylamine, 14.5 g of methacrylic acid chloride was added.

dropwise to the mixture with stirring at a temperature of lower than 25° C. Thereafter, the mixture was further stirred for one hour. Then, 0.5 g of t-butylhydroquinone was added to the mixture, and the resulting mixture was heated to a temperature of 60° C. and stirred for 4 hours.

After cooling, the reaction mixture was added dropwise to one liter of water with stirring (over a period of about 10 minutes) followed by stirring for one hour. After allowing to stand the mixture, water was removed by decantation. After washing twice with water, the reaction mixture was dissolved in 100 ml of tetrahydrofuran, and the solution was reprecipitated from 2 liters of petroleum ether. The precipitates thus formed were collected by decantation and dried under reduced pressure to obtain 65 g of the viscous product having an Mw of  $3.3 \times 10^3$ .



SYNTHESIS EXAMPLE 3 OF  
MACROMONOMER: (M-3)

A mixed solution of 95 g of benzyl methacrylate, 5 g of 2-phosphonoethyl methacrylate, 6 g of 2-amino-ethylmercaptan, and 200 g of tetrahydrofuran was heated to a temperature of 70° C. with stirring under nitrogen gas stream. After adding thereto 1.5 g of A.I.B.N., the reaction was carried out for 4 hours and, after further adding thereto 0.5 g of A.I.B.N., the reaction was carried out for 4 hour.

Then, the reaction mixture was cooled to a temperature of 20° C. and after adding thereto 10 g of acrylic anhydride, the resulting mixture was stirred for one hour at a temperature of from 20° to 25° C. Then, 1.0 g of t-butylhydroquinone was added to the mixture, followed by stirring for 4 hours at a temperature of from 50° to 60° C. After cooling, the reaction mixture was added dropwise to one liter of water with stirring over a period of about 10 minutes followed by stirring for one hour and, after allowing the reaction mixture to stand, water was removed by decantation. After repeatedly washing the mixture twice with water, the reaction mixture was dissolved in 100 ml of tetrahydrofuran, and the solution was reprecipitated from 2 liters of petroleum ether. The precipitates formed were collected by decantation and dried under reduced pressure to obtain 70 g of the viscous product having an Mw of  $6 \times 10^3$ .



SYNTHESIS EXAMPLE 4 OF  
MACROMONOMER: (M-4)

A mixed solution of 90 g of 2-chlorophenyl methacrylate, 10 g of Monomer (I) having the structure shown below, 4 g of thioglycolic acid, and 200 g of toluene was heated to a temperature of 70° C. with stirring under nitrogen gas stream. After adding thereto 1.5 g of A.I.B.N., the reaction was carried out for 5 hours and, after further adding thereto

0.5 g of A.I.B.N., the reaction was carried out for 4 hour. Then, after adding thereto 12.4 g of glycidyl methacrylate, 1.0 g of N,N-dimethyldodecylamine, 1.5 g of t-butylhydroquinone, the reaction was carried out for 8 hours at a temperature of 110° C. After cooling, the reaction mixture was added to a mixture of 3 g of p-toluenesulfonic acid and 100 ml of an aqueous solution of 90% by volume tetrahydrofuran followed by stirring for one hour at a temperature of from 30° to 35° C. The reaction mixture was reprecipitated from 2 liters of a water/ethanol (1/3 by volume) mixed solution, and the precipitates formed were collected by decantation. The precipitates were dissolved in 200 ml of tetrahydrofuran, and the solution was reprecipitated from 2 liters of n-hexane to obtain 58 g of the powder. An Mw of the polymer was  $7.6 \times 10^3$ .



SYNTHESIS EXAMPLE 5 OF  
MACROMONOMER: (M-5)

A mixed solution of 95 g of 2,6-dichlorophenyl methacrylate, 5 g of 3-(2'-nitrobenzyloxy)sulfonylpropyl methacrylate, 150 g of toluene, and 50 g of isopropyl alcohol was heated to a temperature of 80° C. with stirring under nitrogen gas stream. After adding thereto 5.0 g of 2,2'-azobis(2-cyanovaleic acid) (A.C.V.), the reaction was carried out for 5 hours and, after further adding thereto 1.0 g of A.C.V., the reaction was carried out for 4 hours. After cooling, the reaction mixture was reprecipitated from 2 liters of methanol, and the powder formed was collected by filtration and dried under reduced pressure.

A mixture of 50 g of the powder prepared above, 14 g of glycidyl methacrylate, 0.6 g of N,N-dimethyldocylamine,

(M-3)

60 1.0 g of t-butylhydroquinone, and 100 g of toluene was stirred for 10 hours at a temperature of 110° C. After cooling the mixture to a room temperature, the mixture was irradiated by a high-pressure mercury lamp of 80 W for one hour with stirring. Thereafter, the reaction mixture was reprecipitated from one liter of methanol, and the powder formed was collected by filtration and dried under reduced pressure. The yield was 34 g, and the Mw was  $7.3 \times 10^3$ .



(M-5)

SYNTHESIS EXAMPLE 6 OF  
MACROMONOMER: (M-6)

A mixed solution of 80 g of ethyl methacrylate, 5 g of N-vinylpyrrolidone, 29 g of trimethylsilyl methacrylate, 3 g of B-mercaptopropanoic acid, and 200 g of tetrahydrofuran was heated to a temperature of 70° C. with stirring under nitrogen gas stream. After adding thereto 1 g of A.I.B.N., the reaction was carried out for 4 hours and after further adding thereto 0.5 g of A.I.B.N., the reaction was carried out for 4 hours. The reaction mixture was cooled to a temperature of 25° C. and after adding thereto 6.6 g of methacrylic acid, a mixed solution of 8 g of dicarboxylcarbodiimide (D.C.C.), 0.2 g of 4-(N,N-dimethylamino)pyridine and 20 g of methylene chloride was added dropwise to the mixture at a temperature of from 25° to 30° C., followed by stirring for 4 hours under the same condition. Then, 10 g of formic acid

15

20

30

35



SYNTHESIS EXAMPLE i OF RESIN (A): (A-1)

A mixed solution of 70 g of benzyl methacrylate, 30 g of Macromonomer (M-1), 150 g of toluene, and 50 g of isopropanol was heated to a temperature of 80° C. under nitrogen gas stream, and 5 g of A.C.V. was added thereto to effect a reaction for 4 hours. To the reaction mixture was further added 0.5 g of A.C.V., followed by reacting for 4 hours. The resulting copolymer had a weight average molecular weight (Mw) of  $1.0 \times 10^4$ .



Resin (A-1)

SYNTHESIS EXAMPLE 2 OF RESIN (A): (A-2)

A mixed solution of 80 g of 2-chlorophenyl methacrylate, 20 g of a macromonomer corresponding to a repeating unit having the structure shown below (Mw:  $5 \times 10^3$ ), 3.0 g of  $\beta$ -mercaptopropionic acid, and 200 g of toluene was heated to a temperature of 75° C. under nitrogen gas stream. After adding thereto 1.5 g of A.I.B.N., the reaction was carried out for 4 hours. After further adding thereto 0.5 g of A.I.B.N., the reaction was carried out for 4 hours. The resulting copolymer had an Mw of  $8.8 \times 10^3$ .

50 was added to the reaction mixture, followed by stirring for one hour. The insoluble substance deposited was removed by filtration, the filtrate was reprecipitated from one liter of methanol to collect the oily product by filtration. The oily product was dissolved in 200 g of tetrahydrofuran, and after removing the insoluble substance by filtration, the filtrate was again reprecipitated from one liter of methanol. The resulting oily product was collected and dried. The yield was 65 g, and the Mw was  $7 \times 10^3$ .

50

55



10

## SYNTHESIS EXAMPLES 3 TO 9 OF RESIN (A): (A-3) to (A-9)

Each of the copolymers shown in Table 2 below was synthesized in the same manner as described in Synthesis Example 2 of Resin (A) except for using each of monomers and macromonomers corresponding to the repeating units shown in Table 2 below in place of 80 g of 2-chlorophenyl methacrylate and 20 g of the macromonomer in Synthesis Example 2 of Resin (A). The Mw of each of the copolymers was in a range of from  $7.5 \times 10^3$  to  $9 \times 10^3$ . The Mw of each of the macromonomers used was in a range of from  $3.5 \times 10^3$  to  $5 \times 10^3$ .



(A-2)

## SYNTHESIS EXAMPLE 10 OF RESIN (A): (A-10)

15 A mixed solution of 70 g of benzyl methacrylate, 30 g of  
Macromonomer (M-4), and 200 g of toluene was heated to  
a temperature of 80° C. under nitrogen gas stream, and 8 g  
of 2,2'-azobisvaleronitrile (A.I.V.N.) was added thereto to  
effect a reaction for 3 hours. To the reaction mixture was  
further added 1 g of A.I.V.N., followed by reacting for 4  
20 hours. The resulting polymer had an  $M_w$  of  $8.5 \times 10^3$ .

TABLE 2

| $  \begin{array}{c}  \text{HOOC(CH}_2)_2\text{S} \left[ \begin{array}{c} \text{CH}_3 & \text{CH}_3 \\   &   \\ -\text{CH}_2-\text{C} & -\text{CH}_2-\text{C} \\   &   \\ \text{x}_1 & \text{y}_1 \\   &   \\ \text{COOR}^{31} & \text{COOR}^{31} \end{array} \right] \\  \text{COO(CH}_2)_2\text{S} \left[ \begin{array}{c} \text{CH}_3 \\   \\ -\text{CH}_2-\text{C} \\   \\ \text{x}_2 \\   \\ \text{Y} \\   \\ \text{COOR}^{32} \end{array} \right] \\  \end{array}  $ |           |                                                                                     |                                           |                                                                                     |                                                                                                                   |                                           |
|---------------------------------------------------------------------------------------------------------------------------------------------------------------------------------------------------------------------------------------------------------------------------------------------------------------------------------------------------------------------------------------------------------------------------------------------------------------------------|-----------|-------------------------------------------------------------------------------------|-------------------------------------------|-------------------------------------------------------------------------------------|-------------------------------------------------------------------------------------------------------------------|-------------------------------------------|
| Synthesis Example of Resin (A)                                                                                                                                                                                                                                                                                                                                                                                                                                            | Resin (A) | $\text{R}^{31}$                                                                     | $\text{x}^1/\text{y}^1$<br>(weight ratio) | $-\text{R}^{32}$                                                                    | $-\text{Y}-$                                                                                                      | $\text{x}^2/\text{y}^2$<br>(weight ratio) |
| 3                                                                                                                                                                                                                                                                                                                                                                                                                                                                         | A-3       | $-\text{CH}_3$                                                                      | 70/30                                     | $-\text{CH}_2\text{C}_6\text{H}_5$                                                  | —                                                                                                                 | 100/0                                     |
| 4                                                                                                                                                                                                                                                                                                                                                                                                                                                                         | A-4       | $-\text{C}_6\text{H}_5$                                                             | 60/40                                     | $-\text{CH}_2\text{C}_6\text{H}_5$                                                  | —                                                                                                                 | 100/0                                     |
| 5                                                                                                                                                                                                                                                                                                                                                                                                                                                                         | A-5       | $-\text{C}_2\text{H}_5$                                                             | 75/25                                     | $-\text{CH}_2\text{C}_6\text{H}_5$                                                  | $-\text{CH}_2-\text{CH}-$<br>$\text{COOCH}_2\text{C}_6\text{H}_5$                                                 | 60/40                                     |
| 6                                                                                                                                                                                                                                                                                                                                                                                                                                                                         | A-6       | $-\text{CH}_2\text{C}_6\text{H}_5$                                                  | 80/20                                     | $-\text{CH}_3$                                                                      | $-\text{CH}_2-\text{CH}-$<br> | 95/5                                      |
| 7                                                                                                                                                                                                                                                                                                                                                                                                                                                                         | A-7       | $-\text{CH}_2\text{C}_6\text{H}_5$                                                  | 60/40                                     |  | $-\text{CH}_2\text{CH}-$<br>$\text{C}\equiv\text{N}$                                                              | 95/5                                      |
| 8                                                                                                                                                                                                                                                                                                                                                                                                                                                                         | A-8       |  | 80/20                                     | $-\text{C}_6\text{H}_5$                                                             | —                                                                                                                 | 100/0                                     |
| 9                                                                                                                                                                                                                                                                                                                                                                                                                                                                         | A-9       |  | 75/25                                     |  | $-\text{CH}_2\text{CH}-$<br>$\text{COOCH}_3$                                                                      | 80/20                                     |



SYNTHESIS EXAMPLE 11 OF RESIN (A):  
(A-11)

A mixed solution of 60 g of 2-chlorophenyl methacrylate, 35 g of Macromonomer (M-2), 5 g of 2-methoxyethyl methacrylate, 3 g of octadecyl methacrylate, and 200 g of toluene was heated to a temperature of 75° C. under nitrogen gas stream, and 1.0 g of A.I.B.N. was added thereto to effect a reaction for 3 hours. After further adding thereto 0.5 g of A.I.B.N., the reaction was carried out for 3 hours, and after further adding thereto 0.5 g of A.I.B.N., the reaction was carried out for 3 hours. After cooling, the reaction mixture was reprecipitated from one liter of ether, the resulting precipitates were collected and dried to obtain 63 g of the viscous product having an  $M_w$  of  $6.5 \times 10^3$ .

15

20

25

SYNTHESIS EXAMPLES 12 TO 19 OF RESIN  
(A): (A-12) to (A-19)

Each of the polymers shown in Table 3 below was synthesized in the same procedure as described in Synthesis Example 11 of Resin (A) except for using each of monomers and macromonomers corresponding to the polymer components shown in Table 3 below in place of the monomer and macromonomer in Synthesis Example 11 of Resin (A). The  $M_w$  of each of the copolymers was in a range of from  $6 \times 10^3$  to  $8 \times 10^3$ .



TABLE 3

| Synthesis Example of Resin (A) | Resin (A) | $R^{33}$                                                                                         | $R^{34}$                                                                                       | $x^3/y^3$<br>(weight ratio) | $-Y^2-$                                                                                                 |  |
|--------------------------------|-----------|--------------------------------------------------------------------------------------------------|------------------------------------------------------------------------------------------------|-----------------------------|---------------------------------------------------------------------------------------------------------|--|
|                                |           |                                                                                                  |                                                                                                |                             | $\left[ -CH_2 - C_{\gamma_3}^{(Y^2)_{\gamma_3}} - \right]$                                              |  |
| 12                             | A-12      | $-C_2H_5$                                                                                        |               | 90/10                       | $-CH_2 - CH -$<br>   |  |
| 13                             | A-13      | $-C_3H_7$                                                                                        | $-CH_2 -$<br> | 85/15                       | $-CH_2 - C -$<br>    |  |
| 14                             | A-14      | $-C_4H_9$                                                                                        |               | 90/10                       | $-CH_2 - C -$<br>    |  |
| 15                             | A-15      |                | $-CH_3$                                                                                        | 90/10                       | $-CH_2 - CH -$<br>  |  |
| 16                             | A-16      | $-CH_2 -$<br> | $-C_2H_5$                                                                                      | 90/10                       | $-CH_2 - CH -$<br> |  |
| 17                             | A-17      |               | $-C_4H_9$                                                                                      | 92/8                        | $-CH_2 - C -$<br>  |  |
| 18                             | A-18      | $-CH_3$                                                                                          |             | 93/7                        | $-CH_2 - C -$<br>  |  |
| 19                             | A-19      | $-CH_3$                                                                                          | $-C_2H_5$                                                                                      | 90/10                       | $-CH_2 - C -$<br>  |  |

SYNTHESIS EXAMPLE 20 OF RESIN (A):  
(A-20)

A mixed solution of 70 g of 2-chlorophenyl methacrylate, 65 30 g of Macromonomer (M-3), 3.0 g of thioglycolic acid, and 150 g of toluene was heated to a temperature of 80° C.

under nitrogen gas stream, and 1.0 g of A.I.B.N. was added thereto to effect a reaction for 4 hours. After further adding thereto 0.5 g of A.I.B.N., the reaction was carried out for 2 hours, and after further adding 0.3 g of A.I.B.N., the reaction

was carried out for 3 hours. The resulting copolymer had an Mw of  $8.5 \times 10^3$ .



**SYNTHESIS EXAMPLES 21 TO 28 OF RESIN  
(A): (A-21) to (A-28)**

Each of the copolymers shown in Table 4 below was synthesized by a polymerization reaction in the same man-

ner as described in Synthesis Example 20 of Resin (A) using 15 each of 60 g of monomers, 40 g of macromonomers and 0.04 moles of mercapto compounds corresponding to the components shown in Table 4 below. The Mw of each of the copolymers was in a range of from  $6 \times 10^3$  to  $9 \times 10^3$ .

20

25

30

35

40

45

50

55

60

65

TABLE 4

| Synthesis Example of Resin (A) | Resin (A) | W-                                | R <sup>35</sup>          | R <sup>36</sup>                | x'/y <sup>a</sup><br>(weight ratio) | -Y <sup>3-</sup> -                                                       |
|--------------------------------|-----------|-----------------------------------|--------------------------|--------------------------------|-------------------------------------|--------------------------------------------------------------------------|
|                                |           |                                   | HOOC-H <sub>2</sub> C-S- | -C <sub>2</sub> H <sub>5</sub> | 90/10                               | -CH <sub>2</sub> -CH-                                                    |
| 21                             | A-21      |                                   |                          |                                |                                     | COO(CH <sub>2</sub> ) <sub>2</sub> COO(CH <sub>2</sub> ) <sub>2</sub> S- |
|                                |           |                                   |                          |                                |                                     | CH <sub>3</sub>                                                          |
|                                |           |                                   |                          |                                |                                     | COOR <sup>36</sup>                                                       |
|                                |           |                                   |                          |                                |                                     | OH                                                                       |
|                                |           |                                   |                          |                                |                                     |                                                                          |
| 22                             | A-22      | HOOC-CH <sub>2</sub><br>HOOC-CHS- |                          |                                | 85/15                               | CH <sub>2</sub> COOH                                                     |
|                                |           |                                   |                          |                                |                                     | -CH <sub>2</sub> -C-                                                     |
|                                |           |                                   |                          |                                |                                     | COOH                                                                     |
| 23                             | A-23      |                                   |                          |                                | 90/10                               |                                                                          |
|                                |           |                                   |                          |                                |                                     | -CH <sub>2</sub> -C-                                                     |
|                                |           |                                   |                          |                                |                                     | CONH-                                                                    |
|                                |           |                                   |                          |                                |                                     | COOH                                                                     |
|                                |           |                                   |                          |                                |                                     |                                                                          |

TABLE 4-continued

| Synthesis Example of Resin (Å) | Resin (Å) | W -                                                                                                             | R <sup>35</sup>                | R <sup>36</sup>                                                                       | x <sup>3</sup> y <sup>a</sup><br>(weight ratio) | -Y <sup>3</sup> -                                                                                                                                                                              |
|--------------------------------|-----------|-----------------------------------------------------------------------------------------------------------------|--------------------------------|---------------------------------------------------------------------------------------|-------------------------------------------------|------------------------------------------------------------------------------------------------------------------------------------------------------------------------------------------------|
| 24                             | A-24      | $\begin{array}{c} \text{O} \\ \text{H}-\text{P}-\text{OCH}_2\text{CH}_2\text{S}- \\   \\ \text{OH} \end{array}$ | -C <sub>2</sub> H <sub>5</sub> |    | 90/10                                           | $\begin{array}{c} \text{CH}_3 \\   \\ -\text{CH}_2-\text{C}- \\   \\ \text{COO}(\text{CH}_2)_2\text{OCO} \\   \\ \text{C}_6\text{H}_4 \\   \\ \text{C}-\text{O} \\    \\ \text{O} \end{array}$ |
| 25                             | A-25      | HO <sub>3</sub> SCH <sub>2</sub> CH <sub>2</sub> S -                                                            |                                |    | 93/7                                            | $\begin{array}{c} \text{CH}_3 \\   \\ -\text{CH}_2-\text{C}- \\   \\ * \end{array}$                                                                                                            |
| 26                             | A-26      | HOCH <sub>2</sub> CH <sub>2</sub> -S -                                                                          |                                |  | 92/8                                            | $\begin{array}{c} \text{CH}_3 \\   \\ -\text{CH}_2-\text{C}- \\   \\ \text{COO}(\text{CH}_2)_2\text{OCO}(\text{CH}_2)_2\text{COOH} \\   \\ * \end{array}$                                      |
| 27                             | A-27      | HOOC-(CH <sub>2</sub> ) <sub>2</sub> S -                                                                        |                                |  | 95/5                                            | $\begin{array}{c} \text{CH}_3 \\   \\ -\text{CH}_2-\text{C}- \\   \\ \text{COO}(\text{CH}_2)_3\text{SO}_3\text{H} \end{array}$                                                                 |

TABLE 4-continued

| Synthesis Example of Resin (A) | Resin (A) | W-                                                                                                                     | R <sup>35</sup>                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                                              | R <sup>36</sup> | x'/y <sup>a</sup><br>(weight ratio) | -Y <sup>3</sup> - |
|--------------------------------|-----------|------------------------------------------------------------------------------------------------------------------------|--------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|-----------------|-------------------------------------|-------------------|
| 28                             | A-28      | H <sub>5</sub> C <sub>2</sub> O- $\overset{\text{O}}{\underset{\text{OH}}{\text{P}}}(\text{OCH}_2\text{CH}_2\text{S}-$ | -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -  -CH <sub>2</sub> -<img alt="B |                 |                                     |                   |

SYNTHESIS EXAMPLE 29 OF RESIN (A):  
(A-29)

A mixed solution of 60 g of 2-chloro-6-methylphenyl methacrylate, 25 g of Macromonomer (M-4), 15 g of methyl acrylate, 150 g of toluene, and 50 g of isopropanol was heated to a temperature of 80° C. under nitrogen gas stream. After adding thereto 5 g of A.C.V., the reaction was carried out for 5 hours and, after further adding thereto 1.0 g of A.C.V., the reaction was carried out for 4 hours. The resulting copolymer had an Mw of  $9.8 \times 10^3$



25

SYNTHESIS EXAMPLE 101 OF  
MACROMONOMER: (M-101)

A mixed solution of 30 g of triphenylmethyl methacrylate and 100 g of toluene was sufficiently degassed under nitrogen gas stream and cooled to -20° C. Then, 1.0 g of 1,1-diphenylbutyl lithium was added to the mixture, and the reaction was conducted for 10 hours. Separately, a mixed solution of 70 g of ethyl methacrylate and 100 g of toluene was sufficiently degassed under nitrogen gas stream and the resulting mixed solution was added to the above described mixture, and then reaction was further conducted for 10 hours. The reaction mixture was adjusted to 0° C., and carbon dioxide gas was passed through the mixture at a flow rate of 60 ml/min for 30 minutes, then the polymerization reaction was terminated.

The temperature of the resulting reaction solution was raised to a temperature of 25° C. under stirring, 6 g of 2-hydroxyethyl methacrylate was added thereto, then a mixed solution of 12 g of dicyclohexylcarbodiimide, 1.0 g of 4-N,N-dimethylaminopyridine and 20 g of methylene chloride was added dropwise thereto over a period of 30 minutes, and the mixture was stirred for 3 hours.

After removing the precipitated insoluble substances from the reaction mixture by filtration, 10 ml of an ethanol solution of 30% by weight hydrogen chloride was added to the filtrate, and the mixture was stirred for one hour. Then, the solvent of the reaction mixture was distilled off under reduced pressure until the whole volume was reduced to a half, and the mixture was reprecipitated from one liter of petroleum ether. The precipitates thus formed were collected and dried under reduced pressure to obtain 56 g of the macromonomer having an Mw of  $6.5 \times 10^3$ .



5

SYNTHESIS EXAMPLE 102 OF  
MACROMONOMER: (M-102)

A mixed solution of 5 g of benzyl methacrylate, 0.1 g of (tetraphenyl porphynate) aluminum methyl and 60 g of methylene chloride was raised to a temperature of 30° C. under nitrogen gas stream. The mixture was irradiated with light from a xenon lamp of 300 W at a distance of 25 cm through a glass filter, and the reaction was conducted for 12 hours. To the mixture was further added 45 g of butyl methacrylate, after similarly light-irradiating for 8 hours, 10



25

g of 4-bromomethylstyrene was added to the reaction mixture followed by stirring for 30 minutes, then the reaction was terminated. Then, Pd-C was added to the reaction mixture, and a catalytic reduction reaction was conducted for one hour at a temperature of 25° C.

After removing insoluble substances from the reaction mixture by filtration, the reaction mixture was reprecipitated from 500 ml of petroleum ether, and the precipitates thus formed were collected and dried to obtain 33 g of the macromonomer having an Mw of  $7 \times 10^3$ .



40

SYNTHESIS EXAMPLE 103 OF  
MACROMONOMER: (M-103)

A mixed solution of 37.6 g of Monomer (II) having the structure shown below and 100 g of toluene was sufficiently degassed under nitrogen gas stream and cooled to 0° C. Then, 2 g of 1,1-diphenyl-3-methylpentyl lithium was added to the mixture followed by stirring for 6 hours. Separately, a mixed solution of 80 g of 2-chloro-6-methylphenyl methacrylate and 100 g of toluene was sufficiently degassed under nitrogen gas stream and the resulting mixed solution was added to the above described mixture, and then the reaction was further conducted for 8 hours. After introducing ethylene oxide at a flow rate of 30 ml/min into the reaction mixture for 30 minutes with vigorously stirring, the mixture was cooled to a temperature of 15° C., and 12 g of methacrylic acid chloride was added dropwise thereto over a period of 30 minutes, followed by stirring for 3 hours.

55

Then, to the reaction mixture was added 10 g of an ethanol solution of 30% by weight hydrogen chloride and, after stirring the mixture for one hour at 25° C., the mixture was

reprecipitated from one liter of petroleum ether. The precipitates thus formed were collected, washed twice with 300 ml of diethyl ether and dried to obtain 55 g of the macromonomer having an  $M_w$  of  $7.8 \times 10^3$ .



Monomer (II)



SYNTHESIS EXAMPLE 104 OF  
MACROMONOMER: (M-104)

A mixed solution of 40 g of triphenylmethyl acrylate and 100 g of toluene was sufficiently degassed under nitrogen gas stream and cooled to  $-20^\circ\text{C}$ . Then, 2 g of sec-butyl lithium was added to the mixture, and the reaction was conducted for 10 hours. Separately, a mixed solution of 60 g of styrene and 100 g of toluene was sufficiently degassed under nitrogen gas stream and the resulting mixed solution was added to the above described mixture, and then reaction was further conducted for 12 hours. The reaction mixture was adjusted to  $0^\circ\text{C}$ , 11 g of benzyl bromide was added thereto, and the reaction was conducted for one hour, followed by reacting at  $25^\circ\text{C}$ . for 2 hours.

Then, to the reaction mixture was added 10 g of an ethanol solution of 30% by weight hydrogen chloride, followed by stirring for 2 hours. After removing the insoluble substances from the reaction mixture by filtration, the mixture was reprecipitated from one liter of n-hexane. The precipitates thus formed were collected and dried under reduced pressure to obtain 58 g of the macromonomer having an  $M_w$  of  $4.5 \times 10^3$ .



SYNTHESIS EXAMPLE 105 OF  
MACROMONOMER: (M-105)

A mixed solution of 70 g of phenyl methacrylate and 4.8 g of benzyl N-hydroxyethyl-N-ethyldithiocarbamate was placed in a vessel under nitrogen gas stream followed by closing the vessel and heating to a temperature of  $60^\circ\text{C}$ . The mixture was irradiated with light from a high-pressure mercury lamp for 400 W at a distance of 10 cm through a glass filter for 10 hours to conduct a photopolymerization. Then, 30 g of acrylic acid and 180 g of methyl ethyl ketone were added to the mixture and, after replacing the gas in the vessel with nitrogen, the mixture was light-irradiated again for 10 hours.

45 To the resulting reaction mixture was added dropwise 12 g of 2-isocyanatoethyl methacrylate at a temperature of  $30^\circ\text{C}$ . over a period of one hour, and the mixture was stirred for 2 hours. The reaction mixture obtained was reprecipitated from 1.5 liters of hexane, and the precipitates thus formed were collected and dried to obtain 68 g of the macromonomer having an  $M_w$  of  $6.0 \times 10^3$ .



SYNTHESIS EXAMPLE 101 OF RESIN (A):  
(A-101)

A mixed solution of 80 g of ethyl methacrylate, 20 g of Macromonomer (M-101) and 150 g of toluene was heated at 5° C. under nitrogen gas stream, and 6 g of 2,2'-azobisis(isobutyronitrile) (A.I.B.N.) was added thereto to effect reaction for 3 hours. Then, 2 g of A.I.B.N. was further added thereto, followed by reacting for 2 hours, and thereafter 2 g of A.I.B.N. was added thereto, followed by 10° reacting for 2 hours. The resulting copolymer had an Mw of 9×10<sup>3</sup>.

SYNTHESIS EXAMPLE 102 OF RESIN (A):  
(A-102)

A mixed solution of 70 g of 2-chlorophenyl methacrylate, 30 g of Macromonomer (M-102), 2 g of n-dodecylmercaptan and 100 g of toluene was heated at a temperature of 80° C. under nitrogen gas stream, and 3 g of 2,2'-azobisis(isovaleronitrile) (A.I.V.N.) was added thereto to effect reaction for 3 hours. Then, 1 g of A.I.V.N. was further added, followed by reacting for 2 hours, and thereafter 1 g of 30° A.I.V.N. was added thereto, followed by heating to a temperature of 90° C. and reacting for 3 hours. The resulting copolymer had an Mw of 7.6×10<sup>3</sup>.



50

55

SYNTHESIS EXAMPLES 103 TO 118 OF RESIN  
(A): (A-103) to (A-118)

The copolymers shown in Table 5 below were synthesized 60 under the same polymerization conditions as described in Synthesis Example 101 of Resin (A) except for using the monomers shown in Table 5 below in place of the ethyl 65 methacrylate, respectively. The Mw of each of the copolymers obtained was in a range of from 5×10<sup>3</sup> to 9×10<sup>3</sup>.

TABLE 5



$$x + y + 20 = 100 \text{ (weight ratio)}$$

| Synthesis Example of Resin (A) | Resin (A) | -R                                                                                                     | -Y-                                                                                                              | x/y   |
|--------------------------------|-----------|--------------------------------------------------------------------------------------------------------|------------------------------------------------------------------------------------------------------------------|-------|
| 103                            | A-103     | $-\text{C}_4\text{H}_9$                                                                                | —                                                                                                                | 80/0  |
| 104                            | A-104     | $-\text{CH}_2\text{C}_6\text{H}_5$                                                                     | —                                                                                                                | 80/0  |
| 105                            | A-105     | $-\text{C}_6\text{H}_5$                                                                                | —                                                                                                                | 80/0  |
| 106                            | A-106     | $-\text{C}_4\text{H}_9$                                                                                | $-\text{CH}_2-\text{CH}-$<br>   | 65/15 |
| 107                            | A-107     | $-\text{CH}_2\text{C}_6\text{H}_5$                                                                     | $-\text{CH}_2-\text{CH}-$<br>   | 70/10 |
| 108                            | A-108     |                       | —                                                                                                                | 80/0  |
| 109                            | A-109     |                     | —                                                                                                                | 80/0  |
| 110                            | A-110     |                     | —                                                                                                                | 80/0  |
| 111                            | A-111     |                     | —                                                                                                                | 80/0  |
| 112                            | A-112     |                     | —                                                                                                                | 80/0  |
| 113                            | A-113     |                     | $-\text{CH}_2-\text{CH}-$<br> | 70/10 |
| 114                            | A-114     | $-\text{CH}_2-$<br> | —                                                                                                                | 80/0  |

TABLE 5-continued

| Synthesis Example of Resin (A) | Resin (A) | -R                                                                                      | -Y-                                                                                                                                                           | x/y                                                                                                                                                                                                                                                                                                                        |
|--------------------------------|-----------|-----------------------------------------------------------------------------------------|---------------------------------------------------------------------------------------------------------------------------------------------------------------|----------------------------------------------------------------------------------------------------------------------------------------------------------------------------------------------------------------------------------------------------------------------------------------------------------------------------|
| 115                            | A-115     | -CH <sub>3</sub>                                                                        | $  \begin{array}{c}  \text{CH}_3 \\    \\  -\text{CH}_2-\text{C}_x-\text{Y}_y-\text{CH}_2-\text{C}_{20} \\    \\  \text{COOR}  \end{array}  $                 | $  \begin{array}{c}  \text{CH}_3 \\    \\  \left[ \begin{array}{c} \text{CH}_3 & & \text{CH}_3 \\   & \text{b} &   \\ \text{C}_{70} & -\text{CH}_2-\text{C}_{30} \\   & &   \\ \text{COOC}_2\text{H}_5 & & \text{COOH} \end{array} \right] \\    \\  \text{x} + \text{y} + 20 = 100 \text{ (weight ratio)}  \end{array}  $ |
| 116                            | A-116     | -CH <sub>2</sub> C <sub>6</sub> H <sub>5</sub>                                          | $  \begin{array}{c}  \text{CH}_3 \\    \\  -\text{CH}_2-\text{C}_x-\text{Y}_y-\text{CH}_2-\text{C}_{20} \\    \\  \text{COO(CH}_2)_2\text{CN}  \end{array}  $ | 65/15                                                                                                                                                                                                                                                                                                                      |
| 117                            | A-117     | -C <sub>6</sub> H <sub>5</sub>                                                          | $  \begin{array}{c}  \text{CH}_3 \\    \\  -\text{CH}_2-\text{C}_x-\text{Y}_y-\text{CH}_2-\text{C}_{20} \\    \\  \text{CONH}_2  \end{array}  $               | 72/8                                                                                                                                                                                                                                                                                                                       |
| 118                            | A-118     | $  \begin{array}{c}  \text{Cl} \\    \\  \text{---} \\    \\  \text{Cl}  \end{array}  $ | —                                                                                                                                                             | 80/0                                                                                                                                                                                                                                                                                                                       |

SYNTHESIS EXAMPLES 119 TO 135 OF RESIN (A): (A-119) to (A-135)

The copolymers shown in Table 6 below were synthesized under the same polymerization conditions as described in

35

Synthesis Example 102 of Resin (A) except for using the macromonomers (M) shown in Table 6 below in place of Macromonomer (M-102), respectively. The Mw of each of the copolymers obtained was in a range of from  $2 \times 10^3$  to  $1 \times 10^4$ .

TABLE 6

| Synthesis Example of Resin (A) | Resin (A) | -X-                                                                                                          |                                    | a <sub>1</sub> /a <sub>2</sub> | -R                                                |                                   | -Z-                                     | x/y    |
|--------------------------------|-----------|--------------------------------------------------------------------------------------------------------------|------------------------------------|--------------------------------|---------------------------------------------------|-----------------------------------|-----------------------------------------|--------|
|                                |           | -COO(CH <sub>2</sub> ) <sub>2</sub> OOC-                                                                     | -H/-CH <sub>3</sub>                |                                | -COOCH <sub>3</sub>                               | -COOC <sub>6</sub> H <sub>5</sub> |                                         |        |
| 119                            | A-119     |                                                                                                              |                                    |                                |                                                   |                                   | -CH <sub>2</sub> -CH-                   | 7/0/30 |
|                                |           |                                                                                                              |                                    |                                |                                                   |                                   | COOH                                    |        |
| 120                            | A-120     | -COOCH <sub>2</sub> CH(OH)CH <sub>2</sub> OOC-                                                               | -CH <sub>3</sub> /-CH <sub>3</sub> |                                | -COOCH <sub>2</sub> C <sub>6</sub> H <sub>5</sub> |                                   | -CH <sub>2</sub> -CH-                   | 60/40  |
|                                |           |                                                                                                              |                                    |                                |                                                   |                                   | COOH                                    |        |
|                                |           |                                                                                                              |                                    |                                |                                                   |                                   | COO(CH <sub>2</sub> ) <sub>2</sub> COOH |        |
| 121                            | A-121     |                                                                                                              | -H/-CH <sub>3</sub>                |                                | -COOC <sub>6</sub> H <sub>5</sub>                 |                                   | -CH <sub>2</sub> -C-                    | 65/35  |
|                                |           |                                                                                                              |                                    |                                |                                                   |                                   | CH <sub>3</sub>                         |        |
| 122                            | A-122     | -COO(CH <sub>2</sub> ) <sub>2</sub> OCO(CH <sub>2</sub> ) <sub>2</sub> -COO(CH <sub>2</sub> ) <sub>2</sub> - | -CH <sub>3</sub> /-CH <sub>3</sub> |                                | -COOC <sub>2</sub> H <sub>5</sub>                 |                                   | -CH <sub>2</sub> -C-                    | 80/20  |
|                                |           |                                                                                                              |                                    |                                |                                                   |                                   | COOH                                    |        |
| 123                            | A-123     | -COOCH <sub>2</sub> CH <sub>2</sub> -                                                                        | -CH <sub>3</sub> /-H               |                                | -C <sub>6</sub> H <sub>5</sub>                    |                                   | -CH <sub>2</sub> -CH-                   | 50/50  |
|                                |           |                                                                                                              |                                    |                                |                                                   |                                   | COOH                                    |        |



TABLE 6-continued

| Synthesis Example of Resin (A) | Resin (A) | -X-                                                                                                                    |                                    |                                   | -R-                                                                                                    | -Z-                                                                                                    | x/y   |
|--------------------------------|-----------|------------------------------------------------------------------------------------------------------------------------|------------------------------------|-----------------------------------|--------------------------------------------------------------------------------------------------------|--------------------------------------------------------------------------------------------------------|-------|
|                                |           | a <sub>1</sub> /a <sub>2</sub>                                                                                         | -CH <sub>3</sub> /-CH <sub>3</sub> | -COOC <sub>2</sub> H <sub>5</sub> |                                                                                                        |                                                                                                        |       |
| 124                            | A-124     | -COOCH <sub>2</sub> CH(CH <sub>2</sub> OOCH <sub>2</sub> OH-                                                           | -CH <sub>3</sub> /-CH <sub>3</sub> | -COOC <sub>2</sub> H <sub>5</sub> | -CH <sub>3</sub>                                                                                       | -CH <sub>3</sub>                                                                                       | 90/10 |
| 125                            | A-125     | —  —CH <sub>2</sub> O—              | -H/-CH <sub>3</sub>                | -COOC <sub>3</sub> H <sub>7</sub> | -CH <sub>3</sub>                                                                                       | -CH <sub>3</sub>                                                                                       | 80/20 |
| 126                            | A-126     | —  —S—C <sub>2</sub> H <sub>5</sub> | -CH <sub>3</sub> /-CH <sub>3</sub> | -COOC <sub>2</sub> H <sub>5</sub> | -CH <sub>2</sub> —  | -CH <sub>2</sub> —  | 65/35 |
| 127                            | A-127     | "                                                                                                                      | -CH <sub>3</sub> /-H               | -COOC <sub>6</sub> H <sub>5</sub> | CH <sub>3</sub>                                                                                        | CH <sub>3</sub>                                                                                        | 70/30 |
| 128                            | A-128     | —                                 | -CH <sub>3</sub> /-CH <sub>3</sub> | "                                 | -CH <sub>2</sub> —  | -CH <sub>2</sub> —  | 75/25 |

TABLE 6-continued

| Synthesis Example of Resin (A) | Resin (A) | -X-                                      | a <sub>1</sub> /a <sub>2</sub> | -R                                 | -C <sub>6</sub> H <sub>5</sub>                    | -CH <sub>2</sub> -CH- | -Z-  | x/y   |
|--------------------------------|-----------|------------------------------------------|--------------------------------|------------------------------------|---------------------------------------------------|-----------------------|------|-------|
|                                |           |                                          |                                |                                    |                                                   |                       |      |       |
| 129                            | A-129     | -COOCH <sub>2</sub> CH <sub>2</sub> -    |                                | -CH <sub>3</sub> /H                | -CH <sub>3</sub>                                  | -CH <sub>2</sub> -CH- |      | 9/10  |
| 130                            | A-130     | CONHCOOCH <sub>2</sub> CH <sub>2</sub> - |                                | -CH <sub>3</sub> /-CH <sub>3</sub> | -COOCH <sub>2</sub> C <sub>6</sub> H <sub>5</sub> | -CH <sub>3</sub> /C-  |      | 70/30 |
| 131                            | A-131     |                                          |                                | -H/-CH <sub>3</sub>                | -COOC <sub>4</sub> H <sub>9</sub>                 | -CH <sub>3</sub> /C-  | COOH | 80/20 |
| 132                            | A-132     | -COO-                                    |                                | -CH <sub>3</sub> /-CH <sub>3</sub> | -COOCH <sub>3</sub>                               | -CH <sub>2</sub> -CH- | COOH | 70/30 |



TABLE 6-continued

| Synthesis Example of Resin (A) | Resin (A) | $-X-$                                                  | $a_1/a_2$ | $-CH_3/-CH_3$                                                                       | $-R$                                                                               | $-Z-$                                                                               | $xy$  |
|--------------------------------|-----------|--------------------------------------------------------|-----------|-------------------------------------------------------------------------------------|------------------------------------------------------------------------------------|-------------------------------------------------------------------------------------|-------|
| 133                            | A-133     | $-COO(CH_2)_3COOC-$                                    |           |   |  |    | 75/25 |
| 134                            | A-134     |                                                        |           |  | $-H/-H$                                                                            | $-C_6H_5$                                                                           | 70/30 |
| 135                            | A-135     | $\begin{array}{c}   \\ CONHC=S \\    \\ S \end{array}$ |           | $-H/-CH_3$                                                                          | $-COOCH_2C_6H_5$                                                                   |  | 85/15 |

Synthesis examples of the resin (B) are specifically illustrated below.

**SYNTHESIS EXAMPLE 1 OF RESIN (B): Resin (B-1)**

A mixed solution of 67 g of methyl methacrylate, 32 g of methyl acrylate, 1 g of acrylic acid, 17.5 g of Initiator (I-1) having the following structure and 150 g of tetrahydrofuran was heated to a temperature of 50° C. under nitrogen gas stream. The solution was irradiated with light from a high-pressure mercury lamp of 400 W at a distance of 10 cm through a glass filter for 10 hours to conduct photopolymerization. The reaction mixture obtained was reprecipitated in one liter of methanol, and the precipitates formed were collected and dried to obtain 72 g of the polymer having a weight average molecular weight (Mw) of  $5 \times 10^4$ .



**SYNTHESIS EXAMPLE 2 OF RESIN (B): Resin (B-2)**

Resin (B-2) was synthesized under the same condition as described in Synthesis Example 1 of Resin (B) except for using 10 g of Initiator (I-2) having the following structure in 40 place of 17.5 g of Initiator (I-1). The yield of the resulting polymer was 75 g and the Mw thereof was  $6 \times 10^4$ .



**SYNTHESIS EXAMPLES 3 TO 9 OF RESIN (B): Resins (B-3) to (B-9)**

Each of resins (B) shown in Table 7 below was synthesized under the same condition as described in Synthesis Example 1 of Resin (B) except for using a mixed solution of 65 g of methyl methacrylate, 30 g of methyl acrylate, 4 g of N-vinylpyrrolidone, 1 g of methacrylic acid, 0.0312 moles of each of Initiators shown in Table 7 below and 100 g of tetrahydrofuran. The Mw of each of the resulting polymers was in a range of from  $6 \times 10^4$  to  $8 \times 10^4$ .

**Initiator (I-1)**

**Resin (B-1)**

**Initiator (I-2)**

**Resin (B-2)**

TABLE 7

|                                                                                                                                                                                           |                                                                                              |                                                                                      |
|----------------------------------------------------------------------------------------------------------------------------------------------------------------------------------------------------------------------------------------------------------------------------|----------------------------------------------------------------------------------------------|--------------------------------------------------------------------------------------|
| $\text{+P: } \left[ \text{---CH}_2 \text{---C}_{65} \text{---CH}_2 \text{---CH}_{30} \text{---CH}_2 \text{---CH}_4 \text{---CH}_2 \text{---C}_{21} \text{---CH}_3 \right]_n \text{---R}$  |                                                                                              |                                                                                      |
| Synthesis Example<br>of Resin (B)                                                                                                                                                                                                                                          | Initiator (I)                                                                                | -R                                                                                   |
| 3                                                                                                                                                                                                                                                                          | <br>(I-3)   |    |
| 4                                                                                                                                                                                                                                                                          | <br>(I-4)  |    |
| 5                                                                                                                                                                                                                                                                          | <br>(I-5) |  |
| 6                                                                                                                                                                                                                                                                          | <br>(I-6) |  |
| 7                                                                                                                                                                                                                                                                          | <br>(I-7) |   |
| 8                                                                                                                                                                                                                                                                          | <br>(I-8) |  |
|                                                                                                                                                                                         |                                                                                              |                                                                                      |

TABLE 7-continued



## SYNTHESIS EXAMPLES 10 TO 15 OF RESIN (B): Resins (B-10) to (B-15)

30

Each of the resins (B) shown in Table 8 below was synthesized under the same condition as described in Synthesis Example 1 of Resin (B) except for using each of monomers corresponding to the polymer components shown in Table 8 below in place of methyl methacrylate, methyl acrylate and acrylic acid. The Mw of each of the resulting polymers was in a range of from  $5 \times 10^4$  to  $6 \times 10^4$ . 35

TABLE 8

| Synthesis Example | Resin (B) | +P+(weight ratio)                                                                                                                                                                                                                                                                                                                            |
|-------------------|-----------|----------------------------------------------------------------------------------------------------------------------------------------------------------------------------------------------------------------------------------------------------------------------------------------------------------------------------------------------|
| 10                | (B-10)    | $  \begin{array}{c}  \text{CH}_3 \quad \text{CH}_3 \\    \quad   \\  \text{CH}_2 - \text{C}_{68} - \text{CH}_2 - \text{CH}_{30} - \text{CH}_2 - \text{C}_{2} \\    \quad   \\  \text{COOCH}_3 \quad \text{COOCH}_3 \quad \text{COO}(\text{CH}_2)_2 \text{OCO}(\text{CH}_2)_2 \text{COOH}  \end{array}  $                                     |
| 11                | (B-11)    | $  \begin{array}{c}  \text{CH}_3 \quad \text{CH}_3 \\    \quad   \\  \text{CH}_2 - \text{C}_{79.2} - \text{CH}_2 - \text{CH}_{20} - \text{CH}_2 - \text{C}_{0.8} \\    \quad   \\  \text{COOCH}_3 \quad \text{COOC}_2\text{H}_5 \quad \text{COOH}  \end{array}  $                                                                            |
| 12                | (B-12)    | $  \begin{array}{c}  \text{CH}_3 \\    \\  \text{CH}_2 - \text{C}_{82.5} - \text{CH}_2 - \text{CH}_{15} - \text{CH}_2 - \text{C}_{2.5} \\    \quad   \quad   \\  \text{COOCH}_3 \quad \text{COOCH}_3 \quad \text{O}=\text{C} \\  \quad \quad \quad \backslash \quad / \\  \quad \quad \quad \text{O} \quad \text{C}=\text{O}  \end{array}  $ |

TABLE 8-continued

| Synthesis Example | of Resin (B) | Resin (B) | + P+ (weight ratio) |  |                                                                                                                                                                                                                                                                                                                                                                                                                             |
|-------------------|--------------|-----------|---------------------|-----------------------------------------------------------------------------------|--------------------------------------------------------------------------------------------------------------------------------------------------------------------------------------------------------------------------------------------------------------------------------------------------------------------------------------------------------------------------------------------------------------------------------------------------------------------------------------------------------------|
| 13                | (B-13)       |           |                     |  | $+ \left( \text{CH}_2 - \underset{\substack{  \\ \text{COOC}_2\text{H}_5}}{\text{C}} \text{--} \text{CH}_2 \right)_{17} \left( \text{CH}_2 - \underset{\substack{  \\ \text{COOCH}_3}}{\text{CH}} \text{--} \text{CH}_2 \right)_{20} \left( \text{CH}_2 - \underset{\substack{  \\ \text{COOCH}_3}}{\text{CH}} \text{--} \text{CH}_2 \right)_{17}$                                                                                                                                                           |
| 14                | (B-14)       |           |                     |  | $+ \left( \text{CH}_2 - \underset{\substack{  \\ \text{COOCH}_3}}{\text{C}} \text{--} \text{CH}_2 \right)_{66} \left( \text{CH}_2 - \underset{\substack{  \\ \text{COOCH}_3}}{\text{CH}} \text{--} \text{CH}_2 \right)_{30} \left( \text{CH}_2 - \underset{\substack{  \\ \text{CN}}}{\text{CH}} \text{--} \text{CH}_2 \right)_{2,5} \left( \text{CH}_2 - \underset{\substack{  \\ \text{COO}(\text{CH}_2)_2\text{COOH}}}{\text{CH}} \text{--} \text{CH}_2 \right)_{1,5}$                                    |
| 15                | (B-15)       |           |                     |  | $+ \left( \text{CH}_2 - \underset{\substack{  \\ \text{COOCH}_3}}{\text{C}} \text{--} \text{CH}_2 \right)_{30} \left( \text{CH}_2 - \underset{\substack{  \\ \text{COO}(\text{CH}_2)_2\text{OCH}_3}}{\text{C}} \text{--} \text{CH}_2 \right)_8 \left( \text{CH}_2 - \underset{\substack{  \\ \text{COO}(\text{CH}_2)_2\text{O}}}{\text{CH}} \text{--} \text{CH}_2 \right)_2 \left( \text{CH}_2 - \underset{\substack{  \\ \text{O} \\ \text{P} \\   \\ \text{OH}}}{\text{CH}} \text{--} \text{CH}_2 \right)$ |

## SYNTHESIS EXAMPLES 16 TO 19 OF RESIN (B): Resins (B-16) to (B-19)

(B): Resins (B-16) to (B-19)

Each of resins (B) shown in Table 9 below was synthesized under the same condition as described in Synthesis

35 Example 1 of Resin (B) except for using a mixed solution of 71.5 g of methyl methacrylate, 25 g of methyl acrylate, 2.5 g of acrylonitrile, 1 g of acrylic acid, 0.0315 moles of Initiator shown in Table 9 below and 100 g of tetrahydrofuran. The Mw of each of the resulting polymers was in a range of from  $5 \times 10^4$  to  $8 \times 10^4$ .

40

45

50

60

65

TABLE 9

| Synthesis<br>Example of<br>Resin (B) | Resin (B) | [P]                                                                                                                             |                                                                                                                                    | [P]                                                                                                                  |                                                                                              |
|--------------------------------------|-----------|---------------------------------------------------------------------------------------------------------------------------------|------------------------------------------------------------------------------------------------------------------------------------|----------------------------------------------------------------------------------------------------------------------|----------------------------------------------------------------------------------------------|
|                                      |           | Initiator (I)                                                                                                                   | —R                                                                                                                                 | Initiator (I)                                                                                                        | —R                                                                                           |
| 16                                   | (B-16)    | $(\text{CH}_2)_3\text{R}$<br>$\text{R} \leftarrow (\text{CH}_2)_3\text{Si}(\text{CH}_2)_3\text{R}$<br>$(\text{CH}_2)_3\text{R}$ | $-\text{S}-\overset{\text{C}_4\text{H}_9}{\underset{\text{S}}{\text{C}}}-\text{O}-\text{C}_4\text{H}_9$                            | $(\text{CH}_2)_3\text{R}$<br>$\leftarrow (\text{CH}_2)_3\text{Si}(\text{CH}_2)_3-$<br>$(\text{CH}_2)_3-$             |                                                                                              |
| 17                                   | (B-17)    | $\text{CONH}(\text{CH}_2)_3\text{R}$<br>$\text{R} \leftarrow (\text{CH}_2)_3\text{NHCO}$                                        | $-\text{S}-\overset{\text{C}_4\text{H}_9}{\underset{\text{S}}{\text{C}}}-\text{N}-\text{C}_4\text{H}_9$                            | $\text{CONH}(\text{CH}_2)_3\text{R}$<br>$\text{CONH}(\text{CH}_2)_3\text{R}$<br>$\text{CONH}(\text{CH}_2)_3\text{R}$ | $\leftarrow (\text{CH}_2)_3\text{NHCO}$<br>$\text{CONH}(\text{CH}_2)_3\text{R}$              |
| 18                                   | (B-18)    | $\text{COO}(\text{CH}_2)_2\text{R}$<br>$\text{R}(\text{CH}_2)_2\text{OOC}$                                                      | $-\text{S}-\overset{\text{CH}_3}{\underset{\text{S}}{\text{C}}}-\text{O}-\overset{\text{CH}_3}{\underset{\text{CH}_3}{\text{C}}}-$ | $\text{COO}(\text{CH}_2)_2-$<br>$-(\text{CH}_2)_2\text{OOC}$<br>$\text{COO}(\text{CH}_2)_2-$                         | $\text{COO}(\text{CH}_2)_2-$<br>$-(\text{CH}_2)_2\text{OOC}$<br>$\text{COO}(\text{CH}_2)_2-$ |

TABLE 9-continued

| Synthesis Example of Resin (B) | Resin (B)      | Initiator (I)  | $-R$               | $-R$               | $-R$           | $-R$           |
|--------------------------------|----------------|----------------|--------------------|--------------------|----------------|----------------|
| 19 (B-19)                      | $R(CH_2)_2OOC$ | $COO(CH_2)_2R$ | $-S-C(=O)CH_2CH_3$ | $-S-C(=O)CH_2CH_3$ | $COO(CH_2)_2-$ | $COO(CH_2)_2-$ |

SYNTHESIS EXAMPLES 20 TO 24 OF RESIN  
(B): Resins (B-20) to (B-24)

A mixture of 11.3 g of Initiator (I-2) described above and monomers corresponding to the polymer components shown in Table 10 below was heated to a temperature of 40° C. under nitrogen gas stream, followed by light irradiation for polymerization in the same manner as described in Synthesis Example 1 of Resin (B). The solid material obtained was collected, dissolved in 250 ml of tetrahydrofuran, reprecipitated in 1.5 liters of methanol, and the precipitates formed were collected by filtration and dried. The yield of each of the resulting polymers was in a range of from 60 to 75 g and the  $M_w$  thereof was in a range of from  $6 \times 10^4$  to  $8 \times 10^4$ .

mercury lamp of 400 W at a distance of 10 cm through a glass filter for 5 hours to conduct photopolymerization.



10 The resulting polymer was dissolved by adding 100 g of tetrahydrofuran, then 25 g of methyl acrylate and 1.0 g of acrylic acid were added thereto, and the mixture was again heated to a temperature of 50° C. under nitrogen gas stream.

TABLE 10

| Synthesis Example of Resin (B) | Resin (B) | $+P+$ (weight ratio)                                                                 |
|--------------------------------|-----------|--------------------------------------------------------------------------------------|
| 20                             | (B-20)    |    |
| 21                             | (B-21)    |   |
| 22                             | (B-22)    |  |
| 23                             | (B-23)    |  |
| 24                             | (B-24)    |  |

SYNTHESIS EXAMPLE 101 OF RESIN (B):  
Resin (B-101)

A mixture of 74 g of methyl methacrylate and 12.4 g of Initiator (I-1) having the following structure was heated to a temperature of 50° C. under nitrogen gas stream. The solution was irradiated with light from a high-pressure

60 The mixture was irradiated with light in the same manner as above for 10 hours, the reaction mixture obtained was reprecipitated in 2 liters of methanol, and the precipitates formed were collected and dried. The yield of the resulting polymer was 78 g and the weight average molecular weight ( $M_w$ ) thereof was  $6 \times 10^4$ .



wherein  $-b-$  represents a bond between blocks (hereinafter the same).

**SYNTHESIS EXAMPLE 102 OF RESIN (B):  
Resin (B-102)**

Resin (B-102) was synthesized under the same condition as described in Synthesis Example 101 of Resin (B) except for using 16.0 g of Initiator (I-2) having the following structure in place of 12.4 g of Initiator (I-1). The yield of the resulting polymer was 72 g and the Mw thereof was  $6 \times 10^4$ .

15 drofuran, then 30 g of methyl acrylate, 4 g of N-vinylpyrrolidone and 1 g of methacrylic acid were added thereto, and the mixture was subjected to photopolymerization and precipitation in the same manner as described in Synthesis Example 101 of Resin (B). The Mw of each of the resulting polymers was in a range of  $5 \times 10^4$  to  $8 \times 10^4$ .



**SYNTHESIS EXAMPLES 103 TO 109 OF RESIN (B): Resins (B-103) to (B-109)**

A mixture of 65 g of methyl methacrylate and 0.013 moles of each of Initiators shown in Table 11 below was subjected to a photopolymerization reaction in the same manner as described in Synthesis Example 101 of Resin (B). The resulting polymer was dissolved by adding 100 g of tetrahy-

TABLE 11



## SYNTHESIS EXAMPLES 110 TO 115 OF RESIN (B.): Resins (B-110) to (S-115)

Each of resins (B) shown in Table 12 below was synthesized under the same condition as described in Synthesis Example 101 of Resin (B) except for using each of monomers corresponding to the polymer components shown in

65 Table 12 below in place of methyl methacrylate, methyl acrylate and acrylic acid. The Mw of each of the resulting polymers was in a range of from  $5 \times 10^4$  to  $6 \times 10^4$ .

TABLE 12

| Synthesis Example of Resin (B) | Resin (B) | +P+ (weight ratio)  |                      |
|--------------------------------|-----------|---------------------|----------------------|
|                                |           | R+P+CH <sub>2</sub> | CH <sub>2</sub> +P+R |
| 110                            | (B-110)   |                     |                      |
| 111                            | (B-111)   |                     |                      |
| 112                            | (B-112)   |                     |                      |
| 113                            | (B-113)   |                     |                      |
| 114                            | (B-114)   |                     |                      |
| 115                            | (B-115)   |                     |                      |

**SYNTHESIS EXAMPLES 116 TO 121 OF RESIN (B): Resins (B-116) to (A-121)**

A mixed solution of 16.5 g of methyl acrylate, 2.5 g of acrylonitrile, 1.0 g of acrylic acid, 0.0072 moles of Initiator shown in Table 13 below and 20 g of tetrahydrofuran was subjected to light irradiation for 15 hours in the same manner as described in Synthesis Example 101 of Resin (B).

To the reaction mixture were added 60 g of methyl methacrylate, 20 g of methyl acrylate and 80 g of tetrahydrofuran, followed by polymerization reaction and reprecipitation in the same manner as described in Synthesis Example 101 of Resin (B). The Mw of each of the resulting polymers was in a range of from  $5 \times 10^4$  to  $8 \times 10^4$ .

TABLE 13

| Synthesis Example of Resin (B) | Resin (B) | [P]                                                                               |                                                                          | [P]                            |                                                                          | 5,580,690 |
|--------------------------------|-----------|-----------------------------------------------------------------------------------|--------------------------------------------------------------------------|--------------------------------|--------------------------------------------------------------------------|-----------|
|                                |           | X                                                                                 | Initiator                                                                | -R                             | -R                                                                       |           |
| 116                            | (B-116)   |  | $(CH_2)_3R$<br>$R \leftarrow CH_2 - Si - CH_2)_3R$<br>$(CH_2)_3R$        | $-S-C(=O)-CH_9$<br>$S$         | $(CH_2)_3 -$<br>$\leftarrow CH_2 - Si - CH_2)_3 -$<br>$(CH_2)_3 -$       | 107       |
| 117                            | (B-117)   |  | $CONH(CH_2)_3R$<br>$CONH(CH_2)_3R$<br>$CONH(CH_2)_3R$<br>$CONH(CH_2)_3R$ | $-S-C(=O)-N(C_4H_9)_2$<br>$S$  | $CONH(CH_2)_3$<br>$CONH(CH_2)_3$<br>$CONH(CH_2)_3$<br>$CONH(CH_2)_3$     | 108       |
| 118                            | (B-118)   |  | $COO(CH_2)_2R$<br>$COO(CH_2)_2R$<br>$COO(CH_2)_2R$<br>$COO(CH_2)_2R$     | $-S-C(=O)-O-CH(CH_3)_2$<br>$S$ | $COO(CH_2)_2 -$<br>$COO(CH_2)_2 -$<br>$COO(CH_2)_2 -$<br>$COO(CH_2)_2 -$ |           |
| 119                            | (B-119)   |  | $R(CH_2)_2OOC$<br>$R(CH_2)_2OOC$<br>$R(CH_2)_2OOC$<br>$R(CH_2)_2OOC$     | $-S-C(=O)-OC_4H_9$<br>$S$      | $-(CH_2)_2OOC$<br>$-(CH_2)_2OOC$<br>$-(CH_2)_2OOC$<br>$-(CH_2)_2OOC$     |           |

TABLE 13-continued

| Synthesis Example of Resin (B) | Resin (B) | Initiator                                                                                        | -R                                                                                  |                                                                                                                                  |
|--------------------------------|-----------|--------------------------------------------------------------------------------------------------|-------------------------------------------------------------------------------------|----------------------------------------------------------------------------------------------------------------------------------|
| 120                            | (B-120)   | $\begin{array}{c} R(CH_2)_2 \\   \\ NCO(CH_2)_3CON \\   \\ (CH_2)_2R \end{array}$                | $\begin{array}{c} (CH_2)_2R \\   \\ -S-C=O-OCH \\    \\ S \\   \\ CH_3 \end{array}$ | $\begin{array}{c} CH_3 \\   \\ -CH_2 \\   \\ NCO(CH_2)_3CON \\   \\ (CH_2)_2 \\   \\ -CH_2 \\   \\ CON[(CH_2)_2R]_2 \end{array}$ |
| 121                            | (B-121)   | $\begin{array}{c} CON[(CH_2)_2R]_2 \\   \\ \text{Benzene ring} \\   \\ R(CH_2)_2NOC \end{array}$ | $\begin{array}{c} CH_3 \\   \\ -S-C=O-N \\    \\ S \\   \\ CH_3 \end{array}$        | $\begin{array}{c} CH_3 \\   \\ -CH_2 \\   \\ CON[(CH_2)_2R]_2 \\   \\ + (CH_2)_2NOC \\   \\ CON[(CH_2)_2R]_2 \end{array}$        |



121

## 111

SYNTHESIS EXAMPLES 122 TO 126 OF RESIN  
(B): Resins (B-122) to (B-126)

A mixture of monomers corresponding to the polymer components shown in Table 14 below and 14 g of Initiator (I-2) described above was heated to a temperature of 40° C. under nitrogen gas stream, followed by light irradiation in the same manner as described in Synthesis Example 101 of Resin (B) to conduct polymerization for 5 hours. The solid material obtained was collected, dissolved in 100 g of tetrahydrofuran, and then 35 g of methyl acrylate and 1.5 g of acrylic acid were added thereto. The mixture was heated to a temperature of 50° C. under nitrogen gas stream and polymerized by irradiation with light in the same manner as above. The reaction mixture obtained was reprecipitated in one liter of methanol, and the precipitates formed were collected and dried. The yield of each of the resulting polymers was in a range of from 65 to 75 g and the Mw thereof was in a range of from  $5 \times 10^4$  to  $7 \times 10^4$ . 20

## 112

SYNTHESIS EXAMPLES 127 TO 133 OF RESIN  
(B): Resins (B-127) to (B-133)

A mixed solution of 56 g of methyl methacrylate, 24 g of methyl acrylate and 10 g of Initiator (I-3) having the following structure was heated to a temperature of 40° C. under nitrogen gas stream, followed by light irradiation in the same manner as described in Synthesis Example 101 of Resin (B) to conduct polymerization for 4 hours. The solid material obtained was dissolved in 100 g of tetrahydrofuran, and monomers corresponding to the polymer components shown in Table 15 below were added thereto. The mixture was heated to a temperature of 50° C. under nitrogen gas stream and polymerized by irradiation with light in the same manner as above. The reaction mixture obtained was reprecipitated in one liter of methanol, and the precipitates formed were collected and dried. The yield of each of the resulting polymers was in a range of from 65 to 75 g and the Mw thereof was in a range of from  $4 \times 10^4$  to  $7 \times 10^4$ . 15

TABLE 14

| Synthesis Example<br>of Resin (B) | Resin (B) | Polymer Component of Block $+X+$ (weight ratio)                                                                                                                                                                                                                                                                                                                                                                                                                                                                                                                                                                                             |
|-----------------------------------|-----------|---------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| 122                               | (B-122)   | $  \begin{array}{c}  \text{CH}_2 + \text{P} + \text{R} \\    \\  \text{R} + \text{P} + \text{H}_2\text{C} \\    \\  \text{CH}_2 + \text{P} + \text{R} \\    \\  \text{CH}_2 + \text{P} + \text{R}  \end{array}  \quad  \begin{array}{c}  \text{CH}_2 + \text{P} + \text{R} \\    \\  \text{R: } -\text{S}-\text{C}(=\text{S})-\text{N} \\    \\  \text{CH}_3 \\    \\  \text{CH}_3  \end{array}  $ $  + \text{P: } +\text{X}_{163.5}^b - \left( \begin{array}{c} \text{CH}_2 - \text{CH} \\   \\ \text{COOCH}_3 \end{array} \right)_{35} \left( \begin{array}{c} \text{CH}_2 - \text{CH} \\   \\ \text{COOH} \end{array} \right)_{15} -   $ |
| 123                               | (B-123)   | $  \begin{array}{c}  \text{CH}_3 \\    \\  \text{CH}_2 - \text{C}_{163.5}^b - \text{CH}_2 - \text{CH} \\    \quad   \\  \text{COOCH}_3 \quad \text{COOC}_2\text{H}_5  \end{array}  $                                                                                                                                                                                                                                                                                                                                                                                                                                                        |
| 124                               | (B-124)   | $  \begin{array}{c}  \text{CH}_3 \quad \text{CH}_3 \\    \quad   \\  \text{CH}_2 - \text{C}_{163.5}^b - \text{CH}_2 - \text{C}_{20}^b \\    \quad   \\  \text{COOCH}_2\text{C}_6\text{H}_5 \quad \text{COOCH}_3  \end{array}  $                                                                                                                                                                                                                                                                                                                                                                                                             |
| 125                               | (B-125)   | $  \begin{array}{c}  \text{CH}_3 \\    \\  \text{CH}_2 - \text{C}_{163.5}^b - \text{CH}_2 - \text{CH} \\    \quad   \\  \text{COOC}_2\text{H}_5 \quad \text{C}_6\text{H}_5  \end{array}  $                                                                                                                                                                                                                                                                                                                                                                                                                                                  |
| 126                               | (B-126)   | $  \begin{array}{c}  \text{CH}_3 \\    \\  \text{CH}_2 - \text{C}_{163.5}^b - \text{CH}_2 - \text{CH} \\    \quad   \\  \text{COOC}_6\text{H}_5 \quad \text{COOCH}_3  \end{array}  $                                                                                                                                                                                                                                                                                                                                                                                                                                                        |



Initiator (I-3)

TABLE 15

| Synthesis Example<br>of Resin (B) | Resin (B) | Polymer Component of Block $+X+$ (weight ratio) |  |  |
|-----------------------------------|-----------|-------------------------------------------------|--|--|
|                                   |           |                                                 |  |  |
| 127                               | (B-127)   |                                                 |  |  |
| 128                               | (B-128)   |                                                 |  |  |
| 129                               | (B-129)   |                                                 |  |  |
| 130                               | (B-130)   |                                                 |  |  |
| 131                               | (B-131)   |                                                 |  |  |
| 132                               | (B-132)   |                                                 |  |  |
| 133                               | (B-133)   |                                                 |  |  |

## SYNTHESIS EXAMPLE 201 OF RESIN (B):

## Resin (B-201)

A mixture of 74 g of methyl methacrylate and 12.4 g of Initiator (I-201) having the following structure was heated to a temperature of 50° C. under nitrogen gas stream. The solution was irradiated with light from a high-pressure mercury lamp of 400 W at a distance of 10 cm through a glass filter for 5 hours to conduct photopolymerization.



Initiator (I-201)

The resulting polymer was dissolved by adding 100 g of tetrahydrofuran, then 25 g of methyl acrylate and 1.0 g of acrylic acid were added thereto, and the mixture was again heated to a temperature of 50° C. under nitrogen gas stream.

The mixture was irradiated with light in the same manner as above for 10 hours, the reaction mixture obtained was reprecipitated in 2 liters of methanol, and the precipitates formed were collected and dried. The yield of the resulting polymer was 78 g and the weight average molecular weight (Mw) thereof was  $6 \times 10^4$ .



wherein -b- represents a bond between blocks (hereinafter 20 the same).

**SYNTHESIS EXAMPLE 202 OF RESIN (B):  
Resin (B-202)**

A mixture of 50.3 g of methyl methacrylate, 24.7 g of 25 methyl acrylate, 8.0 g of Initiator (I-202) having the following structure and 75 g of tetrahydrofuran was heated to a temperature of 50° C. under nitrogen gas stream. The solution was irradiated with light for 6 hours under the same 30 condition as described in Synthesis Example 201 of Resin (B).



To the resulting polymer was added a mixed solution of 40 23 g of methyl methacrylate, 2.0 g of acrylonitrile and 25 g of tetrahydrofuran, and the mixture was again heated to a temperature of 60° C. under nitrogen gas stream and irradiated with light for 12 hours in the same manner as above 45 to conduct photopolymerization. The reaction mixture obtained was reprecipitated in 1.5 liters of methanol, and the precipitates formed were collected and dried. The yield of the resulting polymer was 75 g and the Mw thereof was  $1.2 \times 10^5$ .

**Resin (B-202)**



**SYNTHESIS EXAMPLES 203 TO 210 OF RESIN  
(B): Resins (B-203) to (B-210)**

A mixture of 65 g of methyl methacrylate and 0.008 moles 5 of each of Initiators shown in Table 16 below was subjected to a photopolymerization reaction in the same manner as

**Resin (B-201)**

described in Synthesis Example 201 of Resin (B). The resulting polymer was dissolved by adding 100 g of tetrahydrofuran, then 32.2 g of methyl acrylate, 2.0 g of N-vinylpyrrolidone and 0.8 g of methacrylic acid were added thereto, and the mixture was subjected to photopolymerization and reprecipitation in the same manner as described in Synthesis Example 201 of Resin (B). The Mw of each of the resulting polymers was in a range of from  $8 \times 10^4$  to  $1.0 \times 10^5$ .

TABLE 16

| Synthesis Example<br>of Resin (B) | Initiator (I)                                                                  | -R                                                                            |                                                                      |
|-----------------------------------|--------------------------------------------------------------------------------|-------------------------------------------------------------------------------|----------------------------------------------------------------------|
|                                   |                                                                                | -S-C(=O)(CH <sub>2</sub> ) <sub>6</sub> COOH                                  | -CH <sub>2</sub> -                                                   |
| 203                               | CH <sub>2</sub> -R                                                             | -S-C(=O)S-                                                                    | -CH <sub>2</sub> -                                                   |
|                                   | 4-CH <sub>2</sub> -C <sub>6</sub> H <sub>4</sub> -CH <sub>2</sub> -R (I-203)   |                                                                               |                                                                      |
| 204                               | R-CH <sub>2</sub> -CH(R)-CH <sub>2</sub> -R (I-204)                            | -S-C(=O)N(CH <sub>3</sub> ) <sub>3</sub> COOH                                 | -CH <sub>2</sub> -CH-CH <sub>2</sub> -                               |
|                                   |                                                                                |                                                                               |                                                                      |
| 205                               | R-H <sub>2</sub> C-N(CH <sub>2</sub> R) <sub>2</sub> CH <sub>2</sub> R (I-205) | -S-C(=O)N(CH <sub>3</sub> ) <sub>3</sub> (CH <sub>2</sub> ) <sub>2</sub> COOH | -H <sub>2</sub> C-N(CH <sub>3</sub> ) <sub>3</sub> CH <sub>2</sub> - |
| 206                               | R-CH <sub>2</sub> -CH(R)-CH <sub>2</sub> -R (I-206)                            | -S-C(=O)N(CH <sub>3</sub> ) <sub>3</sub> (CH <sub>2</sub> ) <sub>4</sub> COOH | -CH <sub>2</sub> -CH-CH <sub>2</sub> -                               |

TABLE 16-continued

| Synthesis Example<br>of Resin (B) | Initiator (I)                                                                                                                                                                                                                                                                                                             | —R                                                                                                                                                                                                                                                                                                                |
|-----------------------------------|---------------------------------------------------------------------------------------------------------------------------------------------------------------------------------------------------------------------------------------------------------------------------------------------------------------------------|-------------------------------------------------------------------------------------------------------------------------------------------------------------------------------------------------------------------------------------------------------------------------------------------------------------------|
|                                   |                                                                                                                                                                                                                                                                                                                           | —CH <sub>2</sub> <sub>2</sub> COOH                                                                                                                                                                                                                                                                                |
| 207                               | $\begin{array}{c} \text{S} \\    \\ \text{CH}_2\text{O}-\text{C}-\text{S}-\text{R} \\   \\ \text{C}_2\text{H}_5-\text{C}-\text{O}-\text{C}-\text{S}-\text{R} \\   \\ \text{S} \end{array}$ $(I-207)$ $\begin{array}{c} \text{S} \\    \\ \text{CH}_2\text{O}-\text{C}-\text{S}-\text{R} \\   \\ \text{S} \end{array}$     | $\begin{array}{c} \text{S} \\    \\ \text{CH}_2\text{O}-\text{C}-\text{S}-\text{R} \\   \\ \text{C}_2\text{H}_5-\text{C}-\text{O}-\text{C}-\text{S}-\text{R} \\   \\ \text{S} \end{array}$ $\begin{array}{c} \text{S} \\    \\ \text{CH}_2\text{O}-\text{C}-\text{S}-\text{R} \\   \\ \text{S} \end{array}$       |
| 208                               |                                                                                                                                                                                                                                                                                                                           | $\begin{array}{c} \text{S} \\    \\ \text{CH}_2\text{O}-\text{C}-\text{S}-\text{R} \\   \\ \text{R}-\text{S}-\text{COCH}_2 \end{array}$ $(I-208)$                                                                                                                                                                 |
| 209                               | $\begin{array}{c} (\text{CH}_2)_2\text{OC}-\text{S}-\text{R} \\   \\ \text{S} \end{array}$ $\begin{array}{c} \text{H}_5\text{C}_2-\text{Si}+(\text{CH}_2)_3\text{OC}-\text{S}-\text{R} \\   \\ \text{S} \end{array}$ $\begin{array}{c} \text{R}-\text{S}-\text{CO}(\text{CH}_2)_3 \\   \\ \text{S} \end{array}$ $(I-209)$ | $\begin{array}{c} (\text{CH}_2)_3\text{O}-\text{C}-\text{S} \\   \\ \text{S} \end{array}$ $\begin{array}{c} \text{H}_5\text{C}_2-\text{Si} \\   \\ \text{S} \end{array}$ $-\text{S}-\text{CO}(\text{CH}_2)_3$ $\begin{array}{c} (\text{CH}_2)_3\text{O}-\text{C}-\text{S} \\   \\ \text{S} \end{array}$ $(I-208)$ |



TABLE 16-continued

| Synthesis Example<br>of I Resin (B) | Initiator (I)                                                                                                | -R                                                                                                                                                                                                                                                                                              |
|-------------------------------------|--------------------------------------------------------------------------------------------------------------|-------------------------------------------------------------------------------------------------------------------------------------------------------------------------------------------------------------------------------------------------------------------------------------------------|
| 210                                 | $\begin{array}{c} \text{R} \\   \\ \text{R}-\text{CH}_2\text{CHCH}_2-\text{R} \\ (\text{I-210}) \end{array}$ | $\begin{array}{c} \text{C}_2\text{H}_5 \\   \\ -\text{S}-\text{C}-\text{N} \\    \\ \text{S} \end{array}$ $\begin{array}{c} \text{OH} \\   \\ (\text{CH}_2)_2\text{O}-\text{P}-\text{OH} \\    \\ \text{O} \end{array}$ $\begin{array}{c}   \\ -\text{CH}_2-\text{CH}-\text{CH}_2- \end{array}$ |

SYNTHESIS EXAMPLES 211 TO 216 OF RESIN  
(B): Resins (B-211) to (B-216).

Each of resins (B) shown in Table 17 below was synthesized under the same condition as described in Synthesis Example 201 of Resin (B) except for using each of monomers corresponding to the polymer components shown in Table 17 below in place of methyl methacrylate, methyl acrylate and acrylic acid. The Mw of each of the resulting polymers was in a range of from  $5 \times 10^4$  to  $6 \times 10^4$ .

TABLE 17

| Synthesis Example<br>of Resin (B) | Resin (B) | $\text{+P+}$ (weight ratio) |                                                                                                                                                 |                                                                                                                                                                 |
|-----------------------------------|-----------|-----------------------------|-------------------------------------------------------------------------------------------------------------------------------------------------|-----------------------------------------------------------------------------------------------------------------------------------------------------------------|
|                                   |           |                             | $\text{CH}_2-\text{C}_6\text{H}_4-\text{CH}_2-\text{CH}_2-\text{CH}_2-\text{P}(=\text{O})(\text{R}')-\text{R}$                                  | $\text{CH}_2-\text{C}_6\text{H}_4-\text{CH}_2-\text{CH}_2-\text{CH}_2-\text{S}-\text{C}(=\text{S})-\text{N}(\text{C}_2\text{H}_5)-(\text{CH}_2)_2\text{COOH}$   |
| 211                               | (B-211)   |                             | $\text{--CH}_2-\text{C}_6\text{H}_4-\text{CH}_2-\text{CH}_2-\text{CH}_2-\text{P}(=\text{O})(\text{CH}_2)_2\text{OCO}(\text{CH}_2)_2\text{COOH}$ | $\text{--CH}_2-\text{C}_6\text{H}_4-\text{CH}_2-\text{CH}_2-\text{CH}_2-\text{S}-\text{C}(=\text{S})-\text{N}(\text{C}_2\text{H}_5)-(\text{CH}_2)_2\text{COOH}$ |
| 212                               | (B-212)   |                             | $\text{--CH}_2-\text{C}_6\text{H}_4-\text{CH}_2-\text{CH}_2-\text{CH}_2-\text{P}(=\text{O})(\text{CH}_2)_2\text{OCO}(\text{CH}_2)_2\text{COOH}$ | $\text{--CH}_2-\text{C}_6\text{H}_4-\text{CH}_2-\text{CH}_2-\text{CH}_2-\text{S}-\text{C}(=\text{S})-\text{N}(\text{C}_2\text{H}_5)-(\text{CH}_2)_2\text{COOH}$ |
| 213                               | (B-213)   |                             | $\text{--CH}_2-\text{C}_6\text{H}_4-\text{CH}_2-\text{CH}_2-\text{CH}_2-\text{P}(=\text{O})(\text{CH}_2)_2\text{OCO}(\text{CH}_2)_2\text{COOH}$ | $\text{--CH}_2-\text{C}_6\text{H}_4-\text{CH}_2-\text{CH}_2-\text{CH}_2-\text{S}-\text{C}(=\text{S})-\text{N}(\text{C}_2\text{H}_5)-(\text{CH}_2)_2\text{COOH}$ |
| 214                               | (B-214)   |                             | $\text{--CH}_2-\text{C}_6\text{H}_4-\text{CH}_2-\text{CH}_2-\text{CH}_2-\text{P}(=\text{O})(\text{CH}_2)_2\text{OCO}(\text{CH}_2)_2\text{COOH}$ | $\text{--CH}_2-\text{C}_6\text{H}_4-\text{CH}_2-\text{CH}_2-\text{CH}_2-\text{S}-\text{C}(=\text{S})-\text{N}(\text{C}_2\text{H}_5)-(\text{CH}_2)_2\text{COOH}$ |
| 215                               | (B-215)   |                             | $\text{--CH}_2-\text{C}_6\text{H}_4-\text{CH}_2-\text{CH}_2-\text{CH}_2-\text{P}(=\text{O})(\text{CH}_2)_2\text{OCO}(\text{CH}_2)_2\text{COOH}$ | $\text{--CH}_2-\text{C}_6\text{H}_4-\text{CH}_2-\text{CH}_2-\text{CH}_2-\text{S}-\text{C}(=\text{S})-\text{N}(\text{C}_2\text{H}_5)-(\text{CH}_2)_2\text{COOH}$ |
| 216                               | (B-216)   |                             | $\text{--CH}_2-\text{C}_6\text{H}_4-\text{CH}_2-\text{CH}_2-\text{CH}_2-\text{P}(=\text{O})(\text{CH}_2)_2\text{OCO}(\text{CH}_2)_2\text{COOH}$ | $\text{--CH}_2-\text{C}_6\text{H}_4-\text{CH}_2-\text{CH}_2-\text{CH}_2-\text{S}-\text{C}(=\text{S})-\text{N}(\text{C}_2\text{H}_5)-(\text{CH}_2)_2\text{COOH}$ |

SYNTHESIS EXAMPLES 217 TO 223 OF RESIN  
(B): Resins (B-217) to (B-223)

A mixed solution of 63.6 g of methyl methacrylate, 31.4 g of methyl acrylate, 5 g of 2-hydroxyethyl methacrylate,  $1 \times 10^{-3}$  mole of Initiator shown in Table 18 below and 100 g of tetrahydrofuran was subjected to light irradiation for 8

hours in the same manner as described in Synthesis Example 201 of Resin (B). The resulting polymer was reprecipitated in 1.5 liters of methanol and the precipitates formed were collected by filtration and dried. The yield of each of the polymers obtained was in a range of from 70 to 80 g and the Mw thereof was in a range of from  $8 \times 10^4$  to  $10 \times 10^4$ .

TABLE 18

| Synthesis Example of Resin (B) | Resin (B) | Initiator (I)                                                                                             |                                                                                                                                              | -R                                                                                        |
|--------------------------------|-----------|-----------------------------------------------------------------------------------------------------------|----------------------------------------------------------------------------------------------------------------------------------------------|-------------------------------------------------------------------------------------------|
|                                |           | [P]                                                                                                       | [P]                                                                                                                                          |                                                                                           |
| 217                            | (B-217)   | $(\text{CH}_2)_4\text{R}$<br>$\text{R} \leftarrow \text{CH}_2\text{Si}(\text{CH}_2)_4\text{R}$<br>(I-211) | $-\text{S}-\overset{\text{CH}_3}{\underset{\text{S}}{\text{C}}}-\text{O}(\text{CH}_2)_4\text{COOH}$                                          | $(\text{CH}_2)_4$<br>$\leftarrow \text{CH}_2\text{Si}(\text{CH}_2)_4$<br>(I-211)          |
| 218                            | (B-218)   | $\text{CONH}(\text{CH}_2)_2\text{R}$<br>$\text{R} \leftarrow \text{CH}_2\text{HNOC}$                      | $-\text{S}-\overset{\text{CH}_3}{\underset{\text{S}}{\text{C}}}-\text{N}-(\text{CH}_2)_2\text{COOH}$<br>(I-212)                              | $\text{CONH}(\text{CH}_2)_2$<br>$\text{HNOC}-(\text{CH}_2)_2$                             |
| 219                            | (B-219)   | $\text{R}(\text{CH}_2)_2\text{OOC}$                                                                       | $-\text{S}-\overset{\text{COO}(\text{CH}_2)_2\text{R}}{\underset{\text{S}}{\text{C}}}-\text{O}(\text{CH}_2)_4\text{SO}_3\text{H}$<br>(I-213) | $-\text{OOC}(\text{CH}_2)_2\text{OOC}$<br>$-(\text{CH}_2)_2\text{OOC}-$                   |
| 220                            | (B-220)   | $\text{R} \leftarrow \text{CH}_2\text{NOC}(\text{CH}_2)_3\text{CON}(\text{CH}_2)_2\text{R}$               | $-\text{S}-\overset{\text{C}_2\text{H}_5}{\underset{\text{S}}{\text{C}}}-\text{N}-(\text{CH}_2)_2\text{COOH}$<br>(I-214)                     | $\text{NCO}(\text{CH}_2)_3\text{CON}(\text{CH}_2)_2-$<br>$\leftarrow \text{CH}_2\text{N}$ |



TABLE 18-continued

| Synthesis<br>Example of<br>Resin (B) | Resin<br>(B) | Initiator (I)                                                                                 | -R                                                                                            |                                                                              |
|--------------------------------------|--------------|-----------------------------------------------------------------------------------------------|-----------------------------------------------------------------------------------------------|------------------------------------------------------------------------------|
|                                      |              |                                                                                               | $\text{CON}(\text{CH}_2)_2\text{R}_2$                                                         | $-\text{S}-\overset{\parallel}{\text{C}}-\text{O}(\text{CH}_2)_3\text{COOH}$ |
| 221                                  | (B-221)      |            |            | $-\text{S}-\overset{\parallel}{\text{C}}-\text{O}(\text{CH}_2)_3\text{COOH}$ |
| 222                                  | (B-222)      | $\text{R}-\text{H}_2\text{C}-\overset{\text{I}}{\underset{\text{R}}{\text{CHCH}_2}}-\text{R}$ | $\text{R}-\text{H}_2\text{C}-\overset{\text{I}}{\underset{\text{R}}{\text{CHCH}_2}}-\text{R}$ | $-\text{S}-\overset{\parallel}{\text{C}}-\text{O}(\text{CH}_2)_6\text{COOH}$ |
| 223                                  | (B-223)      |            |            | $-\text{S}-\overset{\parallel}{\text{C}}-\text{O}(\text{CH}_2)_6\text{COOH}$ |



## 129

SYNTHESIS EXAMPLES 224 TO 228 OF RESIN  
(B): Resins (B-224) to (B-228)

A mixture of monomers corresponding to the polymer components shown in Table 19 below and 15.4 g of Initiator (I-202) described above was heated to a temperature of 40° C. under nitrogen gas stream, followed by light irradiation in the same manner as described in Synthesis Example 201 of Resin (B) to conduct polymerization for 5 hours. The solid material obtained was collected, dissolved in 100 g of tetrahydrofuran, and then 19.5 g of methyl acrylate and 0.5 g of acrylic acid were added thereto. The mixture was heated to a temperature of 50° C. under nitrogen gas stream and polymerized by irradiation with light in the same manner as above. The reaction mixture obtained was reprecipitated in one liter of methanol, and the precipitates formed were collected and dried. The yield of each of the resulting polymers was in a range of from 65 to 75 g and the  $M_w$  thereof was in a range of from  $9 \times 10^4$  to  $1.2 \times 10^5$ .

5

10

15

20

## 130

SYNTHESIS EXAMPLES 229 TO 235 OF RESIN  
(B): Resins (B-229) to (B-235)

A mixture of 57 g of methyl methacrylate, 28 g of methyl acrylate and 1.3 g of Initiator (I-218) having the following structure was heated to a temperature of 40° C. under nitrogen gas stream, followed by light irradiation in the same manner as described in Synthesis Example 201 of Resin (B) to conduct polymerization for 4 hours.

Initiator (I-218)



The solid material obtained was dissolved in 100 g of tetrahydrofuran, and monomers corresponding to the polymer components shown in Table 20 below were added thereto. The mixture was heated to a temperature of 50° C.

TABLE 19

| Synthesis Example of Resin (B) | Resin (B) | Polymer Component of Block $+X+$ (weight ratio)                                                                                                                                                                                                                                                                                                                                                                                                                                                                                                                                                                                                                                                                                                                 |
|--------------------------------|-----------|-----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| 224                            | (B-224)   | $  \begin{array}{c}  \text{CH}_2 + \text{P} + \text{R} \\    \\  \text{R} + \text{P} + \text{H}_2\text{C} \\    \\  \text{CH}_2 + \text{P} + \text{R} \\    \\  \text{CH}_2 + \text{P} + \text{R}  \end{array}  \quad  \begin{array}{c}  \text{CH}_2 + \text{P} + \text{R} \\    \\  \text{R} : -\text{S}-\text{C} \begin{array}{c} \text{N} \backslash \\ \parallel \\ \text{S} / \end{array} \begin{array}{c} \text{C}_2\text{H}_5 \\   \\ (\text{CH}_2)_2\text{COOH} \end{array} \\    \\  \text{COOCH}_3 \quad \text{COOH}  \end{array}  $ $  +\text{P}]: +\text{X} \xrightarrow{80} \text{b} \left( \text{CH}_2 - \text{CH} \xrightarrow{19.5} \text{COOCH}_3 \right)_{19.5} \left( \text{CH}_2 - \text{CH} \xrightarrow{0.5} \text{COOH} \right)_{0.5}  $ |
| 225                            | (B-225)   | $  \begin{array}{c}  \text{CH}_3 \\    \\  \text{CH}_2 - \text{C} \xrightarrow{64} \text{CH}_2 - \text{CH} \xrightarrow{16} \\    \quad   \\  \text{COOCH}_3 \quad \text{COOC}_2\text{H}_5  \end{array}  $                                                                                                                                                                                                                                                                                                                                                                                                                                                                                                                                                      |
| 226                            | (B-226)   | $  \begin{array}{c}  \text{CH}_3 \\    \\  \text{CH}_2 - \text{C} \xrightarrow{53.6} \text{CH}_2 - \text{CH} \xrightarrow{26.4} \\    \quad   \\  \text{COOCH}_3 \quad \text{COOC}_2\text{H}_5  \end{array}  $                                                                                                                                                                                                                                                                                                                                                                                                                                                                                                                                                  |
| 227                            | (B-227)   | $  \begin{array}{c}  \text{CH}_3 \\    \\  \text{CH}_2 - \text{C} \xrightarrow{65} \text{CH}_2 - \text{CH} \xrightarrow{15} \\    \quad   \\  \text{COOC}_2\text{H}_5 \quad \text{C}_6\text{H}_5  \end{array}  $                                                                                                                                                                                                                                                                                                                                                                                                                                                                                                                                                |
| 228                            | (B-228)   | $  \begin{array}{c}  \text{CH}_3 \\    \\  \text{CH}_2 - \text{C} \xrightarrow{70} \text{CH}_2 - \text{CH} \xrightarrow{10} \\    \quad   \\  \text{COOC}_6\text{H}_5 \quad \text{COOCH}_3  \end{array}  $                                                                                                                                                                                                                                                                                                                                                                                                                                                                                                                                                      |

## 131

under nitrogen gas stream and polymerized by irradiation with light in the same manner as above. The reaction mixture obtained was reprecipitated in one liter of methanol, and the precipitates formed were collected and dried. The yield of each of the resulting polymers was in a range of from 70 to 80 g and the  $M_w$  thereof was in a range of from  $9 \times 10^4$  to  $1.1 \times 10^5$ .

## 132

## EXAMPLE I-1

A mixture of 6 g (solid basis) of Resin (A-2), 34 g (solid basis) of Resin (B-1), 200 g of photoconductive zinc oxide, 0.018 g of Methine Dye (I-1) having the following structure, 0.15 g of phthalic anhydride and 300 g of toluene was dispersed by a homogenizer (manufactured by Nippon Seiki K.K.) at a rotation of  $6 \times 10^3$  r.p.m. for 10 minutes to prepare

TABLE 20

| Synthesis Example of Resin (B) | Resin (B) | Polymer Component of Block $\text{+ Y +}$ (weight ratio)                                                                                                                                                                                                                          |  |               |
|--------------------------------|-----------|-----------------------------------------------------------------------------------------------------------------------------------------------------------------------------------------------------------------------------------------------------------------------------------|-----------------------------------------------------------------------------------|---------------|
|                                |           |                                                                                                                                                                                                                                                                                   | $\text{CH}_3$                                                                     | $\text{CH}_3$ |
| 229                            | (B-229)   | $\text{+CH}_2 - \overset{\text{CH}_3}{\underset{\text{COOCH}_2\text{C}_6\text{H}_5}{\text{C}}} \text{H}_{12.5} - \text{CH}_2 - \overset{\text{CH}_3}{\underset{\text{COO}(\text{CH}_2)_2\text{NHCOOCH}_3}{\text{C}}} \text{H}_{2.5} -$                                            | $\text{CH}_3$                                                                     | $\text{CH}_3$ |
| 230                            | (B-230)   | $\text{+CH}_2 - \overset{\text{CH}_3}{\underset{\text{COOCH}_3}{\text{CH}}} \text{H}_{14.2} - \text{CH}_2 - \overset{\text{CH}_3}{\underset{\text{COO}(\text{CH}_2)_2\text{OCO}}{\text{CH}}} \text{H}_{0.8} - \text{C}_6\text{H}_4 - \text{C}(=\text{O}) - \text{C}(=\text{O}) -$ | $\text{CH}_3$                                                                     |               |
| 231                            | (B-231)   | $\text{+CH}_2 - \overset{\text{CH}_3}{\underset{\text{COOCH}_2\text{C}_6\text{H}_5}{\text{CH}}} \text{H}_{14.7} - \text{CH}_2 - \overset{\text{CH}_3}{\underset{\text{CH}_2\text{O}-\text{P}(\text{OH})-\text{OH}}{\text{CH}}} \text{H}_{0.3} -$                                  |                                                                                   |               |
| 232                            | (B-232)   | $\text{+CH}_2 - \overset{\text{CH}_3}{\underset{\text{COOC}_2\text{H}_5}{\text{CH}}} \text{H}_{14.5} - \text{CH}_2 - \overset{\text{CH}_3}{\underset{\text{CONH}-\text{C}_6\text{H}_4-\text{COOH}}{\text{CH}}} \text{H}_{0.5} -$                                                  |                                                                                   |               |
| 233                            | (B-233)   | $\text{+CH}_2 - \overset{\text{CH}_3}{\underset{\text{COOCH}_3}{\text{CH}}} \text{H}_{14.7} - \text{CH}_2 - \overset{\text{CH}_3}{\underset{\text{COO}(\text{CH}_2)_2\text{O}-\text{P}(\text{OCH}_3)-\text{OH}}{\text{CH}}} \text{H}_{0.3} -$                                     |                                                                                   |               |
| 234                            | (B-234)   | $\text{+CH}_2 - \overset{\text{CH}_3}{\underset{\text{COOCH}_3}{\text{C}}} \text{H}_{13} - \text{CH}_2 - \overset{\text{CH}_3}{\underset{\text{COO}(\text{CH}_2)_2\text{OCH}_3}{\text{C}}} \text{H}_2 -$                                                                          | $\text{CH}_3$                                                                     | $\text{CH}_3$ |
| 235                            | (B-235)   | $\text{+CH}_2 - \overset{\text{CH}_3}{\underset{\text{COOCH}_3}{\text{C}}} \text{H}_{10} - \text{CH}_2 - \overset{\text{CH}_3}{\underset{\text{COOCH}_2\text{C}_6\text{H}_5}{\text{CH}}} \text{H}_5 -$                                                                            | $\text{CH}_3$                                                                     | $\text{CH}_3$ |

133

a coating composition for a light-sensitive layer. The coating composition was coated on paper, which had been subjected to electrically conductive treatment, by a wire bar at a dry coverage of 25 g/m<sup>2</sup>, followed by drying at 110°C. for 10 seconds. The coated material was then allowed to stand in a dark place at 20°C. and 65% RH for 24 hours to prepare an electrophotographic light-sensitive material (hereinafter simply referred to as light-sensitive material, sometimes).

### Methine Dye (I-1)



5

10



Mw:  $7.5 \times 10^4$  (graft copolymer)

With each of the light-sensitive material thus prepared,  
15 electrostatic characteristics and image forming performance  
were evaluated. The results obtained are shown in Table I-1  
below.

TABLE I-1

|                                                    | Example I-1 | Comparative Example I-1                                      | Comparative Example I-2                                      |
|----------------------------------------------------|-------------|--------------------------------------------------------------|--------------------------------------------------------------|
| <u>Electrostatic*<sup>1)</sup> Characteristics</u> |             |                                                              |                                                              |
| <u>V<sub>10</sub> (-V)</u>                         |             |                                                              |                                                              |
| I (20° C., 65% RH)                                 | 730         | 700                                                          | 715                                                          |
| II (30° C., 80% RH)                                | 705         | 680                                                          | 690                                                          |
| III (15° C., 30% RH)                               | 745         | 720                                                          | 730                                                          |
| D.R.R. (90 sec value) (%)                          |             |                                                              |                                                              |
| I (20° C., 65% RH)                                 | 88          | 83                                                           | 87                                                           |
| II (30° C., 80% RH)                                | 82          | 77                                                           | 81                                                           |
| III (15° C., 30% RH)                               | 89          | 84                                                           | 85                                                           |
| <u>E<sub>1/10</sub> (erg/cm<sup>2</sup>)</u>       |             |                                                              |                                                              |
| I (20° C., 65% RH)                                 | 17.0        | 21                                                           | 17.5                                                         |
| II (30° C., 80% RH)                                | 16.3        | 20.1                                                         | 17.0                                                         |
| III (15° C., 30% RH)                               | 22          | 27                                                           | 24.5                                                         |
| <u>Image Forming*<sup>2)</sup> Performance</u>     |             |                                                              |                                                              |
| I (20° C., 65% RH)                                 | Very good   | Good                                                         | Good                                                         |
| II (30° C., 80% RH)                                | Good        | Unevenness<br>in half tone<br>area, slight<br>background fog | Unevenness<br>in half tone<br>area, slight<br>background fog |
| III (15° C., 30% RH)                               | Good        | White spots<br>in image<br>portion                           | White spots<br>in image<br>portion                           |

### COMPARATIVE EXAMPLE I-1

An electrophotographic light-sensitive material was prepared in the same manner as in Example I-1, except for using 34 g of Resin (R-I-1) having the following structure in place of 34 g of Resin (B-1) used in Example I-1.

### Comparative Resin (R-I-1)



Mw:  $7 \times 10^4$  (random copolymer)

### COMPARATIVE EXAMPLE I-2

An electrophotographic light-sensitive material was prepared in the same manner as in Example I-1, except for using

50 The evaluation of each item shown in Table I-1 was conducted in the following manner.

#### \*1) Electrostatic Characteristics

The light-sensitive material was charged with a corona discharge to a voltage of -6 kV for 20 seconds in a dark room at a temperature of 20° C. and 65% RH using a paper analyzer ("Paper Analyzer SP-428" manufactured by Kawaguchi Denki K.K.). Ten seconds after the corona discharge, the surface potential  $V_{10}$  was measured. The sample was then allowed to stand in the dark for an additional 90 seconds, and the potential  $V_{100}$  was measured. The dark charge retention rate (DRR; %), i.e., percent retention of potential after dark decay for 90 seconds, was calculated from the following equation:

$$DRR(\%) = (V_{100}/V_{10}) \times 100$$

Separately, the surface of photoconductive layer was charged to  $-400$  V with a corona discharge and then exposed

to light emitted from a gallium-aluminum-arsenic semiconductor laser (oscillation wavelength: 780 nm), and the time required for decay of the surface potential  $V_{10}$  to one-tenth was measured, and the exposure amount  $E_{1/10}$  ( $\text{erg}/\text{cm}^2$ ) was calculated therefrom. The measurements were conducted under ambient condition of 20° C. and 65% RH (I), 30° C. and 80% RH (II) or 15° C. and 30% RH (III).  
\*2) Image Forming Performance

After the light-sensitive material was allowed to stand for one day under the ambient condition shown below, the light-sensitive material was charged to -6 kV and exposed to light emitted from a gallium-aluminum-arsenic semiconductor laser (oscillation wavelength: 780 nm; output: 2.8 mW) at an exposure amount of 64  $\text{erg}/\text{cm}^2$  (on the surface of the photoconductive layer) at a pitch of 25  $\mu\text{m}$  and a scanning speed of 300 m/sec. The thus formed electrostatic latent image was developed with a liquid developer ELP-T (produced by Fuji Photo Film Co., Ltd.), washed with a rinse solution of isoparaffinic solvent Isopar G (manufactured by Esso Chemical K.K.) and fixed. The duplicated image obtained was visually evaluated for fog and image quality. The ambient condition at the time of image formation was 20° C. and 65% RH (Condition I), 30° C. and 80% RH (Condition II) or 15° C. and 30% RH (Condition III).

As can be seen from the results shown in Table I-1, the light-sensitive material according to the present invention exhibited good electrostatic characteristics and provided duplicated image which was clear and free from background fog, even when the ambient condition was fluctuated. On the contrary, while the light-sensitive materials of Comparative Examples I-1 and I-2 exhibited good image forming performance under the ambient condition of normal temperature and normal humidity (Condition I), the occurrence of unevenness was observed in the highly accurate image portions, in particular, half tone areas of continuous gradation under the ambient condition of high temperature and high humidity (Condition II) regardless of the electrostatic characteristics. Also a slight background fog remained without removing after the rinse treatment. Further, the occurrence of unevenness of small white spots at random in the image portion was observed under the ambient condition of low temperature and low temperature (Condition III).

From all these considerations, it is thus clear that an electrophotographic light-sensitive material satisfying both

treated in the same manner as described in Example I-1 to prepare an electrophotographic light-sensitive material.

Methine Dye (I-II)



COMPARATIVE EXAMPLE I-3

An electrophotographic light-sensitive material was prepared in the same manner as in Example I-2, except for using 35 g of Resin (R-I-3) having the following structure in place of 35 g of Resin (B-2) used in Example I-2.

Comparative Resin (R-I-3)



COMPARATIVE EXAMPLE I-4

An electrophotographic light-sensitive material was prepared in the same manner as in Example I-2, except for using 35 g of Resin (R-I-4) having the following structure in place of 35 g of Resin (B-2) used in Example I-2.

Comparative Resin (R-I-4)



requirements of electrostatic characteristics and image forming performance (in particular, for highly accurate image) and being advantageously employed particularly in a scanning exposure system using a semiconductor laser beam can be obtained only using the binder resin according to the present invention.

EXAMPLE I-2

A mixture of 5 g (solid basis) of Resin (A-15), 35 g (solid basis) of Resin (B-2), 200 g of photoconductive zinc oxide, 0.020 g of Methine Dye (I-II) having the following structure, 0.20 g of N-hydroxymaleimide and 300 g of toluene was

55

60

65

With each of the light-sensitive materials thus-prepared, a film property in terms of surface smoothness, mechanical strength, electrostatic characteristics and image forming performance were evaluated. Further, printing property was evaluated when it was used as an electrophotographic lithographic printing plate precursor. The results obtained are shown in Table I-2 below.

TABLE I-2

|                                                                    | Example I-2                | Comparative Example I-3                                                  | Comparative Example I-4                                                  |
|--------------------------------------------------------------------|----------------------------|--------------------------------------------------------------------------|--------------------------------------------------------------------------|
| Smoothness of Photoconductive* <sup>3)</sup> Layer (sec/cc)        | 380                        | 385                                                                      | 390                                                                      |
| Mechanical Strength of* <sup>4)</sup> Photoconductive Layer (%)    | 96                         | 78                                                                       | 84                                                                       |
| <u>Electrostatic Characteristics</u>                               |                            |                                                                          |                                                                          |
| <u><math>V_{10}</math> (-V)</u>                                    |                            |                                                                          |                                                                          |
| I (20° C., 65% RH)                                                 | 685                        | 675                                                                      | 680                                                                      |
| II (30° C., 80% RH)                                                | 665                        | 660                                                                      | 660                                                                      |
| III (15° C., 30% RH)                                               | 700                        | 690                                                                      | 695                                                                      |
| D.R.R. (%) (90 sec value)                                          |                            |                                                                          |                                                                          |
| I (20° C., 65% RH)                                                 | 86                         | 83                                                                       | 85                                                                       |
| II (30° C., 80% RH)                                                | 83                         | 77                                                                       | 81                                                                       |
| III (15° C., 30% RH)                                               | 87                         | 85                                                                       | 86                                                                       |
| <u><math>E_{1/V_{10}}</math> (erg/cm<sup>2</sup>)</u>              |                            |                                                                          |                                                                          |
| I (20° C., 65% RH)                                                 | 17.0                       | 21.4                                                                     | 20.0                                                                     |
| II (30° C., 80% RH)                                                | 16.7                       | 20.3                                                                     | 19.4                                                                     |
| III (15° C., 30% RH)                                               | 20                         | 24.5                                                                     | 23.2                                                                     |
| <u>Image Forming Performance</u>                                   |                            |                                                                          |                                                                          |
| I (20° C., 65% RH)                                                 | Good                       | Good                                                                     | Good                                                                     |
| II (30° C., 80% RH)                                                | Good                       | Unevenness in half tone area                                             | Slight unevenness in half tone area                                      |
| III (15° C., 30% RH)                                               | Good                       | Unevenness in half tone area, unevenness of white spots in image portion | Unevenness in half tone area, unevenness of white spots in image portion |
| <u>Water Retentivity of*<sup>5)</sup> Light-Sensitive Material</u> | No-background stain at all | Background stain                                                         | Slight background stain                                                  |
| Printing Durability* <sup>6)</sup>                                 | 10,000 Prints              | 4,500 Prints                                                             | 6,000 Prints                                                             |

The evaluation of each item shown in Table I-2 was conducted in the following manner.

#### \*3) Smoothness of Photoconductive Layer

The smoothness (sec/cc) of the light-sensitive material was measured using a Beck's smoothness test machine (manufactured by Kumagaya Riko K.K.) under an air volume condition of 1 cc.

#### \*4) Mechanical Strength of Photoconductive Layer

The surface of the light-sensitive material was repeatedly (1000 times) rubbed with emery paper (#1000) under a load of 75 g/cm<sup>2</sup> using a Heidon 14 Model surface testing machine (manufactured by Shinto Kagaku K.K.). After dusting, the abrasion loss of the photoconductive layer was measured to obtain film retention (%).

#### \*5) Water Retentivity of Light-Sensitive Material

A light-sensitive material without subjecting to plate making was passed twice through an etching processor using an aqueous solution obtained by diluting an oil-desensitizing solution ELP-EX (produced by Fuji Photo Film Co., Ltd.) to a five-fold volume with distilled water to conduct an oil-desensitizing treatment of the surface of the photoconductive layer. The material thus-treated was mounted on an offset printing machine ("611XLA-II Model" manufactured by Hamada Printing Machine Manufacturing Co.) and printing was conducted using distilled water as dampening water. The extent of background stain occurred on the 50th print was visually evaluated. This testing method corresponds to evaluation of water retentivity after oil-desensitizing treatment of the light-sensitive material under the forced condition.

#### \*6) Printing Durability

The light-sensitive material was subjected to plate making in the same manner as described in \*2) above to form toner

35 images, and the surface of the photoconductive layer was subjected to oil-desensitization treatment by passing twice through an etching processor using ELP-EX. The resulting lithographic printing plate was mounted on an offset printing machine ("Oliver Model 52", manufactured by Sakurai Seisakusho K.K.), and printing was carried out on paper. The number of prints obtained until background stains in the non-image areas appeared or the quality of the image areas was deteriorated was taken as the printing durability. The larger the number of the prints, the higher the printing durability.

40 As can be seen from the results shown in Table I-2, the light-sensitive material according to the present invention had good surface smoothness, film strength and electrostatic characteristics of the photoconductive layer. The duplicated image obtained was clear and free from background fog. These results appear to be due to sufficient adsorption of the binder resin onto the photoconductive substance and sufficient covering of the surface of the particles with the binder resin. For the same reason, when it was used as an offset master plate precursor, oil-desensitization of the offset master plate precursor with an oil-desensitizing solution was sufficient to render the non-image areas satisfactorily hydrophilic and adhesion of ink was not observed at all as a result of the evaluation of water retentivity under the forced condition. On practical printing using the resulting master plate, 10,000 prints of clear image without background stains were obtained.

45 50 55 60 65 On the contrary, with the light-sensitive materials of Comparative Examples I-3 and I-4, the occurrence of slight background stain in non-image area, unevenness in highly accurate image of continuous gradation and unevenness of white spots in image portion was observed when the image

formation was conducted under severe conditions. Further, as a result of the test on water retentivity of these light-sensitive materials to make offset master plates, the adhesion of ink was observed. The printing durability thereof was in a range of from 4,000 to 6,000 prints.

From these results it is believed that the resin (A) and the resin (B) according to the present invention suitably interacts with zinc oxide particles to form the condition under which an oil-desensitizing reaction proceeds easily and sufficiently with an oil-desensitizing solution and that the remarkable improvement in film strength is achieved by the action of the resin (B).

#### EXAMPLES I-3 TO I-22

Each electrophotographic light-sensitive material was prepared in the same manner as described in Example I-2, except for using each of Resins (A) and Resins (B) shown in Table I-3 below in place of Resin (A-15) and Resin (B-2) used in Example I-2, respectively.

TABLE I-3

| Example | Resin (A) | Resin (B) |
|---------|-----------|-----------|
| I-3     | A-1       | B-1       |
| I-4     | A-6       | B-3       |
| I-5     | A-7       | B-4       |
| I-6     | A-8       | B-5       |
| I-7     | A-9       | B-6       |
| I-8     | A-12      | B-7       |
| I-9     | A-14      | B-8       |
| I-10    | A-18      | B-9       |
| I-11    | A-22      | B-10      |
| I-12    | A-23      | B-11      |
| I-13    | A-24      | B-12      |
| I-14    | A-25      | B-13      |
| I-15    | A-26      | B-14      |
| I-16    | A-27      | B-16      |
| I-17    | A-28      | B-17      |
| I-18    | A-21      | B-18      |
| I-19    | A-17      | B-20      |
| I-20    | A-20      | B-21      |
| I-21    | A-4       | B-23      |
| I-22    | A-29      | B-24      |

40

The electrostatic characteristics and image forming performance of each of the light-sensitive materials were determined in the same manner as described in Example I-1. Each 5 light-sensitive material exhibited good electrostatic characteristics. As a result of the evaluation on image forming performance of each light-sensitive material, it was found that clear duplicated images having good reproducibility of 10 fine lines and letters and no occurrence of unevenness in half tone areas without the formation of background fog were obtained.

Further, when these electrophotographic light-sensitive 15 materials were employed as offset master plate precursors under the same printing condition as described in Example I-2, more than 10,000 good prints were obtained respectively.

20 It can be seen from the results described above that each of the light-sensitive materials according to the present invention was satisfactory in all aspects of the surface 25 smoothness and film strength of the photoconductive layer, electrostatic characteristics and printing property.

#### EXAMPLES I-23 TO I-26

Each electrophotographic light-sensitive material was prepared in the same manner as described in Example I-1, except for using each of the dyes shown in Table I-4 below 35 in place of Methine Dye (I-1) used in Example I-1.

TABLE I-4

| Example      | Dye | Chemical Structure of Dye |
|--------------|-----|---------------------------|
| I-23 (I-III) |     |                           |
| I-24 (I-IV)  |     |                           |

TABLE I-4-continued

| Example | Dye    | Chemical Structure of Dye |
|---------|--------|---------------------------|
| I-25    | (I-V)  |                           |
| I-26    | (I-VI) |                           |

Each of the light-sensitive materials according to the present invention was excellent in charging properties, dark charge retention rate and photosensitivity, and provided clear duplicated images free from background fog even when processed under severe conditions of high temperature and high humidity (30° C. and 80% RH) and low temperature and low humidity (15° C. and 30% RH).

#### EXAMPLES I-27 AND I-28

A mixture of 6.5 g of Resin (A-1) (Example I-27) or Resin (A-7) (Example I-28), 33.5 g of Resin (B-21), 200 g of photoconductive zinc oxide, 0.02 g of uranine, 0.03 g of Methine Dye (I-VII) having the following structure, 0.03 g of Methine Dye (I-VIII) having the following structure, 0.18 g of p-hydroxybenzoic acid and 300 g of toluene was dispersed by a homogenizer at a rotation of  $7 \times 10^3$  r.p.m. for 10 minutes to prepare a coating composition for a light-sensitive layer. The coating composition was coated on paper, which had been subjected to electrically conductive treatment, by a wire bar at a dry coverage of  $25 \text{ g/m}^2$ , and dried for 20 seconds at 110° C. Then, the coated material was allowed to stand in a dark place for 24 hours under the conditions of 20° C. and 65% RH to prepare each electro-photographic light-sensitive material.



#### COMPARATIVE EXAMPLE I-5

An electrophotographic light-sensitive material was prepared in the same manner as in Example I-27, except for using 33.5 g of Resin (R-I-5) having the following structure in place of 33.5 g of Resin (B-21) used in Example I-27.

## Comparative Resin (R-I-5)

Mw:  $7.5 \times 10^4$ 

With each of the light-sensitive materials thus prepared, various characteristics were evaluated in the same manner as in Example I-2. The results obtained are shown in Table I-5 below.

ELP-404V (manufactured by Fuji Photo Film Co., Ltd.) using ELP-T as a toner. The duplicated image thus obtained was visually evaluated for fog and image quality. The ambient condition at the time of image formation was 20°C.

TABLE I-5

|                                                    | Example I-27  | Example I-28  | Comparative Example I-5                            |
|----------------------------------------------------|---------------|---------------|----------------------------------------------------|
| Binder Resin                                       | (A-1)/(B-21)  | (A-7)/(B-21)  | (A-1)/(R-I-5)                                      |
| Smoothness of Photoconductive Layer (sec/cc)       | 450           | 455           | 445                                                |
| Mechanical Strength of Photoconductive Layer (%)   | 95            | 96            | 81                                                 |
| <u>Electrostatic Characteristics<sup>47)</sup></u> |               |               |                                                    |
| <u><math>V_{10}</math> (-V)</u>                    |               |               |                                                    |
| I (20°C, 65% RH)                                   | 650           | 695           | 625                                                |
| II (30°C, 80% RH)                                  | 635           | 680           | 605                                                |
| III (15°C, 30% RH)                                 | 665           | 705           | 640                                                |
| D.R.R. (%)                                         |               |               |                                                    |
| I (20°C, 65% RH)                                   | 90            | 95            | 86                                                 |
| II (30°C, 80% RH)                                  | 87            | 90            | 79                                                 |
| III (15°C, 30% RH)                                 | 91            | 96            | 87                                                 |
| <u><math>E_{1/10}</math> (lux · sec)</u>           |               |               |                                                    |
| I (20°C, 65% RH)                                   | 10.5          | 8.7           | 13.5                                               |
| II (30°C, 80% RH)                                  | 9.6           | 8.1           | 12.7                                               |
| III (15°C, 30% RH)                                 | 11.8          | 10.3          | 14.8                                               |
| <u>Image Forming<sup>48)</sup> Performance</u>     |               |               |                                                    |
| I (20°C, 65% RH)                                   | Good          | Very good     | Good                                               |
| II (30°C, 80% RH)                                  | Good          | Very good     | Edge mark of cutting, unevenness in half tone area |
| III (15°C, 30% RH)                                 | Good          | Very good     | Edge mark of cutting, unevenness in image portion  |
| Water Retentivity of Light-Sensitive Material      | Good          | Good          | Slight background stain                            |
| Printing Durability                                | 10,000 Prints | 10,000 Prints | Background stain from the start of printing        |

The characteristics were evaluated in the same manner as in Example I-2, except that some electrostatic characteristics and image forming performance were evaluated according to the following test methods.

\*7) Electrostatic Characteristics:  $E_{1/10}$ 

The surface of the photoconductive layer was charged to -400 V with corona discharge, and then irradiated by visible light of the illuminance of 2.0 lux on the surface of the photoconductive layer. Then, the time required for decay of the surface potential ( $V_{10}$ ) to  $1/10$  thereof was determined, and the exposure amount  $E_{1/10}$  (lux-sec) was calculated therefrom.

## \*8) Image Forming Performance

The electrophotographic light-sensitive material was allowed to stand for one day under the ambient condition described below, the light-sensitive material was subjected to plate making by a full-automatic plate making machine

and 65% RH (Condition I), 30°C. and 80% RH (Condition II) or 15°C. and 30% RH (Condition III). The original used for the duplication was composed of cuttings of other originals pasted up thereon.

55 From the results, it can be seen that each of the light-sensitive materials according to the present invention exhibited good mechanical strength of the photoconductive layer.

On the contrary, with the light-sensitive material of Comparative Example I-5 the value of mechanical strength was lower than them, and the value of  $E_{1/10}$  of electrostatic characteristics degraded particularly under the ambient condition of low temperature and low humidity (Condition III), while they were good under the ambient condition of normal temperature and normal humidity (Condition I). On the other hand, the electrostatic characteristics of the light-sensitive materials according to the present invention were good. Particularly, those of Example I-28 using the resin (A)

having the specified substituent were very good. The value of  $E_{10}$  thereof was particularly small.

With respect to image forming performance, the edge mark of cuttings pasted up was observed as background fog in the non-image areas in the light-sensitive material of Comparative Example I-5. Also, the occurrence of unevenness in half tone area of continuous gradation and unevenness of small white spots in image portion were observed on the duplicated image when the ambient conditions at the time of the image formation were high temperature and high humidity (Condition II) and low temperature and low humidity (Condition III).

Further, each of these light-sensitive materials was subjected to the oil-desensitizing treatment to prepare an offset printing plate and using the resulting plate printing was conducted. The plates according to the present invention provided 10,000 prints of clear image without background stains. However, with the plate of Comparative Example I-5, the above-described edge mark of cuttings pasted up was not removed with the oil-desensitizing treatment and the background stains occurred from the start of printing.

It can be seen from the results described above that only the light-sensitive materials according to the present invention can have excellent performance.

TABLE I-6

| Example | Resin (A) | Resin (B) |
|---------|-----------|-----------|
| I-30    | A-1       | B-1       |
| I-31    | A-2       | B-3       |
| I-32    | A-3       | B-4       |
| I-33    | A-4       | B-5       |
| I-34    | A-5       | B-7       |
| I-35    | A-6       | B-8       |
| I-36    | A-12      | B-9       |
| I-37    | A-13      | B-10      |
| I-38    | A-15      | B-11      |
| I-39    | A-16      | B-12      |
| I-40    | A-19      | B-13      |
| I-41    | A-22      | B-14      |
| I-42    | A-23      | B-15      |
| I-43    | A-25      | B-16      |
| I-44    | A-26      | B-17      |
| I-45    | A-27      | B-18      |
| I-46    | A-28      | B-19      |
| I-47    | A-24      | B-20      |
| I-48    | A-17      | B-21      |
| I-49    | A-8       | B-22      |
| I-50    | A-9       | B-23      |
| I-51    | A-7       | B-2       |
| I-52    | A-18      | B-16      |
| I-53    | A-16      | B-24      |

Each of the light-sensitive materials according to the present invention was excellent in charging properties, dark charge retention rate and photosensitivity, and provided a clear duplicated image free from background fog and scratches of fine lines even under severe conditions of high temperature and high humidity (30° C. and 80% RH) and low temperature and low humidity (15° C. and 30% RH). Further, when these materials were employed as offset master plate precursors, 10,000 prints of a clear image free from background stains were obtained respectively.

## EXAMPLE I-29

A mixture of 5.5 g of Resin (A-24), 34.5 g of Resin (B-21), 200 g of photoconductive zinc oxide, 0.02 g of uranine, 0.04 g of Rose Bengal, 0.03 g of bromophenol blue, 0.40 g of phthalic anhydride and 300 g of toluene was treated in the same manner as described in Example I-27 to prepare an electrophotographic light-sensitive material.

As the result of the evaluation of various characteristics in the same manner as described in Example I-27, it can be seen that the light-sensitive material according to the present invention is excellent in charging properties, dark charge retention rate and photosensitivity, and provides a clear duplicated image free from background fog under severe conditions of high temperature and high humidity (30° C. and 80% RH) and low temperature and low humidity (15° C. and 30% RH). Further, when the material was employed as an offset master plate precursor, 10,000 prints of clear image were obtained.

## EXAMPLES I-30 TO I-53

Each electrophotographic light-sensitive material was prepared in the same manner as described in Example I-29, except for using 5 g of each of Resin (A) and 35 g of each of Resin (B) shown in Table I-6 below in place of 5.5 g of Resin (A-24) and 34.5 g of Resin (B-21) used in Example I-29, respectively.

40

## EXAMPLE II-1

A mixture of 4 g (solid basis) of Resin (A-102), 36 g (solid basis) of Resin (B-1), 200 g of photoconductive zinc oxide, 0.018 g of Methine Dye (II-1) having the following structure, 0.10 g of phthalic anhydride and 300 g of toluene was dispersed by a homogenizer (manufactured by Nippon Seiki K.K.) at a rotation of  $6 \times 10^3$  r.p.m. for 10 minutes to prepare a coating composition for a light-sensitive layer. The coating composition was coated on paper, which had been subjected to electrically conductive treatment, by a wire bar at a dry coverage of 20 g/m<sup>2</sup>, followed by drying at 110° C. for 10 seconds. The coated material was then allowed to stand in a dark place at 20° C. and 65% RH for 24 hours to prepare an electrophotographic light-sensitive material.

Methine Dye (II-1)



### COMPARATIVE EXAMPLE II-1

An electrophotographic light-sensitive material was prepared in the same manner as in Example II-1, except for using 36 g of Resin (R-II-1) having the following structure in place of 36 g of Resin (B-1) used in Example II-1.

### Comparative Resin (R-II-1)



Mw:  $7 \times 10^4$  (random copolymer)

## COMPARATIVE EXAMPLE II-2

An electrophotographic light-sensitive material was prepared in the same manner as in Example II-1, except for using 36 g of Resin (R-II-2) having the following structure in place of 36 g of Resin (B-i) used in Example II-1.



Mw:  $7.5 \times 10^4$  (graft copolymer)

With each of the light-sensitive material thus prepared, electrostatic characteristics and image forming performance were evaluated. The results obtained are shown in Table II-1 below.

#### \*1) Electrostatic Characteristics

The light-sensitive material was charged with a corona discharge to a voltage of  $-6$  kV for 20 seconds in a dark

room at a temperature of 20° C. and 65% RH using a paper analyzer ("Paper Analyzer SP-428" manufactured by Kawaguchi Denki K.K.). Ten seconds after the corona discharge, the surface potential  $V_{10}$  was measured. The sample was then allowed to stand in the dark for an additional 90 seconds, and the potential  $V_{10}$  was measured.

10 additional 90 seconds, and the potential  $V_{100}$  was measured. The dark charge retention rate (DRR; %), i.e., percent retention of potential after dark decay for 90 seconds, was calculated from the following equation:

$$DRR(\%) = (V_{100}/V_{10}) \times 100$$

Separately, the surface of photoconductive layer was charged to  $-400$  V with a corona discharge and then exposed to light emitted from a gallium-aluminum-arsenic semi-

to light emitted from a gallium-aluminum-arsenic semiconductor laser (oscillation wavelength: 780 nm), and the time required for decay of the surface potential  $V_{10}$  to one-tenth was measured, and the exposure amount  $E_{V_{10}}$  ( $\text{erg}/\text{cm}^2$ ) was calculated therefrom. The measurements were conducted under ambient condition of 20° C. and 65% RH (Condition I), 30° C. and 80% RH (Condition II) or 15° C. and 30% RH (Condition III).

## \*2) Image Forming Performance

After the light-sensitive material was allowed to stand for one day under the ambient condition shown below, the light-sensitive material was charged to  $-6$  kV and exposed to light emitted from a gallium-aluminum-arsenic semiconductor laser (oscillation wavelength: 780 nm; output: 2.8

TABLE II-1

|                                                    | Example II-1 | Comparative Example II-1                                            | Comparative Example II-2                                                   |
|----------------------------------------------------|--------------|---------------------------------------------------------------------|----------------------------------------------------------------------------|
| <u>Electrostatic*<sup>1)</sup> Characteristics</u> |              |                                                                     |                                                                            |
| <u>V<sub>10</sub> (-V)</u>                         |              |                                                                     |                                                                            |
| I (20° C., 65% RH)                                 | 730          | 700                                                                 | 735                                                                        |
| II (30° C., 80% RH)                                | 715          | 680                                                                 | 720                                                                        |
| III (15° C., 30% RH)                               | 725          | 695                                                                 | 725                                                                        |
| D.R.R. (90 sec value) (%)                          |              |                                                                     |                                                                            |
| I (20° C., 65% RH)                                 | 85           | 83                                                                  | 85                                                                         |
| II (30° C., 80% RH)                                | 80           | 78                                                                  | 81                                                                         |
| III (15° C., 30% RH)                               | 85           | 84                                                                  | 84                                                                         |
| <u>E<sub>1/10</sub> (erg/cm<sup>2</sup>)</u>       |              |                                                                     |                                                                            |
| I (20° C., 65% RH)                                 | 22           | 23                                                                  | 23                                                                         |
| II (30° C., 80% RH)                                | 24           | 26                                                                  | 25                                                                         |
| III (15° C., 30% RH)                               | 28           | 32                                                                  | 30                                                                         |
| <u>Image Forming*<sup>2)</sup> Performance</u>     |              |                                                                     |                                                                            |
| I (20° C., 65% RH)                                 | Good         | Good                                                                | Good                                                                       |
| II (30° C., 80% RH)                                | Good         | Unevenness<br>in half tone<br>area                                  | Slight unevenness<br>in half tone<br>area                                  |
| III (15° C., 30% RH)                               | Good         | Unevenness<br>in half tone<br>area, white spots<br>in image portion | Slight unevenness<br>in half tone<br>area, white spots<br>in image portion |

The evaluation of each item shown in Table II-1 was conducted in the following manner.

65 mW) at an exposure amount of 64 erg/cm<sup>2</sup> (on the surface of the photoconductive layer) at a pitch of 25  $\mu$ m and a scanning speed of 300 m/sec. The thus formed electrostatic latent image was developed with a liquid developer ELP-T.

## 149

(produced by Fuji Photo Film Co., Ltd.), washed with a rinse solution of isoparaffinic solvent Isopar G (manufactured by Esso Chemical K.K.) and fixed. The duplicated image obtained was visually evaluated for fog and image quality. The ambient condition at the time of image formation was 20° C. and 65% RH (Condition I), 30° C. and 80% RH (Condition II) or 15° C. and 30% RH (Condition III).

As can be seen from the results shown in Table II-1, the light-sensitive material according to the present invention exhibited good electrostatic characteristics and provided a duplicated image which was clear and free from background



fog, even when the ambient condition was fluctuated. On the contrary, while the light-sensitive materials of Comparative Examples II-1 and II-2 exhibited good image forming performance under the ambient condition of normal temperature and normal humidity (Condition I), the occurrence of unevenness was observed in the highly accurate image portions, in particular, half tone areas of continuous gradation under the ambient condition of high temperature and high humidity (Condition II) regardless of the electrostatic characteristics. Also a slight background fog remained without removing after the rinse treatment. Further, the occurrence of unevenness of small white spots at random in the image portion was observed under the ambient condition of low temperature and low temperature (Condition III).

From all these considerations, it is thus clear that an electrophotographic light-sensitive material satisfying both requirements of electrostatic characteristics and image forming performance (in particular, for highly accurate image) and being advantageously employed particularly in a scanning exposure system using a semiconductor laser beam can

## 150

0.020 g of Methine Dye (II-II) having the following structure, 0.20 g of N-hydroxymaleimide and 300 g of toluene was treated in the same manner as described in Example II-1 to prepare an electrophotographic light-sensitive material.

## COMPARATIVE EXAMPLE II-3

An electrophotographic light-sensitive material was prepared in the same manner as in Example II-2, except for using 35 g of Resin (R-II-3) having the following structure in place of 35 g of Resin (B-2) used in Example II-2.



## COMPARATIVE EXAMPLE II-4

An electrophotographic light-sensitive material was prepared in the same manner as in Example II-2, except for using 35 g of Resin (R-II-4) having the following structure in place of 35 g of Resin (B-2) used in Example II-2.

## Comparative Resin (R-II-4)



be obtained only using the binder resin according to the present invention.

## EXAMPLE II-2

A mixture of 5 g (solid basis) of Resin (A-111), 35 g (solid basis) of Resin (B-2), 200 g of photoconductive zinc oxide,

With each of the light-sensitive materials thus-prepared, a film property in terms of surface smoothness, mechanical strength, electrostatic characteristics and image forming performance were evaluated. Further, printing property was evaluated when it was used as an electrophotographic lithographic printing plate precursor. The results obtained are shown in Table II-2 below.

TABLE II-2

|                                                                | Example II-2  | Comparative Example II-3                                                 | Comparative Example II-4                                                 |
|----------------------------------------------------------------|---------------|--------------------------------------------------------------------------|--------------------------------------------------------------------------|
| Smoothness of Photoconductive* <sup>3</sup> Layer (sec/cc)     | 430           | 450                                                                      | 435                                                                      |
| Mechanical Strength of* <sup>4</sup> Photoconductive Layer (%) | 92            | 80                                                                       | 87                                                                       |
| Electrostatic Characteristics                                  |               |                                                                          |                                                                          |
| <u><math>V_{10}</math> (-V)</u>                                |               |                                                                          |                                                                          |
| I (20° C., 65% RH)                                             | 720           | 695                                                                      | 710                                                                      |
| II (30° C., 80% RH)                                            | 700           | 670                                                                      | 690                                                                      |
| III (15° C., 30% RH)                                           | 715           | 700                                                                      | 715                                                                      |
| D.R.R. (%) (90 sec value)                                      |               |                                                                          |                                                                          |
| I (20° C., 65% RH)                                             | 86            | 84                                                                       | 85                                                                       |
| II (30° C., 80% RH)                                            | 81            | 77                                                                       | 80                                                                       |
| III (15° C., 30% RH)                                           | 85            | 83                                                                       | 83                                                                       |
| <u><math>E_{1/10}</math> (erg/cm<sup>2</sup>)</u>              |               |                                                                          |                                                                          |
| I (20° C., 65% RH)                                             | 20            | 28                                                                       | 25                                                                       |
| II (30° C., 80% RH)                                            | 23            | 34                                                                       | 28                                                                       |
| III (15° C., 30% RH)                                           | 26            | 39                                                                       | 32                                                                       |
| Image Forming Performance                                      |               |                                                                          |                                                                          |
| I (20° C., 65% RH)                                             | Good          | Good                                                                     | Good                                                                     |
| II (30° C., 80% RH)                                            | Good          | Unevenness in half tone area                                             | Unevenness in half tone area                                             |
| III (15° C., 30% RH)                                           | Good          | Unevenness in half tone area, unevenness of white spots in image portion | Unevenness in half tone area, unevenness of white spots in image portion |
| Water Retentivity of* <sup>5</sup> Light-Sensitive Material    | Good          | Slight background stain                                                  | Slight background stain                                                  |
| Printing Durability* <sup>6</sup>                              | 10,000 Prints | 3,000 Prints                                                             | 5,000 Prints                                                             |

The evaluation of each item shown in Table II-2 was 35 conducted in the following manner.

\*3) Smoothness of Photoconductive Layer

The smoothness (sec/cc) of the light-sensitive material was measured using a Beck's smoothness test machine (manufactured by Kumagaya Riko K.K.) under an air volume condition of 1 cc. 40

\*4) Mechanical Strength of Photoconductive Layer

The surface of the light-sensitive material was repeatedly (1000 times) rubbed with emery paper (#1000) under a load of 75 g/cm<sup>2</sup> using a Heidon 14 Model surface testing 45 machine (manufactured by Shinto Kagaku K.K.). After dusting, the abrasion loss of the photoconductive layer was measured to obtain film retention (%).

\*5) Water Retentivity of Light-Sensitive Material

A light-sensitive material without subjecting to plate 50 making was passed twice through an etching processor using an aqueous solution obtained by diluting an oil-desensitizing solution ELP-EX (produced by Fuji Photo Film Co., Ltd.) to a seven-fold volume with distilled water to conduct an oil-desensitizing treatment of the surface of the photoconductive layer. The material thus-treated was mounted on an offset printing machine ("611XLA-II Model" manufactured by Hamada Printing Machine Manufacturing Co.) and printing was conducted using distilled water as dampening water. The extent of background stain occurred on the 50th print 55 was visually evaluated. This testing method corresponds to evaluation of water retentivity after oil-desensitizing treatment of the light-sensitive material under the forced condition.

\*6) Printing Durability

The light-sensitive material was subjected to plate making in the same manner as described in \*2) above to form toner

images, and the surface of the photoconductive layer was subjected to oil-desensitization treatment by passing twice through an etching processor using ELP-EX. The resulting lithographic printing plate was mounted on an offset printing machine ("Oliver Model 52", manufactured by Sakurai Seisakusho K.K.), and printing was carried out on paper. The number of prints obtained until background stains in the non-image areas appeared or the quality of the image areas was deteriorated was taken as the printing durability. The larger the number of the prints, the higher the printing durability.

As can be seen from the results shown in Table II-2, the light-sensitive material according to the present invention had good surface smoothness, film strength and electrostatic characteristics of the photoconductive layer. The duplicated image obtained was clear and free from background fog. These results appear to be due to sufficient adsorption of the binder resin onto the photoconductive substance and sufficient covering of the surface of the particles with the binder resin. For the same reason, when it was used as an offset master plate precursor, oil-desensitization of the offset master plate precursor with an oil-desensitizing solution was sufficient to render the non-image areas satisfactorily hydrophilic and adhesion of ink was not observed at all as a result of the evaluation of water retentivity under the forced condition. On practical printing using the resulting master plate, 10,000 prints of clear image without background stains were obtained.

On the contrary, with the light-sensitive materials of Comparative Examples II-3 and II-4, the occurrence of slight background stain in non-image area, unevenness in highly accurate image of continuous gradation and unevenness of white spots in image portion was observed when the

image formation was conducted under severe conditions. Further, as a result of the test on water retentivity of these light-sensitive materials to make offset master plates, the adhesion of ink was observed. The printing durability thereof was in a range of from 3,000 to 5,000 prints.

From these results it is believed that the resin (A) and the resin (B) according to the present invention suitably interacts with zinc oxide particles to form the condition under which an oil-desensitizing reaction proceeds easily and sufficiently with an oil-desensitizing solution and that the remarkable improvement in film strength is achieved by the action of the resin (B).

#### EXAMPLES II-3 TO II-18

Each electrophotographic light-sensitive material was prepared in the same manner as described in Example II-2, except for using each of Resins (A) and Resins (B) shown in Table II-3 below in place of Resin (A-111) and Resin (B-2) used in Example II-2, respectively.

TABLE II-3

| Example | Resin (A) | Resin (B) |
|---------|-----------|-----------|
| II-3    | A-108     | B-3       |
| II-4    | A-110     | B-4       |
| II-5    | A-112     | B-5       |
| II-6    | A-113     | B-6       |
| II-7    | A-114     | B-7       |
| II-8    | A-119     | B-9       |
| II-9    | A-121     | B-11      |
| II-10   | A-124     | B-12      |
| II-11   | A-127     | B-15      |
| II-12   | A-129     | B-16      |
| II-13   | A-130     | B-17      |
| II-14   | A-132     | B-19      |
| II-15   | A-133     | B-21      |
| II-16   | A-134     | B-22      |

TABLE II-3-continued

| Example | Resin (A) | Resin (B) |
|---------|-----------|-----------|
| 5       | II-17     | A-135     |
|         | II-18     | A-117     |
|         |           | B-23      |
|         |           | B-24      |

The electrostatic characteristics and image forming performance of each of the light-sensitive materials were determined in the same manner as described in Example II-1. Each light-sensitive material exhibited good electrostatic characteristics. As a result of the evaluation on image forming performance of each light-sensitive material, it was found that clear duplicated images having good reproducibility of fine lines and letters and no occurrence of unevenness in half tone areas without the formation of background fog were obtained.

Further, when these electrophotographic light-sensitive materials were employed as offset master plate precursors under the same printing condition as described in Example II-2, more than 10,000 good prints were obtained respectively.

It can be seen from the results described above that each of the light-sensitive materials according to the present invention was satisfactory in all aspects of the surface smoothness and film strength of the photoconductive layer, electrostatic characteristics and printing property.

#### EXAMPLES II-19 TO II-22

Each electrophotographic light-sensitive material was prepared in the same manner as described in Example II-1, except for using each of the dyes shown in Table II-4 below in place of Methine Dye (II-1) used in Example II-1.

TABLE II-4

| Example        | Dye | Chemical Structure of Dye |
|----------------|-----|---------------------------|
| II-19 (II-III) |     |                           |
| II-20 (II-IV)  |     |                           |
| II-21 (II-V)   |     |                           |

TABLE II-4-continued

| Example Dye   | Chemical Structure of Dye                                                          |
|---------------|------------------------------------------------------------------------------------|
| II-22 (II-VI) |  |

15  
Each of the light-sensitive materials according to the present invention was excellent in charging properties, dark charge retention rate and photosensitivity, and provided clear duplicated images free from background fog even when processed under severe conditions of high temperature and high humidity (30° C. and 80% RH) and low temperature and low humidity (15° C. and 30% RH).

### EXAMPLES II-23 AND II-24

A mixture of 6.5 g of Resin (A-101) (Example II-23) or Resin (A-118) (Example II-24), 33.5 g of Resin (B-23), 200 g of photoconductive zinc oxide, 0.02 g of uranine, 0.03 g of Methine Dye (II-VII) having the following structure, 0.03 g of Methine Dye (II-VIII) having the following structure, 0.18 g of p-hydroxybenzoic acid and 300 g of toluene was dispersed by a homogenizer at a rotation of  $7 \times 10^3$  r.p.m. for 10 minutes to prepare a coating composition for a light-sensitive layer. The coating composition was coated on paper, which had been subjected to electrically conductive treatment, by a wire bar at a dry coverage of  $25 \text{ g/m}^2$ , and dried for 20 seconds at  $110^\circ \text{ C}$ . Then, the coated material was allowed to stand in a dark place for 24 hours under the conditions of  $20^\circ \text{ C}$ . and 65% RH to prepare each electro-photographic light-sensitive material.



Mw:  $7.5 \times 10^4$

With each of the light-sensitive materials thus prepared, various characteristics were evaluated in the same manner as in Example II-2. The results obtained are shown in Table II-5 below.

TABLE II-5

|                                                  | Example II-23  | Example II-24 | Comparative Example II-5                                   |
|--------------------------------------------------|----------------|---------------|------------------------------------------------------------|
| Binder Resin                                     | (A-101)/(B-23) | (A-118)/B-23) | (A-101)/(R-II-5)                                           |
| Smoothness of Photoconductive Layer (sec/cc)     | 430            | 450           | 420                                                        |
| Mechanical Strength of Photoconductive Layer (%) | 90             | 91            | 78                                                         |
| Electrostatic Characteristics*7)                 |                |               |                                                            |
| <u><math>V_{10}</math> (-V)</u>                  |                |               |                                                            |
| I (20° C., 65% RH)                               | 600            | 780           | 605                                                        |
| II (30° C., 80% RH)                              | 580            | 765           | 570                                                        |
| III (15° C., 30% RH)                             | 605            | 770           | 600                                                        |
| D.R.R. (%)                                       |                |               |                                                            |
| I (20° C., 65% RH)                               | 90             | 96            | 86                                                         |
| II (30° C., 80% RH)                              | 86             | 92            | 80                                                         |
| III (15° C., 30% RH)                             | 91             | 95            | 84                                                         |
| <u><math>E_{1/10}</math> (lux · sec)</u>         |                |               |                                                            |
| I (20° C., 65% RH)                               | 11.5           | 9.8           | 12.3                                                       |
| II (30° C., 80% RH)                              | 12.0           | 10.4          | 13                                                         |
| III (15° C., 30% RH)                             | 13.1           | 11.0          | 14.4                                                       |
| Image Forming*8) Performance                     |                |               |                                                            |
| I (20° C., 65% RH)                               | Good           | Very good     | Good                                                       |
| II (30° C., 80% RH)                              | Good           | Very good     | Unevenness in half tone area                               |
| III (15° C., 30% RH)                             | Good           | Very good     | Unevenness in half tone area, white spots in image portion |
| Water Retentivity of Light-Sensitive Material    | Good           | Good          | Background stain                                           |
| Printing Durability                              | 10,000 Prints  | 10,000 Prints | Background stain from the start of printing                |

The characteristics were evaluated in the same manner as in Example II-2, except that some electrostatic characteristics and image forming performance were evaluated according to the following test methods.

\*7) Electrostatic Characteristics:  $E_{1/10}$

The surface of the photoconductive layer was charged to -400 V with corona discharge, and then irradiated by visible light of the illuminance of 2.0 lux on the surface of the photoconductive layer. Then, the time required for decay of the surface potential ( $V_{10}$ ) to  $1/10$  thereof was determined, and the exposure amount  $E_{1/10}$  (lux·sec) was calculated therefrom.

\*8) Image Forming Performance

The electrophotographic light-sensitive material was allowed to stand for one day under the ambient condition described below, the light-sensitive material was subjected to plate making by a full-automatic plate making machine ELP-404V (manufactured by Fuji Photo Film Co., Ltd.) using ELP-T as a toner. The duplicated image thus obtained was visually evaluated for fog and image quality. The ambient condition at the time of image formation was 20° C. and 65% RH (Condition I), 30° C. and 80% RH (Condition II) or 15° C. and 30% RH (Condition III). The original used for the duplication was composed of cuttings of other originals pasted up thereon.

From the results, it can be seen that each of the light-sensitive materials according to the present invention exhibited good mechanical strength of the photoconductive layer. On the contrary, with the light-sensitive material of Comparative Example II-5 the value of mechanical strength was lower than them, and the value of  $E_{1/10}$  of electrostatic characteristics degraded particularly under the ambient con-

dition of low temperature and low humidity (Condition III), while they were good under the ambient condition of normal temperature and normal humidity (Condition I). On the other hand, the electrostatic characteristics of the light-sensitive materials according to the present invention were good. Particularly, those of Example II-24 using the resin (A) having the specified substituent were very good. The value of  $E_{1/10}$  thereof was particularly small.

With respect to image forming performance, the edge mark of cuttings pasted up was observed as background fog in the non-image areas in the light-sensitive material of Comparative Example II-5. Also, the occurrence of unevenness in half tone area of continuous gradation and unevenness of small white spots in image portion were observed on the duplicated image when the ambient conditions at the time of the image formation were high temperature and high humidity (Condition II) and low temperature and low humidity (Condition III).

Further, each of these light-sensitive materials was subjected to the oil-desensitizing treatment to prepare an offset printing plate and using the plate printing was conducted. The plates according to the present invention provided 10,000 prints of clear image without background stains. However, with the plate of Comparative Example II-5, the above described edge mark of cuttings pasted up was not removed with the oil-desensitizing treatment and the background stains occurred from the start of printing.

It can be seen from the results described above that only the light-sensitive materials according to the present invention could provide excellent performance.

## EXAMPLE II-25

A mixture of 5 g of Resin (A-123), 35 g of Resin (B-22), 200 g of photoconductive zinc oxide, 0.02 g uranine, 0.04 g of Rose Bengal, 0.03 g of bromophenol blue, 0.40 g of phthalic anhydride and 300 g of toluene was treated in the same manner as described in Example II-24 to prepare an electrophotographic light-sensitive material.

As the result of the evaluation of various characteristics in the same manner as described in Example II-24, it can be seen that the light-sensitive material according to the present invention is excellent in charging properties, dark charge retention rate and photosensitivity, and provides a clear duplicated image free from background fog under severe conditions of high temperature and high humidity (30° C. and 80% RH) and low temperature and low humidity (15° C. and 30% RH). Further, when the material was employed as an offset master plate precursor, 10,000 prints of clear image were obtained.

## EXAMPLES II-26 TO II-49

Each electrophotographic light-sensitive material was prepared in the same manner as described in Example II-25, except for using 5 g of each of Resin (A) and 35 g of each

clear duplicated image free from background fog and scratches of fine lines even under severe conditions of high temperature and high humidity (30° C. and 80% RH) and low temperature and low humidity (15° C. and 30% RH).

Further, when these materials were employed as offset master plate precursors, 10,000 prints of a clear image free from background stains were obtained respectively.

## EXAMPLE III-1

A mixture of 8 g (solid basis) of Resin (A-7), 32 g (solid basis) of Resin (B-101), 200 g of photoconductive zinc oxide, 0.018 g of Methine Dye (III-1) having the following structure, 0.45 g of salicylic acid and 300 g of toluene was dispersed by a homogenizer (manufactured by Nippon Seiki K.K.) at a rotation of  $7 \times 10^3$  r.p.m. for 10 minutes to prepare a coating composition for a light-sensitive layer. The coating composition was coated on paper, which had been subjected to electrically conductive treatment, by a wire bar at a dry coverage of 25 g/m<sup>2</sup>, followed by drying at 110° C. for 10 seconds. The coated material was then allowed to stand in a dark place at 20° C. and 65% RH (relative humidity) for 24 hours to prepare an electrophotographic light-sensitive material.

Methine Dye (III-1)



of Resin (B) shown in Table II-6 below in place of 5 g of Resin (A-123) and 35 g of Resin (B-22) used in Example II-25, respectively.

TABLE II-6

| Example | Resin (A) | Resin (B) |
|---------|-----------|-----------|
| II-26   | A-102     | B-1       |
| II-27   | A-103     | B-2       |
| II-28   | A-104     | B-3       |
| II-29   | A-106     | B-6       |
| II-30   | A-107     | B-7       |
| II-31   | A-109     | B-9       |
| II-32   | A-113     | B-10      |
| II-33   | A-115     | B-11      |
| II-34   | A-116     | B-14      |
| II-35   | A-119     | B-18      |
| II-36   | A-122     | B-24      |
| II-37   | A-123     | B-22      |
| II-38   | A-125     | B-5       |
| II-39   | A-126     | B-19      |
| II-40   | A-127     | B-21      |
| II-41   | A-128     | B-23      |
| II-42   | A-129     | B-24      |
| II-43   | A-130     | B-18      |
| II-44   | A-132     | B-17      |
| II-45   | A-133     | B-8       |
| II-46   | A-134     | B-13      |
| II-47   | A-135     | B-15      |
| II-48   | A-131     | B-22      |
| II-49   | A-118     | B-24      |

Each of the light-sensitive materials according to the present invention was excellent in charging properties, dark charge retention rate and photosensitivity, and provided a

## COMPARATIVE EXAMPLE III-1

An electrophotographic light-sensitive material was prepared in the same manner as in Example III-1, except for using 32 g of Resin (R-III-1) having the following structure in place of 32 g of Resin (B-101) used in Example III-1.

Comparative Resin (R-III-1)



Mw:  $7 \times 10^4$  (random copolymer)

## COMPARATIVE EXAMPLE III-2

An electrophotographic light-sensitive material was prepared in the same manner as in Example III-1, except for using 32 g of Resin (R-III-2) having the following structure in place of 32 g of Resin (B-101) used in Example III-1.

## Comparative Resin (R-III-2)

Mw:  $7.5 \times 10^4$  (graft copolymer)

With each of the light-sensitive materials thus prepared, electrostatic characteristics and image forming performance were evaluated. The results obtained are shown in Table III-1 below.

TABLE III-1

|                                                    | Example III-1 | Comparative Example III-1                                   | Comparative Example III-2                                   |
|----------------------------------------------------|---------------|-------------------------------------------------------------|-------------------------------------------------------------|
| <u>Electrostatic*<sup>1)</sup> Characteristics</u> |               |                                                             |                                                             |
| <u>V<sub>10</sub> (-V)</u>                         |               |                                                             |                                                             |
| I (20° C., 65% RH)                                 | 765           | 750                                                         | 760                                                         |
| II (30° C., 80% RH)                                | 750           | 730                                                         | 750                                                         |
| III (15° C., 30% RH)                               | 770           | 765                                                         | 765                                                         |
| D.R.R. (90 sec value) (%)                          |               |                                                             |                                                             |
| I (20° C., 65% RH)                                 | 86            | 83                                                          | 84                                                          |
| II (30° C., 80% RH)                                | 83            | 78                                                          | 80                                                          |
| III (15° C., 30% RH)                               | 87            | 85                                                          | 85                                                          |
| <u>E<sub>1/10</sub> (erg/cm<sup>2</sup>)</u>       |               |                                                             |                                                             |
| I (20° C., 65% RH)                                 | 20            | 25                                                          | 24                                                          |
| II (30° C., 80% RH)                                | 18            | 21                                                          | 20                                                          |
| III (15° C., 30% RH)                               | 24            | 30                                                          | 30                                                          |
| <u>E<sub>1/100</sub> (erg/cm<sup>2</sup>)</u>      |               |                                                             |                                                             |
| I (20° C., 65% RH)                                 | 31            | 39                                                          | 37                                                          |
| II (30° C., 80% RH)                                | 33            | 42                                                          | 41                                                          |
| III (15° C., 30% RH)                               | 37            | 49                                                          | 45                                                          |
| <u>Image Forming*<sup>2)</sup> Performance</u>     |               |                                                             |                                                             |
| I (20° C., 65% RH)                                 | Good          | Good                                                        | Good                                                        |
| II (30° C., 80% RH)                                | Good          | Unevenness<br>in image portion                              | Unevenness<br>in image portion                              |
| III (15° C., 30% RH)                               | Good          | Unevenness<br>in image portion,<br>slight background<br>fog | Unevenness<br>in image portion,<br>slight background<br>fog |

The evaluation of each item shown in Table III-1 was conducted in the following manner.

## \*1) Electrostatic Characteristics

The light-sensitive material was charged with a corona discharge to a voltage of -6 kV for 20 seconds in a dark room at a temperature of 20° C. and 65% RH using a paper analyzer ("Paper Analyzer SP-428" manufactured by Kawaguchi Denki K.K.). Ten seconds after the corona discharge, the surface potential V<sub>10</sub> was measured. The sample was then allowed to stand in the dark for an additional 90 seconds, and the potential V<sub>100</sub> was measured. The dark charge retention rate (DRR; %), i.e., percent retention of potential after dark decay for 90 seconds, was calculated from the following equation:

$$DRR(\%) = (V_{100}/V_{10}) \times 100$$

Separately, the surface of photoconductive layer was charged to -400 V with a corona discharge and then exposed to light emitted from a gallium-aluminum-arsenic semiconductor laser (oscillation wavelength: 780 nm), and the time required for decay of the surface potential V<sub>10</sub> to one-tenth was measured, and the exposure amount E<sub>1/10</sub> (erg/cm<sup>2</sup>) was calculated therefrom. Further, in the same manner as described above the time required for decay of the surface potential V<sub>10</sub> to one-hundredth was measured, and the exposure amount E<sub>1/100</sub> (erg/cm<sup>2</sup>) was calculated therefrom. The measurements were conducted under ambient condition of 20° C. and 65% RH (Condition I), 30° C. and 80% RH (Condition II) or 15° C. and 30% RH (Condition III).

## \*2) Image Forming Performance

After the light-sensitive material was allowed to stand for one day under the ambient condition shown below, the

light-sensitive material was charged to -6 kV and exposed to light emitted from a gallium-aluminum-arsenic semiconductor laser (oscillation wavelength: 780 nm; output: 2.8 mW) at an exposure amount of 64 erg/cm<sup>2</sup> (on the surface of the photoconductive layer) at a pitch of 25 μm and a scanning speed of 300 m/sec. The thus formed electrostatic latent image was developed with a liquid developer ELP-T (produced by Fuji Photo Film Co., Ltd.), washed with a rinse solution of isoparaffinic solvent Isopar G (manufactured by Esso Chemical K.K.) and fixed. The duplicated image obtained was visually evaluated for fog and image quality. The ambient condition at the time of image formation was 20° C. and 65% RH (Condition I), 30° C. and 80% RH (Condition II) or 15° C. and 30% RH (Condition III).

As can be seen from the results shown in Table III-1, the light-sensitive material according to the present invention had good electrostatic characteristics. The duplicated image obtained thereon was clear and free from background fog.

On the contrary, with the light-sensitive materials of Comparative Examples III-1 and III-2 the decrease in photosensitivity ( $E_{1/10}$  and  $E_{1/100}$ ) occurred, and in the duplicated images the scratches of fine lines and letters were observed and a slight background fog remained without removing after the rinse treatment. Further, the occurrence of unevenness in half tone areas of continuous gradation of the original was observed under the ambient condition II, and the occurrence of small white spots in the image portion was observed under the ambient condition III regardless of the electrostatic characteristics.

The value of  $E_{V100}$  is largely different between the light-sensitive material of the present invention and those of the comparative examples. The value of  $E_{V100}$  indicates an electrical potential remaining in the non-image areas after exposure at the practice of image formation. The smaller this value, the less the background fog in the non-image areas. More specifically, it is required that the remaining potential is decreased to  $-10$  V or less. Therefore, an amount of exposure necessary to make the remaining potential below  $-10$  V is an important factor. In the scanning exposure system using a semiconductor laser beam, it is quite important to make the remaining potential below  $-10$  V by a small exposure amount in view of a design for an optical system of a duplicator (such as cost of the device, and accuracy of the optical system).

From all these considerations, it is thus clear that an electrophotographic light-sensitive material satisfying both

164

### COMPARATIVE EXAMPLE III-3

An electrophotographic light-sensitive material was prepared in the same manner as in Example III-2, except for using 34 g of Resin (R-III-3) having the following structure in place of 34 g of Resin (B-102) used in Example III-2.

### Comparative Resin (R-III-3)



### COMPARATIVE EXAMPLE III-4

An electrophotographic light-sensitive material was prepared in the same manner as in Example III-2, except for using 34 g of Resin (R-III-4) shown below in place of 34 g of Resin (B-102) used in Example III-2.



requirements of electrostatic characteristics and image forming performance and being advantageously employed particularly in a scanning exposure system using a semiconductor laser beam can be obtained only when the binder resin according to the present invention is used.

### EXAMPLE III-2

A mixture of 6 g (solid basis) of Resin (A-23), 34 g (solid basis) of Resin (B-102), 200 g of photoconductive zinc oxide, 0.020 g of Methine Dye (III-II) having the following formula, 0.23 g of N-hydroxyphthalimide and 300 g of toluene was treated in the same manner as described in Example III-1 to prepare an electrophotographic light-sensitive material.

With each of the light-sensitive materials thus-prepared, a film property in terms of surface smoothness, mechanical strength, electrostatic characteristics and image forming performance were evaluated. Further, printing property was evaluated when it was used as an electrophotographic lithographic printing plate precursor. The results obtained are shown in Table III-2 below.

### Methine Dye (III-II)



TABLE III-2

|                                                                 | Example III-2              | Comparative Example III-3                                                | Comparative Example III-4                                                |
|-----------------------------------------------------------------|----------------------------|--------------------------------------------------------------------------|--------------------------------------------------------------------------|
| Smoothness of Photoconductive* <sup>3)</sup> Layer (sec/cc)     | 430                        | 435                                                                      | 425                                                                      |
| Mechanical Strength of* <sup>4)</sup> Photoconductive Layer (%) | 93                         | 76                                                                       | 81                                                                       |
| Electrostatic Characteristics                                   |                            |                                                                          |                                                                          |
| $V_{10}$ (-V)                                                   |                            |                                                                          |                                                                          |
| I (20° C., 65% RH)                                              | 680                        | 640                                                                      | 650                                                                      |
| II (30° C., 80% RH)                                             | 665                        | 620                                                                      | 625                                                                      |
| III (15° C., 30% RH)                                            | 685                        | 650                                                                      | 655                                                                      |
| D.R.R. (%) (90 sec value)                                       |                            |                                                                          |                                                                          |
| I (20° C., 65% RH)                                              | 89                         | 87                                                                       | 89                                                                       |
| II (30° C., 80% RH)                                             | 83                         | 79                                                                       | 82                                                                       |
| III (15° C., 30% RH)                                            | 88                         | 86                                                                       | 87                                                                       |
| $E_{1/10}$ (erg/cm <sup>2</sup> )                               |                            |                                                                          |                                                                          |
| I (20° C., 65% RH)                                              | 20                         | 28                                                                       | 27                                                                       |
| II (30° C., 80% RH)                                             | 19                         | 26                                                                       | 24                                                                       |
| III (15° C., 30% RH)                                            | 27                         | 35                                                                       | 33                                                                       |
| Image Forming Performance                                       |                            |                                                                          |                                                                          |
| I (20° C., 65% RH)                                              | Good                       | Good                                                                     | Good                                                                     |
| II (30° C., 80% RH)                                             | Good                       | Unevenness in half tone area                                             | Slight unevenness in half tone area                                      |
| III (15° C., 30% RH)                                            | Good                       | Unevenness in half tone area, unevenness of white spots in image portion | Unevenness in half tone area, unevenness of white spots in image portion |
| Water Retentivity of* <sup>5)</sup> Light-Sensitive Material    | No background stain at all | Background stain                                                         | Slight background stain                                                  |
| Printing Durability* <sup>6)</sup>                              | 10,000 Prints              | 4,500 Prints                                                             | 6,000 Prints                                                             |

The evaluation of each item shown in Table III-2 was conducted in the following manner.

\*3) Smoothness of Photoconductive Layer

The smoothness (sec/cc) of the light-sensitive material was measured using a Beck's smoothness test machine (manufactured by Kumagaya Riko K.K.) under an air volume condition of 1 cc.

\*4) Mechanical Strength of Photoconductive Layer

The surface of the light-sensitive material was repeatedly (1000 times) rubbed with emery paper (#1000) under a load of 75 g/cm<sup>2</sup> using a Heidon 14 Model surface testing machine (manufactured by Shinto Kagaku K.K.). After dusting, the abrasion loss of the photoconductive layer was measured to obtain film retention (%).

\*5) Water Retentivity of Light-Sensitive Material

A light-sensitive material without subjecting to plate making was passed twice through an etching processor using an aqueous solution obtained by diluting an oil-desensitizing solution ELP-EX (produced by Fuji Photo Film Co., Ltd.) to a five-fold volume with distilled water to conduct an oil-desensitizing treatment of the surface of the photoconductive layer. The material thus-treated was mounted on an offset printing machine ("611XLA-II Model" manufactured by Hamada Printing Machine Manufacturing Co.) and printing was conducted using distilled water as dampening water. The extent of background stain occurred on the 50th print was visually evaluated. This testing method corresponds to evaluation of water retentivity after oil-desensitizing treatment of the light-sensitive material under the forced condition.

\*6) Printing Durability

The light-sensitive material was subjected to plate making in the same manner as described in \*2) above to form toner

images, and the surface of the photoconductive layer was subjected to oil-desensitization treatment by passing twice through an etching processor using ELP-EX. The resulting lithographic printing plate was mounted on an offset printing machine ("Oliver Model 52", manufactured by Sakurai Seisakusho K.K.), and printing was carried out on paper. The number of prints obtained until background stains in the non-image areas appeared or the quality of the image areas was deteriorated was taken as the printing durability. The larger the number of the prints, the higher the printing durability.

As can be seen from the results shown in Table III-2, the light-sensitive material according to the present invention had good surface smoothness, film strength and electrostatic characteristics of the photoconductive layer. The duplicated image obtained was clear and free from background fog. These results appear to be due to sufficient adsorption of the binder resin onto the photoconductive substance and sufficient covering of the surface of the particles with the binder resin. For the same reason, when it was used as an offset master plate precursor, oil-desensitization of the offset master plate precursor with an oil-desensitizing solution was sufficient to render the non-image areas satisfactorily hydrophilic and adhesion of ink was not observed at all as a result of the evaluation of water retentivity under the forced condition. On practical printing using the resulting master plate, 10,000 prints of clear image without background stains were obtained.

On the contrary, with the light-sensitive materials of Comparative Examples III-3 and III-4, the occurrence of slight background stain in non-image area, unevenness in highly accurate image of continuous gradation and unevenness of white spots in image portion was observed when the

image formation was conducted under severe conditions. Further, as a result of the test on water retentivity of these light-sensitive materials to make offset master plates, the adhesion of ink was observed. The printing durability thereof was in a range of from 4,000 to 6,000 prints.

From these results it is believed that the resin (A) and the resin (B) according to the present invention suitably interacts with zinc oxide particles to form the condition under which an oil-desensitizing reaction proceeds easily and sufficiently with an oil-desensitizing solution and that the remarkable improvement in film strength is achieved by the action of the resin (B).

#### EXAMPLES III-3 TO III-22

Each electrophotographic light-sensitive material was prepared in the same manner as described in Example III-2, except for using each of Resins (A) and Resins (B) shown in Table III-3 below in place of Resin (A-23) and Resin (B-102) used in Example III-2, respectively.

TABLE III-3

| Example | Resin (A) | Resin (B) |
|---------|-----------|-----------|
| III-3   | A-1       | B-103     |
| III-4   | A-3       | B-104     |
| III-5   | A-5       | B-101     |
| III-6   | A-6       | B-105     |
| III-7   | A-11      | B-106     |
| III-8   | A-12      | B-107     |
| III-9   | A-16      | B-108     |
| III-10  | A-18      | B-109     |
| III-11  | A-19      | B-111     |
| III-12  | A-20      | B-112     |
| III-13  | A-21      | B-113     |
| III-14  | A-22      | B-115     |
| III-15  | A-23      | B-116     |
| III-16  | A-24      | B-120     |
| III-17  | A-25      | B-121     |
| III-18  | A-26      | 3-123     |
| III-19  | A-27      | B-124     |
| III-20  | A-28      | B-130     |
| III-21  | A-4       | B-131     |
| III-22  | A-10      | 3-133     |

15  
20  
25  
30  
35  
40

The electrostatic characteristics and image forming performance of each of the light-sensitive materials were determined in the same manner as described in Example III-1.

5 Each light-sensitive material exhibited good electrostatic characteristics. As a result of the evaluation on image forming performance of each light-sensitive material, it was found that clear duplicated images having good reproducibility of fine lines and letters and no occurrence of unevenness in half tone areas without the formation of background fog were obtained.

Further, when these electrophotographic light-sensitive materials were employed as offset master plate precursors under the same printing condition as described in Example III-2, more than 10,000 good prints were obtained respectively.

It can be seen from the results described above that each of the light-sensitive materials according to the present invention was satisfactory in all aspects of the surface smoothness and film strength of the photoconductive layer, electrostatic characteristics and printing property.

#### EXAMPLES III-23 TO III-26

Each electrophotographic light-sensitive material was prepared in the same manner as described in Example III-1, except for using each of the dyes shown in Table III-4 below in place of Methine Dye (III-1) used in Example III-1.

TABLE III-4

| Example          | Dye | Chemical Structure of Dye |
|------------------|-----|---------------------------|
| III-23 (III-III) |     |                           |
| III-24 (III-IV)  |     |                           |

TABLE III-4-continued

| Example         | Dye | Chemical Structure of Dye |
|-----------------|-----|---------------------------|
| III-25 (III-V)  |     |                           |
| III-26 (III-VI) |     |                           |

Each of the light-sensitive materials according to the present invention was excellent in charging properties, dark charge retention rate and photosensitivity, and provided clear duplicated images free from background fog even when processed under severe conditions of high temperature and high humidity (30° C. and 80% RH) and low temperature and low humidity (15° C. and 30% RH).

30

## COMPARATIVE EXAMPLE III-5

A mixture of 6.5 g of Resin (A-1) (Example III-27) or Resin (A-22) (Example III-28), 33.5 g of Resin (B-126), 200 g of photoconductive zinc oxide, 0.02 g of uranine, 0.03 g of Methine Dye (III-VII) having the following structure, 0.03 g of Methine Dye (III-VIII) having the following structure, 0.18 g of phthalic anhydride and 300 g of toluene was dispersed by a homogenizer at a rotation of  $7 \times 10^3$  r.p.m. for 8 minutes to prepare a coating composition for a light-sensitive layer. The coating composition was coated on paper, which had been subjected to electrically conductive treatment, by a wire bar at a dry coverage of  $20 \text{ g/m}^2$ , and dried for 20 seconds at 110° C. Then, the coated material was allowed to stand in a dark place for 24 hours under the conditions of 20° C. and 65% RH to prepare each electro-photographic light-sensitive material.

25 An electrophotographic light-sensitive material was prepared in the same manner as in Example III-27, except for using 33.5 g of Resin (R-III-5) having the following structure in place of 33.5 g of Resin (B-126) used in Example III-27.

30

## EXAMPLES III-27 AND III-28

35 A mixture of 6.5 g of Resin (A-1) (Example III-27) or Resin (A-22) (Example III-28), 33.5 g of Resin (B-126), 200 g of photoconductive zinc oxide, 0.02 g of uranine, 0.03 g of Methine Dye (III-VII) having the following structure, 0.03 g of Methine Dye (III-VIII) having the following structure, 0.18 g of phthalic anhydride and 300 g of toluene was dispersed by a homogenizer at a rotation of  $7 \times 10^3$  r.p.m. for 8 minutes to prepare a coating composition for a light-sensitive layer. The coating composition was coated on paper, which had been subjected to electrically conductive treatment, by a wire bar at a dry coverage of  $20 \text{ g/m}^2$ , and dried for 20 seconds at 110° C. Then, the coated material was allowed to stand in a dark place for 24 hours under the conditions of 20° C. and 65% RH to prepare each electro-photographic light-sensitive material.

40

45



Comparative Resin (R-III-5)

Mw:  $7.5 \times 10^4$ 

With each of the light-sensitive materials thus prepared, various characteristics were evaluated in the same manner as in Example III-2. The results obtained are shown in Table III-5 below.

ELP-404V (manufactured by Fuji Photo Film Co., Ltd.) using ELP-T as a toner. The duplicated image thus obtained was visually evaluated for fog and image quality. The ambient condition at the time of image formation was 20° C.

TABLE III-5

|                                                     | Example III-27 | Example III-28 | Comparative Example III-5                          |
|-----------------------------------------------------|----------------|----------------|----------------------------------------------------|
| Binder Resin                                        | (A-1)/(B-126)  | (A-22)/(B-126) | (A-1)/(R-III-5)                                    |
| Smoothness of Photoconductive Layer (sec/cc)        | 430            | 435            | 425                                                |
| Mechanical Strength of Photoconductive Layer (%)    | 93             | 95             | 80                                                 |
| <u>Electrostatic Characteristics<sup>*)7)</sup></u> |                |                |                                                    |
| <u><math>V_{10}</math> (-V)</u>                     |                |                |                                                    |
| I (20° C., 65% RH)                                  | 645            | 750            | 630                                                |
| II (30° C., 80% RH)                                 | 630            | 735            | 605                                                |
| III (15° C., 30% RH)                                | 655            | 760            | 640                                                |
| D.R.R. (%)                                          |                |                |                                                    |
| I (20° C., 65% RH)                                  | 92             | 95             | 92                                                 |
| II (30° C., 80% RH)                                 | 89             | 90             | 84                                                 |
| III (15° C., 30% RH)                                | 93             | 96             | 91                                                 |
| <u><math>E_{1/10}</math> (lux · sec)</u>            |                |                |                                                    |
| I (20° C., 65% RH)                                  | 10.2           | 8.9            | 13.2                                               |
| II (30° C., 80% RH)                                 | 10.8           | 9.2            | 12.9                                               |
| III (15° C., 30% RH)                                | 11.5           | 10.0           | 13.9                                               |
| <u>Image Forming<sup>*)8)</sup> Performance</u>     |                |                |                                                    |
| I (20° C., 65% RH)                                  | Good           | Very good      | Good                                               |
| II (30° C., 80% RH)                                 | Good           | Very good      | Edge mark of cutting, unevenness in half tone area |
| III (15° C., 30% RH)                                | Good           | Very good      | Edge mark of cutting, unevenness in image portion  |
| Water Retentivity of Light-Sensitive Material       | Good           | Good           | Slight background stain                            |
| Printing Durability                                 | 10,000 Prints  | 10,000 Prints  | Background stain from the start of printing        |

The characteristics were evaluated in the same manner as in Example III-2, except that some electrostatic characteristics and image forming performance were evaluated according to the following test methods.

<sup>\*)7)</sup> Electrostatic Characteristics:  $E_{1/10}$

The surface of the photoconductive layer was charged to -400 V with corona discharge, and then irradiated by visible light of the illuminance of 2.0 lux on the surface of the photoconductive layer. Then, the time required for decay of the surface potential ( $V_{10}$ ) to  $1/10$  thereof was determined, and the exposure amount  $E_{1/10}$  (lux-sec) was calculated therefrom.

<sup>\*)8)</sup> Image Forming Performance

The electrophotographic light-sensitive material was allowed to stand for one day under the ambient condition described below, the light-sensitive material was subjected to plate making by a full-automatic plate making machine

and 65% RH (Condition I), 30° C. and 80% RH (Condition II) or 15° C. and 30% RH (Condition III). The original used for the duplication was composed of cuttings of other originals pasted up thereon.

From the results, it can be seen that each of the light-sensitive materials according to the present invention exhibited good mechanical strength of the photoconductive layer.

On the contrary, with the light-sensitive material of Comparative Example III-5 the value of mechanical strength was lower than them, and the value of  $E_{1/10}$  of electrostatic characteristics degraded particularly under the ambient condition of low temperature and low humidity (Condition III), while they were good under the ambient condition of normal temperature and normal humidity (Condition I). On the other hand, the electrostatic characteristics of the light-sensitive materials according to the present invention were good. Particularly, those of Example III-28 using the resin

(A) having the specified substituent were very good. The value of  $E_{\%}$  thereof was particularly small.

With respect to image forming performance, the edge mark of cuttings pasted up was observed as background fog in the non-image areas in the light-sensitive material of Comparative Example III-5. Also the occurrence of unevenness in half tone area of continuous gradation and unevenness of small white spots in image portion were observed on the duplicated image when the ambient conditions at the time of the image formation were high temperature and high humidity (Condition II) and low temperature and low humidity (Condition III).

Further, each of these light-sensitive materials was subjected to the oil-desensitizing treatment to prepare an offset printing plate and using the resulting plate printing was conducted. The plates according to the present invention provided 10,000 prints of clear image without background stains. However, with the plate of Comparative Example III-5, the above described edge mark of cuttings pasted up was not removed with the oil-desensitizing treatment and the background stains occurred from the start of printing.

It can be seen from the results described above that only the light-sensitive materials according to the present invention could provide excellent performance.

#### EXAMPLE III-29

A mixture of 5 g of Resin (A-7), 35 g of Resin (B-108), 200 g of photoconductive zinc oxide, 0.02 g of uranine, 0.04 g of Rose Bengal, 0.03 g of bromophenol blue, 0.40 g of phthalic anhydride and 300 g of toluene was treated in the same manner as described in Example III-27 to prepare an electrophotographic light-sensitive material.

With each of the light-sensitive materials thus prepared, various characteristics were evaluated in the same manner as in Example III-27. It can be seen from the results that the light-sensitive material according to the present invention is excellent in charging properties, dark charge retention rate and photosensitivity, and provides a clear duplicated image free from background fog under severe conditions of high temperature and high humidity (30° C. and 80% RH) and low temperature and low humidity (15° C. and 30% RH). Further, when the material was employed as an offset master plate precursor, 10,000 prints of clear image were obtained.

#### EXAMPLES III-30 TO III-53

Each electrophotographic light-sensitive material was prepared in the same manner as described in Example III-27, except for using 5 g of each of Resin (A) and 35 g of each of Resin (B) shown in Table III-6 below in place of 5 g of Resin (A-7) and 35 g of Resin (B-108) used in Example III-29, respectively.

TABLE III-6

| Example | Resin (A) | Resin (B) |
|---------|-----------|-----------|
| III-30  | A-1       | B-106     |
| III-31  | A-3       | B-101     |
| III-32  | A-4       | B-102     |
| III-33  | A-5       | B-104     |
| III-34  | A-6       | B-105     |
| III-35  | A-9       | B-106     |
| III-36  | A-10      | B-108     |
| III-37  | A-11      | B-110     |
| III-38  | A-12      | B-112     |
| III-39  | A-13      | B-114     |
| III-40  | A-17      | B-116     |
| III-41  | A-19      | B-119     |
| III-42  | A-21      | B-120     |
| III-43  | A-22      | B-121     |
| III-44  | A-24      | B-122     |
| III-45  | A-25      | B-123     |
| III-46  | A-26      | B-124     |
| III-47  | A-27      | B-125     |
| III-48  | A-28      | B-126     |
| III-49  | A-29      | B-127     |
| III-50  | A-14      | B-128     |
| III-51  | A-16      | B-129     |
| III-52  | A-23      | B-131     |
| III-53  | A-27      | B-132     |

Each of the light-sensitive materials according to the present invention was excellent in charging properties, dark charge retention rate and photosensitivity, and provided a clear duplicated image free from background fog and scratches of fine lines even under severe conditions of high temperature and high humidity (30° C. and 80% RH) and low temperature and low humidity (15° C. and 30% RH). Further, when these materials were employed as offset master plate precursors, 10,000 prints of a clear image free from background stains were obtained respectively.

#### EXAMPLE IV-1

A mixture of 6 g (solid basis) of Resin (A-102), 34 g (solid basis) of Resin (B-101), 200 g of photoconductive zinc oxide, 0.018 g of Methine Dye (IV-1) having the following structure, 0.10 g of phthalic anhydride and 300 g of toluene was dispersed by a homogenizer (manufactured by Nippon Seiki K.K.) at a rotation of  $6 \times 10^3$  r.p.m. for 10 minutes to prepare a coating composition for a light-sensitive layer. The coating composition was coated on paper, which had been subjected to electrically conductive treatment, by a wire bar at a dry coverage of 26 g/m<sup>2</sup> followed by drying at 110° C. for 10 seconds. The coated material was then allowed to stand in a dark place at 20° C. and 65% RH for 24 hours to prepare an electrophotographic light-sensitive material.



## COMPARATIVE EXAMPLE IV-1

An electrophotographic light-sensitive material was prepared in the same manner as in Example IV-1, except for using 34 g of Resin (R-IV-1) having the following structure in place of 34 g of Resin (B-101) used in Example IV-1.

Comparative Resin (R-IV-1)



## COMPARATIVE EXAMPLE IV-2

An electrophotographic light-sensitive material was prepared in the same manner as in Example IV-1, except for using 34 g of Resin (R-IV-2) having the following structure in place of 34 g of Resin (B-101) used in Example IV-1.

Comparative Resin (R-IV-2)



Mw:  $7.5 \times 10^4$  (graft copolymer)

With each of the light-sensitive material thus prepared, electrostatic characteristics and image forming performance were evaluated. The results obtained are shown in Table IV-1 below.

The evaluation of each item shown in Table IV-1 was conducted in the following manner.

## \*1) Electrostatic Characteristics

The light-sensitive material was charged with a corona discharge to a voltage of  $-6$  kV for 20 seconds in a dark room at a temperature of  $20^\circ\text{C}$ . and 65% RH using a paper analyzer ("Paper Analyzer SP-428" manufactured by Kawaguchi Denki K.K.). Ten seconds after the corona discharge, the surface potential  $V_{10}$  was measured. The sample was then allowed to stand in the dark for an additional 90 seconds, and the potential  $V_{100}$  was measured. The dark charge retention rate (DRR; %), i.e., percent retention of potential after dark decay for 90 seconds, was calculated from the following equation:

$$DRR(\%) = (V_{100}/V_{10}) \times 100$$

Separately, the surface of photoconductive layer was charged to  $-400$  V with a corona discharge and then exposed to light emitted from a gallium-aluminum-arsenic semi-

conductor laser (oscillation wavelength:  $780$  nm), and the time required for decay of the surface potential  $V_{10}$  to one-tenth was measured, and the exposure amount  $E_{1/10}$  ( $\text{erg}/\text{cm}^2$ ) was calculated therefrom. The measurements

TABLE IV-1

|                                                                    | Example IV-1 | Comparative Example IV-1                   | Comparative Example IV-2                   |
|--------------------------------------------------------------------|--------------|--------------------------------------------|--------------------------------------------|
| <u>Electrostatic*1) Characteristics</u>                            |              |                                            |                                            |
| <u><math>V_{10}</math> (-V)</u>                                    |              |                                            |                                            |
| I (20° C., 65% RH)                                                 | 785          | 740                                        | 770                                        |
| II (30° C., 80% RH)                                                | 770          | 715                                        | 750                                        |
| III (15° C., 30% RH)                                               | 790          | 745                                        | 770                                        |
| DRR. (90 sec value) (%)                                            |              |                                            |                                            |
| I (20° C., 65% RH)                                                 | 89           | 85                                         | 88                                         |
| II (30° C., 80% RH)                                                | 85           | 80                                         | 84                                         |
| III (15° C., 30% RH)                                               | 89           | 84                                         | 89                                         |
| <u><math>E_{1/10}</math> (<math>\text{erg}/\text{cm}^2</math>)</u> |              |                                            |                                            |
| I (20° C., 65% RH)                                                 | 25           | 30                                         | 28                                         |
| II (30° C., 80% RH)                                                | 24           | 27                                         | 26                                         |
| III (15° C., 30% RH)                                               | 30           | 35                                         | 33                                         |
| <u>Image Forming*2) Performance</u>                                |              |                                            |                                            |
| I (20° C., 65% RH)                                                 | Good         | Good                                       | Good                                       |
| II (30° C., 80% RH)                                                | Good         | Unevenness in half tone area               | Unevenness in half tone area               |
| III (15° C., 30% RH)                                               | Good         | Unevenness of white spots in image portion | Unevenness of white spots in image portion |

were conducted under ambient condition of 20° C. and 65% RH (Condition I), 30° C. and 80% RH (Condition II) or 15° C. and 30% RH (Condition III).

\*2) Image Forming Performance

After the light-sensitive material was allowed to stand for one day under the ambient condition shown below, the light-sensitive material was charged to -6 kV and exposed to light emitted from a gallium-aluminum-arsenic semiconductor laser (oscillation wavelength: 780 nm; output: 2.8 mW) at an exposure amount of 64 erg/cm<sup>2</sup> (on the surface of the photoconductive layer) at a pitch of 25 μm and a scanning speed of 300 m/sec. The thus formed electrostatic latent image was developed with a liquid developer ELP-T (produced by Fuji Photo Film Co., Ltd.), washed with a rinse solution of isoparaffinic solvent Isopar G (manufactured by Esso Chemical K.K.) and fixed. The duplicated image obtained was visually evaluated for fog and image quality. The ambient condition at the time of image formation was 20° C. and 65% RH (Condition I), 30° C. and 80% RH (Condition II) or 15° C. and 30% RH (Condition III).

As can be seen from the results shown in Table IV-1, the light-sensitive material according to the present invention

and being advantageously employed particularly in a scanning exposure system using a semiconductor laser beam can be obtained only when the binder resin according to the present invention is used.

EXAMPLE IV-2

A mixture of 6 g (solid basis) of Resin (A-111), 34 g (solid basis) of Resin (B-102), 200 g of photoconductive zinc oxide, 0.020 g of Methine Dye (IV-II) having the following structure, 0.20 g of N-hydroxymaleimide and 300 g of toluene was treated in the same manner as described in Example IV-1 to prepare an electrophotographic light-sensitive material.



exhibited good electrostatic characteristics and provided duplicated image which was clear and free from background fog, even when the ambient condition was fluctuated. On the contrary, while the light-sensitive materials of Comparative Examples IV-1 and IV-2 exhibited good image forming performance under the ambient condition of normal temperature and normal humidity (Condition I), the occurrence of unevenness was observed in the highly accurate image portions, in particular, half tone areas of continuous gradation under the ambient condition of high temperature and high humidity (Condition II) regardless of the electrostatic characteristics. Also, a slight background fog remained without removing after the rinse treatment. Further, the occurrence of unevenness of small white spots at random in the image portion was observed under the ambient condition of low temperature and low temperature (Condition III).

From all these considerations, it is thus clear that an electrophotographic light-sensitive material satisfying both requirements of electrostatic characteristics and image forming performance (in particular, for highly accurate image)

35

COMPARATIVE EXAMPLE IV-3

An electrophotographic light-sensitive material was prepared in the same manner as in Example IV-2, except for using 34 g of Resin (R-IV-3) having the following structure in place of 34 g of Resin (B-102) used in Example IV-2.

Comparative Resin (R-IV-3)



COMPARATIVE EXAMPLE IV-4

An electrophotographic light-sensitive material was prepared in the same manner as in Example IV-2, except for using 34 g of Resin (R-IV-4) having the following structure in place of 34 g of Resin (B-102) used in Example IV-2.

Comparative Resin (R-IV-4)



Mw:  $5.5 \times 10^4$  (graft copolymer)  
 —b— represents a bond between blocks.

With each of the light-sensitive materials thus-prepared, a film property in terms of surface smoothness, mechanical strength, electrostatic characteristics and image forming performance were evaluated. Further, printing property was evaluated when it was used as an electrophotographic lithographic printing plate precursor. The results obtained are shown in Table IV-2 below.

dusting, the abrasion loss of the photoconductive layer was measured to obtain film retention (%).

#### \*5) Water Retentivity of Light-Sensitive Material

A light-sensitive material without subjecting to plate making was passed twice through an etching processor using an aqueous solution obtained by diluting an oil-desensitizing solution ELP-EX (produced by Fuji Photo Film Co., Ltd.) to

TABLE IV-2

|                                                              | Example IV-2               | Comparative Example IV-3                              | Comparative Example IV-4                   |
|--------------------------------------------------------------|----------------------------|-------------------------------------------------------|--------------------------------------------|
| Smoothness of Photoconductive* <sup>3</sup> Layer (sec/cc)   | 410                        | 400                                                   | 420                                        |
| Mechanical Strength of * <sup>4</sup>                        | 92                         | 80                                                    | 86                                         |
| Photoconductive Layer (%)                                    |                            |                                                       |                                            |
| Electrostatic Characteristics                                |                            |                                                       |                                            |
| <u><math>V_{10}</math> (-V)</u>                              |                            |                                                       |                                            |
| I (20° C., 65% RH)                                           | 785                        | 760                                                   | 770                                        |
| II (30° C., 80% RH)                                          | 770                        | 740                                                   | 750                                        |
| III (15° C., 30% RH)                                         | 790                        | 760                                                   | 765                                        |
| D.R.R. (%) (90 sec value)                                    |                            |                                                       |                                            |
| I (20° C., 65% RH)                                           | 87                         | 85                                                    | 87                                         |
| II (30° C., 80% RH)                                          | 84                         | 80                                                    | 85                                         |
| III (15° C., 30% RH)                                         | 88                         | 84                                                    | 86                                         |
| <u><math>E_{1/10}</math> (erg/cm<sup>2</sup>)</u>            |                            |                                                       |                                            |
| I (20° C., 65% RH)                                           | 25                         | 31                                                    | 27                                         |
| II (30° C., 80% RH)                                          | 23                         | 28                                                    | 25                                         |
| III (15° C., 30% RH)                                         | 30                         | 38                                                    | 34                                         |
| <u>Image Forming Performance</u>                             |                            |                                                       |                                            |
| I (20° C., 65% RH)                                           | Good                       | Good                                                  | Good                                       |
| II (30° C., 80% RH)                                          | Good                       | Unevenness in half tone area, slight background stain | Unevenness in half tone area               |
| III (15° C., 30% RH)                                         | Good                       | Unevenness of white spots in image portion            | Unevenness of white spots in image portion |
| Water Retentivity of * <sup>5</sup> Light-Sensitive Material | No background stain at all | Slight background stain                               | Good                                       |
| Printing Durability* <sup>6</sup>                            | 10,000 Prints              | 3,000 Prints                                          | 5,000 Prints                               |

The evaluation of each item shown in Table IV-2 was 55 conducted in the following manner.

#### \*3) Smoothness of Photoconductive Layer

The smoothness (sec/cc) of the light-sensitive material was measured using a Beck's smoothness test machine (manufactured by Kumagaya Riko K.K.) under an air volume condition of 1 cc.

#### \*4) Mechanical Strength of Photoconductive Layer

The surface of the light-sensitive material was repeatedly (1000 times) rubbed with emery paper (#1000) under a load of 75 g/cm<sup>2</sup> using a Heidon 14 Model surface testing machine (manufactured by Shinto Kagaku K.K.). After

60 a five-fold volume with distilled water to conduct an oil-desensitizing treatment of the surface of the photoconductive layer. The material thus-treated was mounted on an offset printing machine ("611XLA-II Model" manufactured by Hamada Printing Machine Manufacturing Co.) and printing was conducted using distilled water as dampening water. The extent of background stain occurred on the 50th print was visually evaluated. This testing method corresponds to evaluation of water retentivity after oil-desensitizing treatment of the light-sensitive material under the forced condition.

## \*6) Printing Durability

The light-sensitive material was subjected to plate making in the same manner as described in \*2) above to form toner images, and the surface of the photoconductive layer was subjected to oil-desensitization treatment by passing twice through an etching processor using ELP-EX. The resulting lithographic printing plate was mounted on an offset printing machine ("Oliver Model 52", manufactured by Sakurai Sei-sakusho K.K.), and printing was carried out on paper. The number of prints obtained until background stains in the non-image areas appeared or the quality of the image areas was deteriorated was taken as the printing durability. The larger the number of the prints, the higher the printing durability.

As can be seen from the results shown in Table IV-2, the light-sensitive material according to the present invention had good surface smoothness, film strength and electrostatic characteristics of the photoconductive layer. The duplicated image obtained was clear and free from background fog. These results appear to be due to sufficient adsorption of the binder resin onto the photoconductive substance and sufficient covering of the surface of the particles with the binder resin. For the same reason, when it was used as an offset master plate precursor, oil-desensitization of the offset master plate precursor with an oil-desensitizing solution was sufficient to render the non-image areas satisfactorily hydrophilic and adhesion of ink was not observed at all as a result of the evaluation of water retentivity under the forced condition. On practical printing using the resulting master plate, 10,000 prints of clear image without background stains were obtained.

On the contrary, with the light-sensitive materials of Comparative Examples IV-3 and IV-4, the occurrence of slight background stain in non-image area, unevenness in highly accurate image of continuous gradation and unevenness of white spots in image portion was observed when the image formation was conducted under severe conditions. Further, as a result of the test on water retentivity of these light-sensitive materials to make offset master plates, the adhesion of ink was observed. The printing durability thereof was at most 5,000 prints.

From these results it is believed that the resin (A) and the resin (B) according to the present invention suitably interacts with zinc oxide particles to form the condition under which an oil-desensitizing reaction proceeds easily and sufficiently with an oil-desensitizing solution and that the remarkable improvement in film strength is achieved by the action of the resin (B).

## EXAMPLES IV-3 TO IV-24

Each electrophotographic light-sensitive material was prepared in the same manner as described in Example IV-2, except for using each of Resins (A) and Resins (B) shown in Table IV-3 below in place of Resin (A-111) and Resin (B-102) used in Example IV-2, respectively.

TABLE IV-3

| Example | Resin (A) | Resin (B) |
|---------|-----------|-----------|
| IV-3    | A-104     | B-103     |
| IV-4    | A-105     | B-104     |
| IV-5    | A-107     | B-105     |
| IV-6    | A-108     | B-106     |
| IV-7    | A-133     | B-107     |
| IV-8    | A-110     | B-108     |
| IV-9    | A-112     | B-109     |
| IV-10   | A-133     | B-110     |
| IV-11   | A-127     | B-111     |
| IV-12   | A-129     | B-112     |
| IV-13   | A-133     | B-123     |
| IV-14   | A-114     | B-113     |
| IV-15   | A-116     | B-114     |
| IV-16   | A-117     | B-115     |
| IV-17   | A-118     | B-118     |
| IV-18   | A-120     | B-119     |
| IV-19   | A-124     | B-121     |
| IV-20   | A-125     | B-124     |
| IV-21   | A-128     | B-128     |
| IV-22   | A-135     | B-131     |
| IV-23   | A-132     | B-132     |
| IV-24   | A-130     | B-133     |

The electrostatic characteristics and image forming performance of each of the light-sensitive materials were determined in the same manner as described in Example IV-1. Each light-sensitive material exhibited good electrostatic characteristics. As a result of the evaluation on image forming performance of each light-sensitive material, it was found that clear duplicated images having good reproducibility of fine lines and letters and no occurrence of unevenness in half tone areas without formation of background fog were obtained.

Further, when these electrophotographic light-sensitive materials were employed as offset master plate precursors under the same printing condition as described in Example IV-2, more than 10,000 good prints were obtained respectively.

It can be seen from the results described above that each of the light-sensitive materials according to the present invention was satisfactory in all aspects of the surface smoothness and film strength of the photoconductive layer, electrostatic characteristics and printing property.

## EXAMPLES IV-25 TO IV-28

Each electrophotographic light-sensitive material was prepared in the same manner as described Example IV-1, except for using each of the dyes shown in Table IV-4 below in place of Methine Dye (IV-1) used in Example IV-1.

TABLE IV-4

| Example        | Dye | Chemical Structure of Dye |
|----------------|-----|---------------------------|
| IV-25 (IV-III) |     |                           |
| IV-26 (IV-IV)  |     |                           |
| IV-27 (IV-V)   |     |                           |
| IV-28 (IV-VI)  |     |                           |

Each of the light-sensitive materials according to the present invention was excellent in charging properties, dark charge retention rate and photosensitivity, and provided clear duplicated images free from background fog even when processed under severe conditions of high temperature and high humidity (30° C. and 80% RH) and low temperature and low humidity (15° C. and 30% RH).

#### EXAMPLES IV-29 AND IV-30

A mixture of 6.5 g of Resin (A-101) (Example IV-29) or Resin (A-119) (Example IV-30), 33.5 g of Resin (B-123), 200 g of photoconductive zinc oxide, 0.02 g of uranine, 0.03

g of Methine Dye (IV-VII) having the following structure, 40 0.03 g of Methine Dye (IV-VIII) having the following structure shown, 0.18 g of p-hydroxybenzoic acid and 300 g of toluene was dispersed by a homogenizer at a rotation of 7×10<sup>3</sup> r.p.m. for 6 minutes to prepare a coating composition for a light-sensitive layer. The coating composition was coated on paper, which had been subjected to electrically conductive treatment, by a wire bar at a dry coverage of 25 g/m<sup>2</sup>, and dried for 20 seconds at 110° C. Then, the coated material was allowed to stand in a dark place for 24 hours under the conditions of 20° C. and 65% RH to prepare each electrophotographic light-sensitive material.



185

-continued



186

## COMPARATIVE EXAMPLE IV-5

An electrophotographic light-sensitive material was prepared in the same manner as in Example IV-29, except for using 33.5 g of Resin (R-IV-5) having the following structure in place of 33.5 g of Resin (B-123) used in Example IV-29.

Comparative Resin (R-IV-5)

Mw:  $7.5 \times 10^4$ 

With each of the light-sensitive materials thus prepared, various characteristics were evaluated in the same manner as in Example IV-2. The results obtained are shown in Table IV-5 below.

10

The characteristics were evaluated in the same manner as in Example IV-2, except that some electrostatic characteristics and image forming performance were evaluated according to the following test methods.

15 \*7) Electrostatic Characteristics:  $E_{1/10}$ 

The surface of the photoconductive layer was charged to -400 V with corona discharge, and then irradiated by visible light of the illuminance of 2.0 lux on the surface of the photoconductive layer. Then, the time required for decay of

TABLE IV-5

|                                                   | Example IV-29   | Example IV-30   | Comparative Example IV-5                    |
|---------------------------------------------------|-----------------|-----------------|---------------------------------------------|
| Binder Resin                                      | (A-101)/(B-123) | (A-119)/(B-123) | (A-101)/R-IV-5                              |
| Smoothness of Photoconductive Layer (sec/cc)      | 450             | 440             | 455                                         |
| Mechanical Strength of Photoconductive Layer (%)  | 92              | 93              | 85                                          |
| <u>Electrostatic Characteristics<sup>7)</sup></u> |                 |                 |                                             |
| <u><math>V_{10}</math> (-V)</u>                   |                 |                 |                                             |
| I (20° C., 65% RH)                                | 580             | 740             | 545                                         |
| II (30° C., 80% RH)                               | 560             | 725             | 530                                         |
| III (15° C., 30% RH)                              | 585             | 750             | 555                                         |
| D.R.R. (%)                                        |                 |                 |                                             |
| I (20° C., 65% RH)                                | 88              | 95              | 86                                          |
| II (30° C., 80% RH)                               | 84              | 92              | 80                                          |
| III (15° C., 30% RH)                              | 87              | 94              | 85                                          |
| <u><math>E_{1/10}</math> (lux · sec)</u>          |                 |                 |                                             |
| I (20° C., 65% RH)                                | 11.8            | 8.9             | 14.0                                        |
| II (30° C., 80% RH)                               | 10.5            | 8.4             | 13.2                                        |
| III (15° C., 30% RH)                              | 12.9            | 9.8             | 15.4                                        |
| <u>Image Forming<sup>8)</sup> Performance</u>     |                 |                 |                                             |
| I (20° C., 65% RH)                                | Good            | Very good       | Slight edge mark of cutting                 |
| II (30° C., 80% RH)                               | Good            | Very good       | Unevenness in half tone area                |
| III (15° C., 30% RH)                              | Good            | Very good       | White spots in image portion                |
| Water Retentivity of Light-Sensitive Material     | Good            | Good            | Slight background stain                     |
| Printing Durability                               | 10,000 Prints   | 10,000 Prints   | Background stain from the start of printing |

the surface potential ( $V_{10}$ ) to  $1/10$  thereof was determined, and the exposure amount  $E_{1/10}$  (lux.sec) was calculated therefrom.

\*8) Image Forming Performance

The electrophotographic light-sensitive material was allowed to stand for one day under the ambient condition described below, the light-sensitive material was subjected to plate making by a full-automatic plate making machine ELP-404V (manufactured by Fuji Photo Film Co., Ltd.) using ELP-T as a toner. The duplicated image thus obtained was visually evaluated for fog and image quality. The ambient condition at the time of image formation was 20° C. and 65% RH (Condition I), 30° C. and 80% RH (Condition II) or 15° C. and 30% RH (Condition III). The original used for the duplication was composed of cuttings of other originals pasted up thereon.

From the results, it can be seen that each of the light-sensitive materials according to the present invention exhibited good mechanical strength of the photoconductive layer. On the contrary, with the light-sensitive material of Comparative Example IV-5 the value of mechanical strength was lower than them, and the value of  $E_{1/10}$  of electrostatic characteristics degraded particularly under the ambient condition of low temperature and low humidity (Condition III), while they were good under the ambient condition of normal temperature and normal humidity (Condition I). On the other hand, the electrostatic characteristics of the light-sensitive materials according to the present invention were good. Particularly, those of Example IV-30 using the resin (A) having the specified constituent were very good. The value of  $E_{1/10}$  thereof was particularly small.

With respect to image forming performance, the edge mark of cuttings pasted up was observed as background fog in the non-image areas in the light-sensitive material of Comparative Example IV-5. Also the occurrence of unevenness in half tone area of continuous gradation and unevenness of small white spots in image portion were observed on the duplicated image when the ambient conditions at the time of the image formation were high temperature and high humidity (Condition II) and low temperature and low humidity (Condition III).

Further, each of these light-sensitive materials was subjected to the oil-desensitizing treatment to prepare an offset printing plate and using the resulting plate printing was conducted. The plates according to the present invention provided 10,000 prints of clear image without background stains. However, with the plate of Comparative Example IV-5, the above described edge mark of cuttings pasted up was not removed with the oil-desensitizing treatment and the background stains occurred from the start of printing.

It can be seen from the results described above that only the light-sensitive materials according to the present invention could provide excellent performance.

EXAMPLE IV-31

A mixture of 5 g of Resin (A-123), 35 g of Resin (B-122), 200 g of photoconductive zinc oxide, 0.02 g of uranine, 0.04 g of Rose Bengal, 0.03 g of bromophenol blue, 0.40 g of phthalic anhydride and 300 g of toluene was treated in the same manner as described in Example IV-30 to prepare an electrophotographic light-sensitive material.

As the result of the evaluation of various characteristics in the same manner as described in Example IV-30, it can be seen that the light-sensitive material according to the present invention is excellent in charging properties, dark charge retention rate and photosensitivity, and provides a clear

duplicated image free from background fog under severe conditions of high temperature and high humidity (30° C. and 80% RH) and low temperature and low humidity (15° C. and 30% RH). Further, when the material was employed as an offset master plate precursor, 10,000 prints of clear image were obtained.

EXAMPLES IV-32 TO IV-55

Each electrophotographic light-sensitive material was prepared in the same manner as described in Example IV-31, except for using 5 g of each of Resin (A) and 35 g of each of Resin (B) shown in Table IV-6 below in place of 5 g of Resin (A-123) and 35 g of Resin (B-122) used in Example IV-31, respectively.

TABLE IV-6

| Example | Resin (A) | Resin (B) |
|---------|-----------|-----------|
| IV-32   | A-102     | B-102     |
| IV-33   | A-103     | B-101     |
| IV-34   | A-104     | B-106     |
| IV-35   | A-106     | B-107     |
| IV-36   | A-107     | B-109     |
| IV-37   | A-109     | B-110     |
| IV-38   | A-112     | B-111     |
| IV-39   | A-113     | B-112     |
| IV-40   | A-115     | B-113     |
| IV-41   | A-116     | B-114     |
| IV-42   | A-121     | B-115     |
| IV-43   | A-122     | B-116     |
| IV-44   | A-123     | B-117     |
| IV-45   | A-126     | B-118     |
| IV-46   | A-129     | B-119     |
| IV-47   | A-130     | B-120     |
| IV-48   | A-131     | B-121     |
| IV-49   | A-134     | B-122     |
| IV-50   | A-135     | B-124     |
| IV-51   | A-133     | B-125     |
| IV-52   | A-118     | B-126     |
| IV-53   | A-117     | B-128     |
| IV-54   | A-116     | B-129     |
| IV-55   | A-107     | B-130     |

Each of the light-sensitive materials according to the present invention was excellent in charging properties, dark charge retention rate and photosensitivity, and provided a clear duplicated image free from background fog and scratches of fine lines even under severe conditions of high temperature and high humidity (30° C. and 80% RH) and low temperature and low humidity (15° C. and 30% RH). Further, when these materials were employed as offset master plate precursors, 10,000 prints of a clear image free from background stains were obtained respectively.

EXAMPLE V-1

55 A mixture of 4 g (solid basis) of Resin (A-7), 36 g (solid basis) of Resin (B-201), 200 g of photoconductive zinc oxide, 0.018 g of Methine Dye (V-1) having the following structure, 0.45 g of phthalic anhydride and 300 g of toluene was dispersed by a homogenizer (manufactured by Nippon Seiki K.K.) at a rotation of  $6 \times 10^3$  r.p.m. for 10 minutes to 60 prepare a coating composition for a light-sensitive layer. The coating composition was coated on paper, which had been subjected to electrically conductive treatment, by a wire bar at a dry coverage of  $25 \text{ g/m}^2$ , followed by drying at 110° C. for 10 seconds. The coated material was then allowed to stand in a dark place at 20° C. and 65% RH for 24 hours to 65 prepare an electrophotographic light-sensitive material.



## COMPARATIVE EXAMPLE V-1

An electrophotographic light-sensitive material was prepared in the same manner as in Example V-1, except for using 36 g of Resin (R-V-1) shown below in place of 36 g of Resin (B-201) used in Example V-1.

## Comparative Resin (R-V-1)



## COMPARATIVE EXAMPLE V-2

An electrophotographic light-sensitive material was prepared in the same manner as in Example V-1, except for using 36 g of Resin (R-V-2) shown below in place of 36 g of Resin (B-201) used in Example V-1.

## Comparative Resin (R-V-2)



Mw:  $7.5 \times 10^4$  (graft copolymer)

## COMPARATIVE EXAMPLE V-3

An electrophotographic light-sensitive material was prepared in the same manner as in Example V-1, except for using 36 g of Resin (R-V-3) shown below in place of 36 g of Resin (B-201) used in Example V-1.

## Comparative Resin (R-V-3)



Mw:  $7.5 \times 10^4$  (graft copolymer)

With each of the light-sensitive material thus prepared, electrostatic characteristics and image forming performance were evaluated. The results obtained are shown in Table V-1 below.

TABLE V-1

|                                                    | Example V-1 | Comparative Example V-1                               | Comparative Example V-2                               | Comparative Example V-3                               |
|----------------------------------------------------|-------------|-------------------------------------------------------|-------------------------------------------------------|-------------------------------------------------------|
| <u>Electrostatic Characteristics*1)</u>            |             |                                                       |                                                       |                                                       |
| <u><math>V_{10}</math> (-V)</u>                    |             |                                                       |                                                       |                                                       |
| I (20° C., 65% RH)                                 | 680         | 600                                                   | 630                                                   | 635                                                   |
| II (30° C., 80% RH)                                | 660         | 570                                                   | 610                                                   | 620                                                   |
| D.R.R. (90 sec value) (%)                          |             |                                                       |                                                       |                                                       |
| I (20° C., 65% RH)                                 | 89          | 85                                                    | 86                                                    | 86                                                    |
| II (30° C., 80% RH)                                | 86          | 80                                                    | 82                                                    | 83                                                    |
| <u><math>E_{1/10}</math> (erg/cm<sup>2</sup>)</u>  |             |                                                       |                                                       |                                                       |
| I (20° C., 65% RH)                                 | 18          | 31                                                    | 28                                                    | 25                                                    |
| II (30° C., 80% RH)                                | 20          | 35                                                    | 34                                                    | 30                                                    |
| <u><math>E_{1/100}</math> (erg/cm<sup>2</sup>)</u> |             |                                                       |                                                       |                                                       |
| I (20° C., 65% RH)                                 | 27          | 53                                                    | 46                                                    | 41                                                    |
| II (30° C., 80% RH)                                | 31          | 63                                                    | 58                                                    | 50                                                    |
| <u>Image Forming Performance*2)</u>                |             |                                                       |                                                       |                                                       |
| I (20° C., 65% RH)                                 | Very good   | Unevenness in half tone area                          | Unevenness in half tone area                          | Unevenness in half tone area                          |
| II (30° C., 80% RH)                                | Very good   | Scratches of fine lines and letters, background stain | Scratches of fine lines and letters, background stain | Scratches of fine lines and letters, background stain |

The evaluation of each item shown in Table V-1 was conducted in the following manner.

\*1) Electrostatic Characteristics

The light-sensitive material was charged with a corona discharge to a voltage of -6 kV for 20 seconds in a dark room at a temperature of 20° C. and 65% RH using a paper analyzer ("Paper Analyzer SP-428" manufactured by Kawaguchi Denki K.K.). Ten seconds after the corona discharge, the surface potential  $V_{10}$  was measured. The sample was then allowed to stand in the dark for an additional 90 seconds, and the potential  $V_{100}$  was measured. The dark charge retention rate (DRR; %), i.e., percent retention of potential after dark decay for 90 seconds, was calculated from the following equation:

$$DRR (\%) = (V_{100}/V_{10}) \times 100$$

Separately, the surface of photoconductive layer was charged to -400 V with a corona discharge and then exposed to light emitted from a gallium-aluminum-arsenic semiconductor laser (oscillation wavelength: 780 nm), and the time required for decay of the surface potential  $V_{10}$  to one-tenth was measured, and the exposure amount  $E_{1/10}$  (erg/cm<sup>2</sup>) was calculated therefrom. Further, in the same manner as described above the time required for decay of the surface potential  $V_{10}$  to one-hundredth was measured, and the exposure amount  $E_{1/100}$  (erg/cm<sup>2</sup>) was calculated therefrom. The measurements were conducted under ambient condition of 20° C. and 65% RH (Condition I) or 30° C. and 80% RH (Condition II).

\*2) Image Forming Performance

After the light-sensitive material was allowed to stand for one day under the ambient condition shown below, the light-sensitive material was charged to -6 kV and exposed to light emitted from a gallium-aluminum-arsenic semiconductor laser (oscillation wavelength: 780 nm; output: 2.8 mW) at an exposure amount of 64 erg/cm<sup>2</sup> (on the surface of the photoconductive layer) at a pitch of 25 μm and a scanning speed of 300 m/sec. The thus formed electrostatic latent image was developed with a liquid developer ELP-T

(produced by Fuji Photo Film Co., Ltd.), washed with a rinse solution of isoparaffinic solvent Isopar G (manufactured by Esso Chemical K.K.) and fixed. The duplicated image obtained was visually evaluated for fog and image quality. The ambient condition at the time of image formation was 20° C. and 65% RH (Condition I) or 30° C. and 80% RH (Condition II).

As can be seen from the results shown in Table V-1, the light-sensitive material according to the present invention had good electrostatic characteristics. The duplicated image obtained thereon was clear and free from background fog. On the contrary, with the light-sensitive materials of Comparative Examples V-1, V-2 and V-3 the decrease in photosensitivity ( $E_{1/10}$  and  $E_{1/100}$ ) occurred, and in the duplicated images the scratches of fine lines and letters were observed and a slight background fog remained without removing after the rinse treatment. Further, the occurrence of unevenness in half tone areas of continuous gradation of the original was observed regardless of the electrostatic characteristics.

The value of  $E_{1/100}$  is largely different between the light-sensitive material of the present invention and those of the comparative examples. The value of  $E_{1/100}$  indicates an electrical potential remaining in the non-image areas after exposure at the practice of image formation. The smaller the value, the less the background fog in the non-image areas. More specifically, it is requested that the remaining potential is decreased to -10V or less. Therefore, an amount of exposure necessary to make the remaining potential below -10V is an important factor. In the scanning exposure system using a semiconductor laser beam, it is quite important to make the remaining potential below -10V by a small exposure amount in view of a design for an optical system of a duplicator (such as cost of the device, and accuracy of the optical system).

From all these considerations, it is thus clear that an electrophotographic light-sensitive material satisfying both requirements of electrostatic characteristics and image forming performance and being advantageously employed particularly in a scanning exposure system using a semiconductor laser beam can be obtained only when the binder resin according to the present invention is used.

## EXAMPLE V-2

A mixture of 6 g (solid basis) of Resin (A-10), 34 g (solid basis) of Resin (B-202), 200 g of photoconductive zinc oxide, 0.020 g of Methine Dye (V-II) having the following structure, 0.20 g of N-hydroxymaleimide and 300 g of toluene was treated in the same manner as described in Example V-1 to prepare an electrophotographic light-sensitive material.

Methine Dye (V-II)



With the light-sensitive material thus-prepared, a film property in terms of surface smoothness, electrostatic characteristics and image forming performance were evaluated. Further, printing property was evaluated when it was used as an electrophotographic lithographic printing plate precursor. The results obtained are shown in Table V-2 below.

TABLE V-2

|                                                                | Example V-2                |
|----------------------------------------------------------------|----------------------------|
| Smoothness of Photoconductive Layer* <sup>3)</sup><br>(sec/cc) | 200                        |
| <u>Electrostatic Characteristics</u>                           |                            |
| <u>V<sub>10</sub> (-V)</u>                                     |                            |
| I (20° C., 65% RH)                                             | 700                        |
| II (30° C., 80% RH)                                            | 680                        |
| D.R.R. (90 sec value) (%)                                      |                            |
| I (20° C., 65% RH)                                             | 90                         |
| II (30° C., 80% RH)                                            | 87                         |
| <u>E<sub>1/10</sub> (erg/cm<sup>2</sup>)</u>                   |                            |
| I (20° C., 65% RH)                                             | 19                         |
| II (30° C., 80% RH)                                            | 23                         |
| <u>E<sub>1/100</sub> (erg/cm<sup>2</sup>)</u>                  |                            |
| I (20° C., 65% RH)                                             | 29                         |
| II (30° C., 80% RH)                                            | 36                         |
| <u>Image Forming Performance</u>                               |                            |
| I (20° C., 65% RH)                                             | Very good                  |
| II (30° C., 80% RH)                                            | Very good                  |
| Contact Angle with Water* <sup>4)</sup> (°)                    | 0                          |
| Printing Durability* <sup>5)</sup>                             | more than<br>10,000 prints |

The evaluation of each item shown in Table V-2 was conducted in the following manner.

## \*3) Smoothness of Photoconductive Layer

The smoothness (sec/cc) of the light-sensitive material was measured using a Beck's smoothness test machine (manufactured by Kumagaya Riko K.K.) under an air volume condition of 1 cc.

## \*4) Contact Angle with Water

The light-sensitive material was passed once through an etching processor using a solution prepared by diluting an oil-desensitizing solution ELP-EX (produced by Fuji Photo Film Co., Ltd.) to a two-fold volume with distilled water to conduct oil-desensitization treatment on the surface of the photoconductive layer. On the thus oil-desensitized surface

was placed a drop of 2  $\mu$ l of distilled water, and the contact angle formed between the surface and water was measured using a goniometer.

## \*5) Printing Durability

The light-sensitive material was subjected to plate making in the same manner as described in \*2) above to form toner images, and the surface of the photoconductive layer was subjected to oil-desensitization treatment under the same condition as in \*4) above. The resulting lithographic printing

20

plate was mounted on an offset printing machine ("Oliver Model 52", manufactured by Sakurai Seisakusho K.K.), and printing was carried out on paper. The number of prints obtained until background stains in the non-image areas appeared or the quality of the image areas was deteriorated was taken as the printing durability. The larger the number of the prints, the higher the printing durability.

25

As can be seen from the results shown in Table V-2, the light-sensitive material according to the present invention had good surface smoothness and electrostatic characteristics of the photoconductive layer. The duplicated image obtained was clear and free from background fog. These results appear to be due to sufficient adsorption of the binder resin onto the photoconductive substance and sufficient covering of the surface of the particles with the binder resin. For the same reason, when it was used as an offset master plate precursor, oil-desensitization of the offset master plate precursor with an oil-desensitizing solution was sufficient to render the non-image areas satisfactorily hydrophilic, as shown by a small contact angle of 0° with water. On practical printing using the resulting master plate, more than 10,000 prints of clear image without background stains were obtained.

30

From these results it is believed that the resin (A) and the resin (B) according to the present invention suitably interacts with zinc oxide particles to form the condition under which an oil-desensitizing reaction proceeds easily and sufficiently with an oil-desensitizing solution and that the remarkable improvement in film strength is achieved by the action of the resin (B).

35

40

45

50

## EXAMPLES V-3 TO V-24

Each electrophotographic light-sensitive material was prepared in the same manner as described in Example V-2, except for using each of Resins (A) and Resins (B) shown in Table V-3 below in place of Resin (A-10) and Resin (B-202) used in Example V-2, respectively.

60

TABLE V-3

| Example | Resin (A) | Resin (B) |
|---------|-----------|-----------|
| V-3     | A-4       | B-203     |
| V-4     | A-6       | B-204     |
| V-5     | A-8       | B-206     |
| V-6     | A-9       | B-207     |
| V-7     | A-11      | B-208     |

TABLE V-3-continued

| Example | Resin (A) | Resin (B) |
|---------|-----------|-----------|
| V-8     | A-12      | B-209     |
| V-9     | A-13      | B-210     |
| V-10    | A-14      | B-211     |
| V-11    | A-15      | B-212     |
| V-12    | A-17      | B-213     |
| V-13    | A-18      | B-216     |
| V-14    | A-21      | B-217     |
| V-15    | A-22      | B-221     |
| V-16    | A-23      | B-223     |
| V-17    | A-24      | B-224     |
| V-18    | A-25      | B-225     |
| V-19    | A-26      | B-227     |
| V-20    | A-27      | B-228     |
| V-21    | A-28      | B-229     |
| V-22    | A-20      | B-230     |
| V-23    | A-29      | B-231     |
| V-24    | A-1       | B-233     |

The electrostatic characteristics of the resulting light-sensitive materials were evaluated in the same manner as described in Example V-2.

As a result of the evaluation on image forming performance of each light-sensitive material, it was found that clear duplicated images having good reproducibility of fine

lines and letters and no occurrence of unevenness in half tone areas without the formation of background fog were obtained.

5 Further, when these electrophotographic light-sensitive materials were employed as offset master plate precursors under the same printing condition as described in Example V-2, more than 10,000 good prints were obtained respectively.

10 It can be seen from the results described above that each  
of the light-sensitive materials according to the present  
invention was satisfactory in all aspects of the surface  
smoothness and film strength of the photoconductive layer,  
15 electrostatic characteristics, and printing property. Also, it  
can be seen that the electrostatic characteristics are further  
improved by the use of the resin (A).

#### EXAMPLES V-25 TO V-28

Each electrophotographic light-sensitive material was prepared in the same manner as described in Example V-1, except for using each of the dyes shown in Table V-4 below in place of Methine Dye (V-1) used in Example V-1.

TABLE V-4

| Example | Dye     | Chemical Structure of Dye                                                            |
|---------|---------|--------------------------------------------------------------------------------------|
| V-25    | (V-III) |  |
| V-26    | (V-IV)  |  |
| V-27    | (V-V)   |  |
| V-28    | (V-VI)  |  |

Each of the light-sensitive materials according to the present invention was excellent in charging properties, dark charge retention rate and photosensitivity, and provided clear duplicated images free from background fog even when processed under severe condition of high temperature 5 and high humidity (30° C. and 80% RH).

## EXAMPLES V-29 AND V-30

A mixture of 6 g of Resin (A-19) (Example V-29) or Resin (A-9) (Example V-30), 34 g of Resin (B-232), 200 g of photoconductive zinc oxide, 0.02 g of uranine, 0.03 g of Methine Dye (V-VII) having the following structure, 0.03 g of Methine Dye (V-VIII) having the following structure, 0.18 g of p-hydroxybenzoic acid and 300 g of toluene was dispersed by a homogenizer at a rotation of  $7 \times 10^3$  r.p.m. for 8 minutes to prepare a coating composition for a light-sensitive layer. The coating composition was coated on paper, which had been subjected to electrically conductive treatment, by a wire bar at a dry coverage of  $25 \text{ g/m}^2$ , and dried for 20 seconds at 110° C. Then, the coated material was allowed to stand in a dark place for 24 hours under the conditions of 20° C. and 65% RH to prepare each electro-photographic light-sensitive material.

Methine Dye (V-VII)

25



30

Methine Dye (V-VIII)

35



40

## COMPARATIVE EXAMPLE V-4

45

An electrophotographic light-sensitive material was prepared in the same manner as in Example V-29, except for using 34 g of Resin (R-V-4) having the following structure in place of 34 g of Resin (B-232) used in Example V-29.

Comparative Resin (R-V-4)

Mw:  $7.5 \times 10^4$  (graft copolymer)

60

With each of the light-sensitive materials thus prepared, various characteristics were evaluated in the same manner as in Example V-2. The results obtained are shown in Table V-5 below.

TABLE V-5

|                                              | Example V-29   | Example V-30  | Comparative Example V-4                                                     |
|----------------------------------------------|----------------|---------------|-----------------------------------------------------------------------------|
| Binder Resin                                 | (A-19)/(B-232) | (A-9)/(B-232) | (A-19)/R-V-4)                                                               |
| Smoothness of Photoconductive Layer (sec/cc) | 210            | 220           | 200                                                                         |
| Electrostatic Characteristics*6)             |                |               |                                                                             |
| <u><math>V_{10}</math> (-V)</u>              |                |               |                                                                             |
| I (20° C., 65% RH)                           | 600            | 730           | 585                                                                         |
| II (30° C., 80% RH)                          | 580            | 710           | 560                                                                         |
| D.R.R. (%)                                   |                |               |                                                                             |
| I (20° C., 65% RH)                           | 88             | 95            | 87                                                                          |
| II (30° C., 80% RH)                          | 85             | 91            | 84                                                                          |
| $E_{1/10}$ (lux · sec)                       |                |               |                                                                             |
| I (20° C., 65% RH)                           | 10.3           | 7.8           | 12.2                                                                        |
| II (30° C., 80% RH)                          | 11.0           | 8.3           | 13.1                                                                        |
| $E_{1/100}$ (lux · sec)                      |                |               |                                                                             |
| I (20° C., 65% RH)                           | 17             | 12            | 21                                                                          |
| II (30° C., 80% RH)                          | 18             | 13            | 23                                                                          |
| Image Forming*7) Performance                 |                |               |                                                                             |
| I (20° C., 65% RH)                           | Good           | Very good     | Unevenness in half tone area, edge mark of cutting                          |
| II (30° C., 80% RH)                          | Good           | Very good     | Unevenness in half tone area, edge mark of cutting                          |
| Contact Angle with Water (°)                 | 0              | 0             | 0                                                                           |
| Printing Durability                          | 10,000 Prints  | 10,000 Prints | Background stain and Unevenness in image portion from the start of printing |

The characteristics were evaluated in the same manner as in Example V-2, except that some electrostatic characteristics and image forming performance were evaluated according to the following test methods.

\*6) Electrostatic Characteristics:  $E_{1/10}$  and  $E_{1/100}$

The surface of the photoconductive layer was charged to -400 V with corona discharge, and then irradiated by visible light of the illuminance of 2.0 lux on the surface of the photoconductive layer. Then, the time required for decay of the surface potential ( $V_{10}$ ) to  $1/10$  or  $1/100$  thereof was determined, and the exposure amount  $E_{1/10}$  or  $E_{1/100}$  (lux.sec) was calculated therefrom.

\*7) Image Forming Performance

The electrophotographic light-sensitive material was allowed to stand for one day under the ambient condition described below, the light-sensitive material was subjected to plate making by a full-automatic plate making machine ELP-404V (manufactured by Fuji Photo Film Co., Ltd.) using ELP-T as a toner. The duplicated image thus obtained was visually evaluated for fog and image quality. The ambient condition at the time of image formation was 20° C. and 65% RH (Condition I) or 30° C. and 80% RH (Condition II). The original used for the duplication was composed of cuttings of other originals pasted up thereon.

From the results shown above, it can be seen that each light-sensitive material exhibited almost the same properties with respect to the surface smoothness of the photoconductive layer. However, on the electrostatic characteristics, the light-sensitive material of Comparative Example V-4 had the particularly large value of photosensitivity  $E_{1/100}$ , and this tendency increased under the high temperature and high humidity condition. On the contrary, the electrostatic characteristics of the light-sensitive material according to the

present invention were good. Further, those of Example V-30 using the resin (A') having the specified substituent were very good. The value of  $E_{1/100}$  thereof was particularly small.

With respect to image forming performance, the occurrence of unevenness was observed in half tone areas of continuous gradation of highly accurate image and the edge mark of cuttings pasted up was observed as background fog in the non-image areas in the light-sensitive material of Comparative Example V-4. On the contrary, the light-sensitive materials according to the present invention provided clear duplicated images free from background fog.

Further, each of these light-sensitive materials was subjected to the oil-desensitizing treatment to prepare an offset printing plate and using the resulting plate printing was conducted. The plates according to the present invention provided 10,000 prints of clear image without background stains. However, with the plate of Comparative Example V-4, the above described edge mark of cuttings pasted up was not removed with the oil-desensitizing treatment and the background stains occurred from the start of printing.

It can be seen from the results described above that only the light-sensitive materials according to the present invention could provide excellent performance.

#### EXAMPLE V-31

A mixture of 5 g of Resin (A-29), 35 g of Resin (B-209), 200 g of photoconductive zinc oxide, 0.02 g of uranine, 0.04 g of Rose Bengal, 0.03 g of bromophenol blue, 0.40 g of phthalic anhydride and 300 g of toluene was treated in the same manner as described in Example V-29 to prepare an electrophotographic light-sensitive material.

## 201

As the result of the evaluation of various characteristics in the same manner as described in Example V-29, it can be seen that the light-sensitive material according to the present invention is excellent in charging properties, dark charge retention rate and photosensitivity, and provides a clear duplicated image free from background fog under severe conditions of high temperature and high humidity (30° C. and 80% RH). Further, when the material was employed as an offset master plate precursor, 10,000 prints of clear image were obtained.

## EXAMPLES V-32 TO V-43

Each electrophotographic light-sensitive material was prepared in the same manner as described in Example V-31, except for using 6 g of each of Resin (A) and 34 g of each of Resin (B) shown in Table V-6 below in place of 5 g of Resin (A-29) and 35 g of Resin (B-209) used in Example V-31, respectively.

TABLE V-6

| Example | Resin (A) | Resin (B) |
|---------|-----------|-----------|
| V-32    | A-5       | B-203     |
| V-33    | A-6       | B-205     |
| V-34    | A-9       | B-214     |
| V-35    | A-14      | B-215     |
| V-36    | A-17      | B-217     |
| V-37    | A-18      | B-218     |
| V-38    | A-23      | B-221     |
| V-39    | A-24      | B-226     |
| V-40    | A-25      | B-227     |
| V-41    | A-27      | B-232     |
| V-42    | A-28      | B-233     |
| V-43    | A-26      | B-234     |

Each of the light-sensitive materials according to the present invention was excellent in charging properties, dark charge retention rate and photosensitivity, and provided a clear duplicated image free from the occurrence of background fog and scratches of fine lines even under severe condition of high temperature and high humidity (30° C. and 80% RH). Further, when these materials were employed as offset master plate precursors, 10,000 prints of a clear image free from background stains were obtained respectively.

## 202

stand in a dark place at 20° C. and 65% RH for 24 hours to prepare an electrophotographic light-sensitive material.

## Methine Dye (VI-1)



Mw:  $7.5 \times 10^4$  (graft copolymer)

With each of the light-sensitive material thus prepared, electrostatic characteristics and image forming performance were evaluated. The results obtained are shown in Table VI-1 below.

the exposure amount  $E_{1/100}$  ( $\text{erg}/\text{cm}^2$ ) was calculated therefrom. The measurements were conducted under ambient condition of 20° C. and 65% RH (Condition I) or 30° C. and 80% RH (Condition II).

\*2) Image Forming Performance

After the light-sensitive material was allowed to stand for one day under the ambient condition shown below, the light-sensitive material was charged to -6 kV and exposed to light emitted from a gallium-aluminum-arsenic semiconductor laser (oscillation wavelength: 780 nm; output: 2.8 mW) at an exposure amount of 64  $\text{erg}/\text{cm}^2$  (on the surface of the photoconductive layer) at a pitch of 25  $\mu\text{m}$  and a

TABLE VI-1

|                                                                     | Example VI-1 | Comparative Example VI-1                                          | Comparative Example VI-2                                          | Comparative Example VI-3                                          |
|---------------------------------------------------------------------|--------------|-------------------------------------------------------------------|-------------------------------------------------------------------|-------------------------------------------------------------------|
| <u>Electrostatic Characteristics*1)</u>                             |              |                                                                   |                                                                   |                                                                   |
| <u><math>V_{10}</math> (-V)</u>                                     |              |                                                                   |                                                                   |                                                                   |
| I (20° C., 65% RH)                                                  | 760          | 705                                                               | 735                                                               | 740                                                               |
| II (30° C., 80% RH)                                                 | 745          | 680                                                               | 720                                                               | 720                                                               |
| D.R.R. (90 sec value) (%)                                           |              |                                                                   |                                                                   |                                                                   |
| I (20° C., 65% RH)                                                  | 88           | 85                                                                | 87                                                                | 87                                                                |
| II (30° C., 80% RH)                                                 | 85           | 80                                                                | 80                                                                | 82                                                                |
| <u><math>E_{1/10}</math> (<math>\text{erg}/\text{cm}^2</math>)</u>  |              |                                                                   |                                                                   |                                                                   |
| I (20° C., 65% RH)                                                  | 19           | 35                                                                | 30                                                                | 26                                                                |
| II (30° C., 80% RH)                                                 | 23           | 33                                                                | 28                                                                | 28                                                                |
| <u><math>E_{1/100}</math> (<math>\text{erg}/\text{cm}^2</math>)</u> |              |                                                                   |                                                                   |                                                                   |
| I (20° C., 65% RH)                                                  | 33           | 62                                                                | 51                                                                | 44                                                                |
| II (30° C., 80% RH)                                                 | 41           | 65                                                                | 55                                                                | 48                                                                |
| <u>Image Forming Performance*2)</u>                                 |              |                                                                   |                                                                   |                                                                   |
| I (20° C., 65% RH)                                                  | Very good    | Scratches of fine lines and letters, unevenness in half tone area | Scratches of fine lines and letters, unevenness in half tone area | Scratches of fine lines and letters, unevenness in half tone area |
| II (30° C., 80% RH)                                                 | Very good    | Scratches of fine lines and letters, unevenness in half tone area | Scratches of fine lines and letters, unevenness in half tone area | Scratches of fine lines and letters, unevenness in half tone area |

The evaluation of each item shown in Table VI-1 was conducted in the following manner.

\*1) Electrostatic Characteristics

The light-sensitive material was charged with a corona discharge to a voltage of -6 kV for 20 seconds in a dark room at a temperature of 20° C. and 65% RH using a paper analyzer ("Paper Analyzer SP-428" manufactured by Kawaguchi Denki K.K.). Ten seconds after the corona discharge, the surface potential  $V_{10}$  was measured. The sample was then allowed to stand in the dark for an additional 90 seconds, and the potential  $V_{100}$  was measured. The dark charge retention rate (DRR, %), i.e., percent retention of potential after dark decay for 90 seconds, was calculated from the following equation:

$$\text{DRR} (\%) = (V_{100}/V_{10}) \times 100$$

Separately, the surface of photoconductive layer was charged to -400 V with a corona discharge and then exposed to light emitted from a gallium-aluminum-arsenic semiconductor laser (oscillation wavelength: 780 nm), and the time required for decay of the surface potential  $V_{10}$  to one-tenth was measured, and the exposure amount  $E_{1/10}$  ( $\text{erg}/\text{cm}^2$ ) was calculated therefrom. Further, in the same manner as described above the time required for decay of the surface potential  $V_{10}$  to one-hundredth was measured, and

scanning speed of 300 m/sec. The thus formed electrostatic latent image was developed with a liquid developer ELP-T (produced by Fuji Photo Film Co., Ltd.), washed with a rinse solution of isoparaffinic solvent Isopar G (manufactured by Esso Chemical K.K.) and fixed. The duplicated image obtained was visually evaluated for fog and image quality. The ambient condition at the time of image formation was 20° C. and 65% RH (Condition I) or 30° C. and 80% RH (Condition II).

As can be seen from the results shown in Table VI-1, the light-sensitive material according to the present invention had good electrostatic characteristics. The duplicated image obtained thereon was clear and free from background fog.

On the contrary, with the light-sensitive materials of Comparative Examples VI-1, VI-2 and VI-3 the decrease in photosensitivity ( $E_{1/10}$  and  $E_{1/100}$ ) occurred, and in the duplicated images the scratches of fine lines and letters were observed and a slight background fog remained without removing after the rinse treatment. Further, the occurrence of unevenness in half tone areas of continuous gradation of the original was observed regardless of the electrostatic characteristics.

The value of  $E_{1/100}$  is largely different between the light-sensitive material of the present invention and those of the comparative examples. The value of  $E_{1/100}$  indicates an electrical potential remaining in the non-image areas after

exposure at the practice of image formation. The smaller the value, the less the background fog in the non-image areas. More specifically, it is required that the remaining potential is decreased to -10V or less. Therefore, an amount of exposure necessary to make the remaining potential below -10V is an important factor. In the scanning exposure system using a semiconductor laser beam, it is quite important to make the remaining potential below -10V by a small exposure amount in view of a design for an optical system of a duplicator (such as cost of the device, and accuracy of the optical system).

From all these considerations, it is thus clear that an electrophotographic light-sensitive material satisfying both requirements of electrostatic characteristics and image forming performance and being advantageously employed particularly in a scanning exposure system using a semiconductor laser beam can be obtained only using the binder resin according to the present invention.

#### EXAMPLE VI-2

A mixture of 6 g (solid basis) of Resin (A-135), 34 g (solid basis) of Resin (B-202), 200 g of photoconductive zinc oxide, 0.020 g of Methine Dye (VI-II) having the following structure, 0.20 g of N-hydroxymaleimide and 300 g of toluene was treated in the same manner as described in Example VI-1 to prepare an electrophotographic light-sensitive material.

Methine Dye (VI-II)



With the light-sensitive material thus-prepared, a film property in terms of surface smoothness, electrostatic characteristics and image forming performance were evaluated. Further, printing property was evaluated when it was used as an electrophotographic lithographic printing plate precursor. The results obtained are shown in Table VI-2 below.

TABLE VI-2

|                                                               | Example VI-2 |
|---------------------------------------------------------------|--------------|
| Smoothness of Photoconductive Layer* <sup>3</sup><br>(sec/cc) | 230          |
| Electrostatic Characteristics                                 |              |
| <u><math>V_{10}</math> (-V)</u>                               |              |
| I (20° C., 65% RH)                                            | 790          |
| II (30° C., 80% RH)                                           | 770          |
| D.R.R. (90 sec value) (%)                                     |              |
| I (20° C., 65% RH)                                            | 89           |
| II (30° C., 80% RH)                                           | 85           |
| <u><math>E_{1/10}</math> (erg/cm<sup>2</sup>)</u>             |              |
| I (20° C., 65% RH)                                            | 21           |
| II (30° C., 80% RH)                                           | 24           |
| <u><math>E_{1/100}</math> (erg/cm<sup>2</sup>)</u>            |              |
| I (20° C., 65% RH)                                            | 33           |
| II (30° C., 80% RH)                                           | 39           |

TABLE VI-2-continued

|                                            | Example VI-2  |
|--------------------------------------------|---------------|
| <u>Image Forming Performance</u>           |               |
| I (20° C., 65% RH)                         | Very good     |
| II (30° C., 80% RH)                        | Very good     |
| Contact Angle with Water* <sup>4</sup> (°) | 0             |
| Printing Durability* <sup>5</sup>          | 10,000 Prints |

The evaluation of each item shown in Table VI-2 was conducted in the following manner.

\*3) Smoothness of Photoconductive Layer

The smoothness (sec/cc) of the light-sensitive material was measured using a Beck's smoothness test machine (manufactured by Kumagaya Riko K.K.) under an air volume condition of 1 cc.

\*4) Contact Angle with Water

The light-sensitive material was passed once through an etching processor using a solution prepared by diluting an oil-desensitizing solution ELP-EX (produced by Fuji Photo Film Co., Ltd.) to a two-fold volume with distilled water to conduct oil-desensitization treatment on the surface of the photoconductive layer. On the thus oil-desensitized surface was placed a drop of 2  $\mu$ l of distilled water, and the contact angle formed between the surface and water was measured using a goniometer.

\*5) Printing Durability

The light-sensitive material was subjected to plate making in the same manner as described in \*2) above to form toner images, and the surface of the photoconductive layer was subjected to oil-desensitization treatment under the same condition as in \*4) above. The resulting lithographic printing plate was mounted on an offset printing machine ("Oliver Model 52", manufactured by Sakurai Seisakusho K.K.), and printing was carried out on paper. The number of prints obtained until background stains in the non-image areas appeared or the quality of the image areas was deteriorated was taken as the printing durability. The larger the number of the prints, the higher the printing durability.

As can be seen from the results shown in Table VI-2, the light-sensitive material according to the present invention had good electrostatic characteristics. The duplicated image obtained was clear and free from background fog. Also, surface smoothness and mechanical strength of the photoconductive layer were good. These results appear to be due to sufficient adsorption of the binder resin onto the photoconductive substance and sufficient covering of the surface of the particles with the binder resin. For the same reason, when it was used as an offset master plate precursor, oil-desensitization of the offset master plate precursor with an oil-desensitizing solution was sufficient to render the non-image areas satisfactorily hydrophilic, as shown by a small contact angle of 0° with water. On practical printing using the resulting master plate, 10,000 prints of clear image without background stains were obtained.

From these results it is believed that the resin (A) and the resin (B) according to the present invention suitably interacts with zinc oxide particles to form the condition under which an oil-desensitizing reaction proceeds easily and sufficiently with an oil-desensitizing solution and that the remarkable improvement in film strength is achieved by the action of the resin (B). 5

## EXAMPLES VI-3 TO VI-24

Each electrophotographic light-sensitive material was prepared in the same manner as described in Example VI-2, except for using each of Resins (A) and Resins (B) shown in Table VI-3 below in place of Resin (A-135) and Resin (B-202) used in Example VI-2, respectively. 10

TABLE VI-3

| Example | Resin (A) | Resin (B) |
|---------|-----------|-----------|
| VI-3    | A-104     | B-203     |
| VI-4    | A-108     | B-204     |
| VI-5    | A-111     | B-206     |
| VI-6    | A-112     | B-207     |
| VI-7    | A-113     | B-209     |
| VI-8    | A-114     | B-211     |
| VI-9    | A-118     | B-213     |
| VI-10   | A-124     | B-214     |
| VI-11   | A-125     | B-215     |
| VI-12   | A-126     | B-216     |
| VI-13   | A-127     | B-217     |
| VI-14   | A-128     | B-219     |
| VI-15   | A-129     | B-221     |
| VI-16   | A-131     | B-223     |
| VI-17   | A-133     | B-225     |
| VI-18   | A-134     | B-227     |
| VI-19   | A-135     | B-228     |
| VI-20   | A-119     | B-229     |
| VI-21   | A-116     | B-230     |
| VI-22   | A-120     | B-231     |

TABLE VI-3-continued

| Example | Resin (A) | Resin (B) |
|---------|-----------|-----------|
| VI-23   | A-121     | B-233     |
| VI-24   | A-123     | B-235     |

The electrostatic characteristics of the resulting light-sensitive materials were evaluated in the same manner as described in Example VI-2. 10

As a result of the evaluation on image forming performance of each light-sensitive material, it was found that clean duplicated images having good reproducibility of fine lines and letters and no occurrence of unevenness in half tone areas without the formation of background fog were obtained. 15

Further, when these electrophotographic light-sensitive materials were employed as offset master plate precursors under the same printing condition as described in Example VI-2, more than 10,000 good prints were obtained respectively. 20

It can be seen from the results described above that each of the light-sensitive materials according to the present invention was satisfactory in all aspects of the surface smoothness and film strength of the photoconductive layer, electrostatic characteristics, and printing property. Also, it can be seen that the electrostatic characteristics are further improved by the use of the resin (A'). 25

30

## EXAMPLES VI-25 TO VI-28

Each electrophotographic light-sensitive material was prepared in the same manner as described Example VI-1, except for using each of the dyes shown in Table VI-4 below in place of Methine Dye (VI-1) used in Example VI-1. 35

TABLE VI-4

| Example        | Dye | Chemical Structure of Dye                                                            |
|----------------|-----|--------------------------------------------------------------------------------------|
| VI-25 (VI-III) |     |  |
| VI-26 (VI-IV)  |     |  |
| VI-27 (VI-V)   |     |  |

TABLE VI-4-continued

| Example       | Dye | Chemical Structure of Dye |
|---------------|-----|---------------------------|
| VI-28 (VI-VI) |     |                           |

Each of the light-sensitive materials according to the present invention was excellent in charging properties, dark charge retention rate and photosensitivity, and provided clear duplicated images free from background fog even when processed under severe condition of high temperature and high humidity (30° C. and 80% RH).

## EXAMPLES VI-29 AND VI-30

A mixture of 6 g of Resin (A-101) (Example VI-29) or Resin (A-135) (Example VI-30), 34 g of Resin (B-225), 200 g of photoconductive zinc oxide, 0.02 g of uranine, 0.03 g of Methine Dye (VI-VII) having the following structure, 0.03 g of Methine Dye (VI-VIII) having the following structure, 0.18 g of p-hydroxybenzoic acid and 300 g of toluene was dispersed by a homogenizer at a rotation of  $7 \times 10^3$  r.p.m. for 8 minutes to prepare a coating composition for a light-sensitive layer. The coating composition was coated on paper, which had been subjected to electrically conductive treatment, by a wire bar at a dry coverage of 25 g/m<sup>2</sup>, and dried for 20 seconds at 110° C. Then, the coated material was allowed to stand in a dark place for 24 hours under the conditions of 20° C. and 65% RH to prepare each 45 electrophotographic light-sensitive material.



## COMPARATIVE EXAMPLE VI-4

An electrophotographic light-sensitive material was prepared in the same manner as in Example VI-29, except for using 34 g of Resin (R-VI-4) having the following structure in place of 34 g of Resin (B-225) used in Example VI-29.

## Comparative Resin (R-VI-4)



With each of the light-sensitive materials thus prepared, various characteristics were evaluated in the same manner as in Example VI-2. The results obtained are shown in Table VI-5 below.

TABLE VI-5

|                                                   | Example VI-29   | Example VI-30   | Comparative Example VI-4                                                |
|---------------------------------------------------|-----------------|-----------------|-------------------------------------------------------------------------|
| Binder Resin                                      | (A-101)/(B-225) | (A-135)/(B-225) | (A-101)/R-VI-4)                                                         |
| Smoothness of Photoconductive Layer (sec/cc)      | 220             | 215             | 205                                                                     |
| <u>Electrostatic Characteristics<sup>6)</sup></u> |                 |                 |                                                                         |
| <u><math>V_{10}</math> (-V)</u>                   |                 |                 |                                                                         |
| I (20° C., 65% RH)                                | 600             | 685             | 585                                                                     |
| II (30° C., 80% RH)                               | 585             | 670             | 565                                                                     |
| <u>D.R.R. (%)</u>                                 |                 |                 |                                                                         |
| I (20° C., 65% RH)                                | 90              | 96              | 88                                                                      |
| II (30° C., 80% RH)                               | 87              | 93              | 84                                                                      |
| <u><math>E_{1/10}</math> (lux · sec)</u>          |                 |                 |                                                                         |
| I (20° C., 65% RH)                                | 10.5            | 8.1             | 12.8                                                                    |
| II (30° C., 80% RH)                               | 11.2            | 8.8             | 13.3                                                                    |
| <u><math>E_{1/100}</math> (lux · sec)</u>         |                 |                 |                                                                         |
| I (20° C., 65% RH)                                | 17              | 13              | 21                                                                      |
| II (30° C., 80% RH)                               | 19              | 14              | 23                                                                      |
| <u>Image Forming<sup>7)</sup> Performance</u>     |                 |                 |                                                                         |
| I (20° C., 65% RH)                                | Good            | Very good       | Edge mark of cutting                                                    |
| II (30° C., 80% RH)                               | Good            | Very good       | Edge mark of cutting, unevenness in half tone area                      |
| <u>Contact Angle with Water (°)</u>               | 0               | 0               | 0                                                                       |
| Printing Durability                               | 10,000 Prints   | 10,000 Prints   | Background stain due to edge mark of cutting from the start of printing |

The characteristics were evaluated in the same manner as in Example VI-2, except that some electrostatic characteristics and image forming performance were evaluated according to the following test methods.

\*6) Electrostatic Characteristics:  $E_{1/10}$  and  $E_{1/100}$

The surface of the photoconductive layer was charged to -400 V with corona discharge, and then irradiated by visible light of the illuminance of 2.0 lux on the surface of the photoconductive layer. Then, the time required for decay of the surface potential ( $V_{10}$ ) to  $1/10$  or  $1/100$  thereof was determined, and the exposure amount  $E_{1/10}$  or  $E_{1/100}$  (lux.sec) was calculated therefrom.

\*7) Image Forming Performance

The electrophotographic light-sensitive material was allowed to stand for one day under the ambient condition described below, the light-sensitive material was subjected to plate making by a full-automatic plate making machine ELP-404V (manufactured by Fuji Photo Film Co., Ltd.) using ELP-T as a toner. The duplicated image thus obtained was visually evaluated for fog and image quality. The ambient condition at the time of image formation was 20° C. and 65% RH (Condition I) or 30° C. and 80% RH (Condition II). The original used for the duplication was composed of cuttings of other originals pasted up thereon.

From the results shown above, it can be seen that each light-sensitive material exhibited almost same properties with respect to the surface smoothness of the photoconductive layer. However, on the electrostatic characteristics, the light-sensitive material of Comparative Example VI-4 had the particularly large value of photosensitivity  $E_{1/100}$  and this tendency increased under the high temperature and high humidity condition. On the contrary, the electrostatic characteristics of the light-sensitive material according to the present invention were good. Further, those of Example VI-30 using the resin (A') having the specified substituent

35

40

45

50

55

60

65

were very good. The value of  $E_{1/100}$  thereof was particularly small.

With respect to image forming performance, the occurrence of the edge mark of cuttings pasted up was observed as background fog in the non-image areas in the light-sensitive material of Comparative Example VI-4. On the contrary, the light-sensitive materials according to the present invention provided clear duplicated images free from background fog.

Further, each of these light-sensitive materials was subjected to the oil-desensitizing treatment to prepare an offset printing plate and using the resulting plate printing was conducted. The plates according to the present invention provided 10,000 prints of clear image without background stains. However, with the plate of Comparative Example VI-4, the above described edge mark of cuttings pasted up was not removed with the oil-desensitizing treatment and the background stains occurred from the start of printing.

It can be seen from the results described above that only the light-sensitive materials according to the present invention could provide excellent performance.

#### EXAMPLE VI-31

A mixture of 5 g of Resin (A-129), 35 g of Resin (B-230), 200 g of photoconductive zinc oxide, 0.02 g of uranine, 0.04 g of Rose Bengal, 0.03 g of bromophenol blue, 0.40 g of phthalic anhydride and 300 g of toluene was treated in the same manner as described in Example VI-29 to prepare an electrophotographic light-sensitive material.

As the result of the evaluation of various characteristics in the same manner as described in Example VI-29, it can be seen that the light-sensitive material according to the present

invention is excellent in charging properties, dark charge retention rate and photosensitivity, and provides a clear duplicated image free from background fog under severe conditions of high temperature and high humidity (30° C. and 80% RH). Further, when the material was employed as an offset master plate precursor, 10,000 prints of clear image were obtained.

## EXAMPLES VI-32 TO VI-43

Each electrophotographic light-sensitive material was prepared in the same manner as described in Example VI-31, except for using 6 g of each of Resin (A) and 34 g of each of Resin (B) shown in Table VI-6 below in place of 5 g of Resin (A-129) and 35 g of Resin (B-230) used in Example VI-31, respectively.

TABLE VI-6

| Example | Resin (A) | Resin (B) |
|---------|-----------|-----------|
| VI-32   | A-103     | B-218     |
| VI-33   | A-104     | B-219     |
| VI-34   | A-106     | B-210     |
| VI-35   | A-107     | B-213     |
| VI-36   | A-109     | B-216     |
| VI-37   | A-110     | B-217     |
| VI-38   | A-112     | B-220     |
| VI-39   | A-117     | B-221     |
| VI-40   | A-129     | B-226     |
| VI-41   | A-131     | B-230     |
| VI-42   | A-132     | B-232     |
| VI-43   | A-125     | B-231     |

Each of the light-sensitive materials according to the present invention was excellent in charging properties, dark charge retention rate and photosensitivity, and provided a clear duplicated image free from the occurrence of background fog and scratches of fine lines even under severe condition of high temperature and high humidity (30° C. and 80% RH). Further, when these materials were employed as offset master plate precursors, 10,000 prints of a clear image free from background stains were obtained respectively.

## POSSIBILITY OF UTILIZATION IN INDUSTRY

In accordance with the present invention, an electrophotographic light-sensitive material which exhibits excellent electrostatic characteristics (particularly, under severe conditions) and mechanical strength and provides clear images of good quality can be obtained. The electrophotographic light-sensitive material according to the present invention is particularly useful in the scanning exposure system using a semiconductor laser beam. The electrostatic characteristics are further improved by using the resin according to the present invention which contains a reapeating unit having the specific methacrylate component.

What is claimed is:

1. An electrophotographic light-sensitive material having a photoconductive layer containing at least an inorganic photoconductive substance, a spectral sensitizing dye and a binder resin, wherein the binder resin comprises at least one resin selected from the group consisting of resin (A<sub>1</sub>), resin (A<sub>2</sub>) and resin (A<sub>3</sub>) shown below and at least one resin (B) shown below:

Resin (A<sub>1</sub>):

a copolymer having a weight average molecular weight of from 1×10<sup>3</sup> to 2×10<sup>4</sup> as determined by gel permeation chromatography and being formed at least from a monofunctional macromonomer (M<sub>1</sub>) described below and a monomer corresponding to a repeating unit represented by the general formula (I) described below, wherein the copolymer has a polymer component containing at least one polar group selected from the group consisting of —PO<sub>3</sub>H<sub>2</sub>, —SO<sub>3</sub>H, —COOH,



(wherein R<sup>1</sup> represents a hydrocarbon group or —OR<sup>2</sup> (wherein R<sup>2</sup> represents a hydrocarbon group)) and a cyclic acid anhydride group bonded at one terminal of the main chain thereof;

Monofunctional macromonomer (M<sub>1</sub>):

a monofunctional macromonomer having a weight average molecular weight of not more than 2×10<sup>4</sup> as determined by gel permeation chromatography and having a polymerizable double bond group bonded at only one terminal of the main chain of a polymer containing not less than 30% by weight of a polymer component corresponding to a repeating unit represented by the general formula (I) described below:

## 30 Formula (I)



(wherein a<sup>1</sup> and a<sup>2</sup> each represents a hydrogen atom, a halogen atom, a cyano group, a hydrocarbon group —COOR<sup>4</sup> or —COOR<sup>4</sup> bonded via a hydrocarbon group (wherein R<sup>4</sup> represents a hydrocarbon group); and R<sup>3</sup> represents a hydrocarbon group);

40 Resin (A<sub>2</sub>):

a copolymer having a weight average molecular weight of from 1×10<sup>3</sup> to 2×10<sup>4</sup> as determined by gel permeation chromatography and being formed at least from a monofunctional macromonomer (M<sub>2</sub>) described below and a monomer corresponding to a repeating unit represented by the general formula (I) described above; Monofunctional macromonomer (M<sub>2</sub>):

a monofunctional macromonomer having a weight average molecular weight of not more than 2×10<sup>4</sup> as determined by gel permeation chromatography and having a polymerizable double bond group at only one terminal of the main chain of a polymer containing at random not less than 30% by weight of a polymer component corresponding to a repeating unit represented by the general formula (I) described above and from 1 to 50% by weight of a polymer component containing at least one polar group selected from the specified polar groups as described in the resin (A<sub>1</sub>) above;

60 Resin (A<sub>3</sub>):

a copolymer having a weight average molecular weight of from 1×10<sup>3</sup> to 2×10<sup>4</sup> as determined by gel permeation chromatography and being formed at least from a monofunctional macromonomer (M<sub>3</sub>) described below and a monomer corresponding to a repeating unit represented by the general formula (I) described above;

Monofunctional macromonomer ( $M_3$ ):

a monofunctional macromonomer having a weight average molecular weight of not more than  $2 \times 10^4$  as determined by gel permeation chromatography, comprising an AB block copolymer composed of an A block containing a polymer component containing at least one polar group selected from the specified polar groups as described in the resin ( $A_1$ ) above and a B block containing a polymer component corresponding to a repeating unit represented by the general formula (II) described below and having a polymerizable double bond group bonded at the terminal of the main chain of the B block polymer:

Formula (II)



wherein  $b^1$  and  $b^2$  each represents a hydrogen atom, a halogen atom, a cyano group a hydrocarbon group,  $-\text{COOR}^4$  or  $-\text{COOR}^4$  bonded via a hydrocarbon group (wherein  $R^4$  represents a hydrocarbon group);  $V^1$  represents  $-\text{COO}-$ ,  $-\text{OCO}-$ ,  $-(\text{CH}_2)_a \text{OCO}-$ ,  $-(\text{CH}_2)_a \text{COO}-$  (wherein  $a$  represents an integer of from 1 to 3),  $-\text{O}-$ ,  $-\text{SO}_2-$ ,  $-\text{CO}-$ ,



(wherein  $Z^1$  represent a hydrogen atom or a hydrocarbon group),  $-\text{CONHCOCO}-$ ,  $-\text{CONHCONH}-$  or



and  $R^5$  represents a hydrocarbon group, provided that when  $V^1$  represents



$R^5$  represents a hydrogen atom or a hydrocarbon group; Resin (B):

a starlike polymer having a weight average molecular weight of from  $3 \times 10^4$  to  $1 \times 10^6$  and comprising an organic molecule having bonded thereto at least three polymer chains each containing a polymer component containing at least one polar group selected from the specified polar groups as described in the resin ( $A_1$ ) above and a polymer component corresponding to a repeating unit represented by the general formula (I) as described in the resin ( $A_1$ ) above, wherein the polymer contains the polymer component containing a polar group in an amount of from 0.01 to 10% by weight based on the polymer and the polymer component corresponding to the general formula (I) in an amount not less than 30% by weight based on the polymer.

2. An electrophotographic light-sensitive material as claimed in claim 1, wherein the resin ( $A_1$ ), ( $A_2$ ) or ( $A_3$ )

5

10

15

20

25

30

35

40

45

50

55

60

contains, as the polymer component represented by the general formula (I), at least one methacrylate component having an aryl group represented by the following general formulae (Ia) and (Ib):



Formula (Ia)



Formula (Ib)

wherein  $T_1$  and  $T_2$  each represents a hydrogen atom, a halogen atom, a hydrocarbon group having from 1 to 10 carbon atoms, a cyano group,  $-\text{COR}_a$  or  $-\text{COOR}_a$  wherein  $R_a$  represents a hydrocarbon group having from 1 to 10 carbon atoms; and  $L_1$  and  $L_2$  each represents a mere bond or a linking group containing from 1 to 4 linking atoms, which connects  $-\text{COO}-$  and the benzene ring.

3. An electrophotographic light-sensitive material as claimed in claim 1, wherein the total amount of the specific polar group-containing polymer component contained in the polymer of the resin (B) is from 10 to 50% by weight based on the total amount of the specific polar group-containing polymer component present in the resin ( $A_1$ ), ( $A_2$ ) or ( $A_3$ ).

4. An electrophotographic light-sensitive material as claimed in claim 1, wherein the resin ( $A_2$ ) is a copolymer further having a polymer component containing at least one polar group selected from the specified polar groups described in the resin ( $A_1$ ) above bonded at one terminal of the main chain thereof.

5. An electrophotographic light-sensitive material as claimed in claim 1, wherein the at least three polymer chains in the resin (B) each comprise an AB block polymer chain composed of an A block comprising a polymer component containing the polar group and a B block comprising a polymer component corresponding to the general formula (I).

6. An electrophotographic light-sensitive material as claimed in claim 5, wherein the at least three polymer chains in the resin (B) each comprise an AB block copolymer chain in which a polymer component containing the specified polar group is bonded at one terminal of the A block polymer chain and the B block polymer chain is bonded at the other terminal of the A block polymer chain.

7. An electrophotographic light-sensitive material as claimed in claim 1, wherein the at least three polymer chains in the resin (B) each comprise a polymer component corresponding to the general formula (I), and are each bonded to the organic molecule at one terminal thereof and have a polymer component containing the specified polar group at the other terminal thereof.

\* \* \* \* \*